

# United States Patent [19]

Honda et al.

[11] Patent Number: 4,762,762

[45] Date of Patent: Aug. 9, 1988

[54] ELECTROPHOTOGRAPHIC LIGHT RECEIVING MEMBERS COMPRISING AMORPHOUS SILICON AND SUBSTRATE HAVING MINUTE IRREGULARITIES

[75] Inventors: Mitsuru Honda; Atsushi Koike, both of Chiba; Kyosuke Ogawa, Miye; Keiichi Murai, Chiba, all of Japan

[73] Assignee: Canon Kabushiki Kaisha, Tokyo, Japan

[21] Appl. No.: 921,638

[22] Filed: Oct. 22, 1986

## [30] Foreign Application Priority Data

|                    |             |           |
|--------------------|-------------|-----------|
| Oct. 24, 1985 [JP] | Japan ..... | 60-236286 |
| Oct. 28, 1985 [JP] | Japan ..... | 60-239551 |
| Oct. 29, 1985 [JP] | Japan ..... | 60-241891 |
| Oct. 30, 1985 [JP] | Japan ..... | 60-241574 |
| Oct. 31, 1985 [JP] | Japan ..... | 60-242786 |
| Nov. 1, 1985 [JP]  | Japan ..... | 60-244141 |

[51] Int. Cl. 4 .....

G03G 5/082; G03G 5/14

[52] U.S. Cl. .....

430/65; 430/67;  
430/69; 430/84; 430/945; 430/950

[58] Field of Search .....

430/84, 507, 950, 945,  
430/65, 67, 69

[56]

## References Cited

### U.S. PATENT DOCUMENTS

|           |         |                    |          |
|-----------|---------|--------------------|----------|
| 4,292,389 | 9/1981  | Kojima et al. .... | 430/950  |
| 4,352,847 | 10/1982 | Okiyama .....      | 430/950  |
| 4,514,582 | 4/1985  | Tiedje .....       | 427/39 X |

Primary Examiner—J. David Welsh

Attorney, Agent, or Firm—Fitzpatrick, Cella, Harper & Scinto

[57]

## ABSTRACT

A light receiving member comprises a support and a light receiving layer of a multi-layered structure having at least a photosensitive layer composed of an amorphous silicon, said support having a surface provided with irregularities composed of spherical dimples each of which having an inside face provided with minute irregularities. The light receiving layer may contain a surface layer comprising an outer abrasion-resistant layer and an inner reflection prevention layer, wherein the optical band gap possessed by the surface layer and optical band gap possessed by the photosensitive layer on which the surface layer is disposed are matched at their interface. The light receiving member can effectively prevent the occurrence of interference fringes in the formed images, forming visible images of excellent quality even when coherent laser beams are used as the light source. The member can also effectively prevent reflection of incident light at the interface between the surface layer and the photosensitive layer.

57 Claims, 40 Drawing Sheets

FIG. 1

(A)



FIG. 1

(B)



FIG. 1

(C)



FIG. 2



FIG. 3



FIG. 4



FIG. 5



## FIG. 6

(A)



FIG. 6

(B)



FIG. 7



FIG. 8



FIG. 9



FIG. 10



FIG. 11



FIG. 12



FIG. 13



FIG. 14



FIG. 15



FIG. 16



FIG. 17



FIG. 18



FIG. 19



FIG. 20

(A)



FIG. 20

(B)



FIG. 21



FIG. 22



FIG. 23



FIG. 24



FIG. 25



FIG. 26



FIG. 27



FIG. 28



FIG. 29



FIG. 30



FIG. 31



FIG. 32



FIG. 33



FIG. 34



FIG. 35



FIG. 36



FIG. 37



FIG. 38



FIG. 39



FIG. 40



FIG. 41



FIG. 42



FIG. 43





FIG. 44



**ELECTROPHOTOGRAPHIC LIGHT RECEIVING  
MEMBERS COMPRISING AMORPHOUS  
SILICON AND SUBSTRATE HAVING MINUTE  
IRREGULARITIES**

**BACKGROUND OF THE INVENTION**

**1. Field of the Invention**

This invention concerns light receiving members being sensitive to electromagnetic waves such as light (which herein means in a broader sense those lights such as ultraviolet rays, visible rays, infrared rays, X-rays and  $\gamma$ -rays). More specifically, the invention relates to improved light receiving members suitable particularly for use in the case where coherent lights such as laser beams are applied.

**2. Description of the Prior Art**

For recording of digital image information, there have been known such a method as forming electrostatic latent images by optically scanning a light receiving member with laser beams modulated in accordance with the digital image information, and then developing the latent images or further applying transfer, fixing or like other treatment as required. Particularly, in the method of forming images by an electrophotographic process, image recording has usually been conducted by using a He, Ne laser or a semiconductor laser (usually having emission wavelength as from 650 to 820 nm), which is small in size and inexpensive in cost as the laser source.

By the way, as the light receiving members for electrophotography being suitable for use in the case of using the semiconductor laser, those light receiving members comprising amorphous materials containing silicon atoms (hereinafter referred to as "a-Si"), for example, as disclosed in Japanese Patent Laid-Open Nos. 86341/1979 and 83746/1981 have been evaluated as being worthy of attention. They have a high Vickers hardness and cause less problems in the public pollution, in addition to their excellent matching property in the photosensitive region as compared with other kinds of known light receiving members.

However, when the light receiving layer constituting the light receiving member as described above is formed as an a-Si layer of a mono-layer structure, it is necessary to structurally incorporate hydrogen or halogen atoms or, further, boron atoms within a range of specific amount into the layer in order to maintain the required dark resistance of greater than  $10^{12} \Omega\text{cm}$  as for the electrophotography while maintaining their high photosensitivity. Therefore, the degree of freedom for the design of the light receiving member undergoes a rather severe limit such as the requirement for the strict control for various kind of conditions upon forming the layer. Then, there have been made several proposals to overcome such problems for the degree of freedom in view of the design in that the high photosensitivity can effectively be utilized while reducing the dark resistance to some extent. That is, the light receiving layer is so constituted as to have two or more layers prepared by laminating those layers of different conductivity in which a depletion layer is formed to the inside of the light receiving layer as disclosed in Japanese Patent Laid-Open Nos. 171743/1979, 4053/1982 and 4172/1982, or the apparent dark resistance is improved by providing a multi-layered structure in which a barrier layer is disposed between a support and a light receiving layer and/or on the upper surface of the light

receiving layer as disclosed, for example, in Japanese Patent Publication Nos. 52178, 52179, 52180, 58159, 58160 and 58161/1981.

However, such light receiving members as having a light receiving layer of multi-layered structure have unevenness in the thickness for each of the layers. In the case of conducting the laser recording by using such members, since the laser beams comprise coherent light, the respective light beams reflected from the free surface of the light receiving layer on the side of the laser beam irradiation and from the layer boundary between each of the layers constituting the light receiving layer and between the support and the light receiving layer (hereinafter both of the free surface and the layer interface are correctively referred to as "interface") often interfere with each other.

The interference results in a so-called interference fringe pattern in the formed visible images which causes defective images. Particularly, in the case of forming intermediate tone images with high gradation, the images obtained become extremely poor in quality.

In addition, as an important point there exist problems that the foregoing interference phenomenon will become remarkably due to that the absorption of the laser beams in the light receiving layer is decreased as the wavelength region of the semiconductor laser beams used is increased.

That is, in the case of two or more layer (multi-layered) structure, interference effects occur as for each of the layers, and those interference effects are synergistically acted with each other to exhibit interference fringe patterns, which directly influence on the transfer member thereby to transfer and fix the interference fringe on the member, and thus bringing about defective images in the visible images corresponding to the interference fringe pattern.

In order to overcome these problems, there have been proposed, for example, (a) a method of cutting the surface of the support with diamond means to form a light scattering surface formed with unevenness of  $\pm 500 \text{ \AA} \pm 10,000 \text{ \AA}$  (refer, for example, to Japanese Patent Laid-Open No. 162975/1983), (b) a method of disposing a light absorbing layer by treating the surface of an aluminum support with black alumite or by dispersing carbon, colored pigment or dye into a resin (refer, for example, to Japanese Patent Laid-Open No. 165845/1982) and (c) a method of disposing a light scattering reflection prevention layer on the surface of an aluminum support by treating the surface of the support with a satin-line alumite processing or by disposing a fine grain-like unevenness by means of sand blasting (refer, for example, to Japanese Patent Laid-Open No. 16554/1982).

Although these proposed methods provide satisfactory results to some extent, they are not sufficient for completely eliminating the interference fringe pattern which forms in the images.

That is, in the method (a), since a plurality of irregularities with a specific  $t$  are formed at the surface of the support, occurrence of the interference fringe pattern due to the light scattering effect can be prevented to some extent. However, since the positive reflection light component is still left as the light scattering, the interference fringe pattern due to the positive reflection light still remains and, in addition, the irradiation spot is widened due to the light scattering effect at the support

surface to result in a substantial reduction in the resolution power.

In the method (b), it is impossible to obtain complete absorption only by the black alumite treatment, and the reflection light still remains at the support surface. And in the case of disposing the resin layer dispersed with the pigment, there are various problems; degasification is caused from the resin layer upon forming a-Si layer to invite a remarkable deterioration on the quality of the resulting light receiving layer: the resin layer is damaged by the plasma upon forming the a-Si layer wherein the inherent absorbing function is reduced and undesired effects are given to the subsequent formation of the a-Si layer due to the worsening in the surface state.

In the method (c), referring to incident light for instance, a portion of the incident light is reflected at the surface of the light receiving layer to be a reflected light, while the remaining portion intrudes as the transmitted light to the inside of the light receiving layer. And a portion of the transmitted light is scattered as a diffused light at the surface of the support and the remaining portion is regularly reflected as a reflected light, a portion of which goes out as the outgoing light. However, the outgoing light is a component to interfere with the reflected light. In any event, since the light remains, the interference fringe pattern cannot be completely eliminated.

For preventing the interference in this case, attempts have been made to increase the diffusibility at the surface of the support so that no multi-reflection occurs at the inside of the light receiving layer. However, this somewhat diffuses the light in the light receiving layer thereby causing halation and, accordingly, reducing the resolution power.

Particularly, in the light receiving member of the multi-layered structure, if the support surface is roughened irregularly, the reflection light at the surface of the first layer, the reflection layer at the second layer and the positive reflection light at the support surface interfere with each other which results in the interference fringe pattern in accordance with the thickness of each layer in the light receiving member. Accordingly, it is impossible to completely prevent the interference fringe by unevenly roughening the surface of the support in the light receiving member of the multi-layered structure.

In the case of unevenly roughening the surface of the support by the sand blasting or like other method, scattering of the roughness is often caused between the lots and the unevenness in the roughness occurs even in an identical lot thereby causing problems in view of the production control. In addition, relatively large protrusions are frequently formed at random and such large protrusions cause local break down in the light receiving layer.

Further, even if the surface of the support is regularly roughened, since the light receiving layer is usually deposited along with the uneven shape at the surface of the support, the inclined surface on the unevenness at the support are in parallel with the inclined surface on the unevenness at the light receiving layer, where the incident light brings about bright and dark areas. Further, in the light receiving layer, since the layer thickness is not uniform over the entire light receiving layer, a dark and bright stripe pattern results. Accordingly, mere orderly roughening the surface of the support can not completely prevent the occurrence of the interference fringe pattern.

Furthermore, in the case of depositing the light receiving layer of a multi-layered structure on the support having the surface which is regularly roughened, since the interference due to the reflection light at the interface between each of the layers is joined to the interference between the positive reflection light at the surface of the support and the reflection light at the surface of the light receiving layer, the situation is more complicated than the occurrence of the interference fringe in the light receiving member of a single layer structure.

Furthermore, the problem of the interference due to the reflection light in the receiving member of such multi-layered structure also concerns with the surface layer. That is, as can be seen from the foregoing, if the thickness of the surface layer is not uniform, interference occurs due to the reflected light at the interface between the surface layer and the photosensitive layer adjacent thereto to result in trouble in the functioning of the light receiving member.

The unevenness of the thickness of the surface layer is brought about upon forming the surface layer, as well as by abrasion, particularly, partial abrasion during use of the light receiving member. Particularly, in the latter case, it results in the occurrence of the interference pattern as described above and, in addition, also results in the change in the sensitivity, uneven sensitivity or the like over the entire light receiving member.

To eliminate such problems regarding the surface layer, it has been attempted to increase the thickness of the surface layer as much as possible. However this leads to the increase in the residual potential and rather increases the unevenness in the layer thickness of the surface layer. Since the light receiving member having such a surface layer involves the factors for causing problems such as changes in the sensitivity and uneven sensitivity already when the layer has been formed, the member will provide those images that can not be appreciated from the initial time of use.

#### SUMMARY OF THE INVENTION

The object of this invention is to provide a light receiving member comprising a light receiving layer mainly composed of a-Si, free from the foregoing problems and capable of satisfying various kinds of requirements.

That is, the main object of this invention is to provide a light receiving member having a light receiving layer constituted with a-Si in which electrical, optical and photoconductive properties are always substantially stable scarcely depending on the working circumstances, and which is excellent against optical fatigue, causes no degradation upon repeated use, excellent in durability and moisture-proofness, exhibits no or scarcely any residual potential and provides easy production control.

Another object of this invention is to provide a light receiving member having a light receiving layer composed of a-Si which has a high photosensitivity in the entire visible region of light, particularly, an excellent matching property with a semiconductor laser and shows rapid light response.

Other object of this invention is to provide a light receiving member having a light receiving layer composed of a-Si which has high photosensitivity, high S/N ratio and high electrical voltage withstanding property.

A further object of this invention is to provide a light receiving member having a light receiving layer composed of a-Si which is excellent in the close bondability

between a support and a layer disposed on the support or between each of the laminated layers, dense and stable in view of the structural arrangement and of high layer quality.

A further object of this invention is to provide a light receiving member having a light receiving layer composed of a-Si which is suitable to the image formation by using coherent light, free from the occurrence of interference fringe pattern and spots upon reversed development even after repeated use for a long period of time, free from defective images or blurring in the images, shows high density with clear half tone, and has a high resolution power and can provide high quality images.

#### BRIEF DESCRIPTION OF THE DRAWINGS

These and other objects, as well as the features of this invention will become apparent by reading the following descriptions of preferred embodiments according to this invention while referring to the accompanying drawings, wherein:

FIGS. 1(A)-(C) are views schematically illustrating typical examples of light receiving members according to this invention;

FIGS. 2 and 3 are enlarged views for a portion illustrating the principle of preventing the occurrence of an interference fringe in the light receiving member according to this invention, in which

FIG. 2 is a view illustrating that the occurrence of the interference fringe can be prevented in the light receiving member in which unevenness constituted with spherical dimples is formed to the surface of a support, and

FIG. 3 is a view illustrating that the interference fringe results in the conventional light receiving member in which the light receiving layer is deposited on a support roughened regularly at the surface;

FIGS. 4 and 5 are schematic views for illustrating the uneven shape at the surface of the support of the light receiving member according to this invention and a method of preparing the uneven shape;

FIGS. 6(A) and 6(B) illustrate a chart schematically illustrating a constitutional example of a device suitable for forming the uneven shape formed to the support of the light receiving member according to this invention, in which

FIG. 6(A) is a front elevational view and

FIG. 6(B) is a vertical cross-sectional view;

FIGS. 7 through 15 are views illustrating the distribution state, in the direction of the layer thickness, of at least one of the elements selected from oxygen atoms, carbon atoms and nitrogen atoms, and group III or group V atoms in the photosensitive layer of the light receiving layer of the light receiving member according to this invention,

FIGS. 16 through 18 are views illustrating the distribution state, in the direction of the layer thickness, of at least one of the elements selected from oxygen atoms, carbon atoms and nitrogen atoms in the surface layer of the light receiving layer of the light receiving member according to this invention, respectively in which the ordinate represents the thickness of the light receiving layer and the abscissa represents the distribution concentration for each of the atoms;

FIG. 19 is a schematic explanatory view of a fabrication device by glow discharging process as an example of the device for preparing the light receiving layer of the light receiving member according to this invention;

FIGS. 20A and 20B are views for illustrating the image exposing device by the laser beams; and

FIGS. 21 through 45 are views illustrating the variations in the gas flow rates in forming the light receiving layer according to this invention, in which the ordinate represents the position along the layer thickness and the abscissa represents the gas flow rate.

#### DETAILED DESCRIPTION OF THE INVENTION

The present inventors have made earnest studies for overcoming the foregoing problems on the conventional light receiving members and attaining the objects as described above and, as a result, have accomplished this invention based on the findings as described below.

That is, one of the findings is that the problems for the interference fringe pattern occurring upon image formation in the light receiving member having a plurality of layers on a support can be significantly overcome by disposing unevenness constituted with a plurality of spherical dimples each of which having an inside face provided with minute irregularities on the surface of the support.

Another finding is that in a case where the optical band gap possessed by a surface layer and the optical band gap possessed by a photosensitive layer to which the surface layer is disposed directly are matched at the interface between the surface layer and the photosensitive layer, in the light receiving member comprising the surface layer and the photosensitive layer on the support, the reflection of the incident light at the interface between the surface layer and the photosensitive layer can be prevented and the problems such as the interference fringe or uneven sensitivity resulting from the uneven layer thickness upon forming the surface layer and/or uneven layer thickness due to the abrasion of the surface layer can be significantly overcome.

A further finding is that in a case where the surface layer is constituted as a multi-layered structure having an abrasion-resistant layer at the outermost side and at least the reflection preventive layer in the inside of the light receiving member comprising the surface layer and the photosensitive layer on the support, the reflection of the incident light at the interface between the surface layer and the photosensitive layer can be significantly prevented and the problems such as the interference fringe or uneven sensitivity resulting from the uneven layer thickness upon forming the surface layer and/or uneven layer thickness due to the abrasion of the surface layer can be significantly overcome.

This invention has been accomplished based on the findings as described above, and one of the aspect thereof resides in a light receiving member comprising a support and a light receiving layer of a multi-layered structure at least having a photosensitive layer composed of amorphous material containing silicon atoms, and at least one of elements selected from oxygen atoms, carbon atoms and nitrogen atoms, wherein the support has a surface provided irregularities composed of spherical dimples each of which having an inside face provided with minute irregularities.

Another aspect of this invention resides in a light receiving member comprising a support and a light receiving layer constituted by a photosensitive layer composed of amorphous material based on silicon atoms and a surface layer, wherein the support has a surface provided with irregularities composed of a plurality of

spherical dimples each of which having an inside face provided with minute irregularities.

A further aspect of this invention resides in a light receiving member comprising a support and a light receiving layer constituted by a photosensitive layer composed of amorphous material containing silicon atoms, and at least one of elements selected from oxygen atoms, carbon atoms and nitrogen atoms and a surface layer, wherein the support has a surface provided with irregularities composed of a plurality of spherical dimples each of which having an inside face provided with minute irregularities.

A still further aspect of this invention resides in a light receiving member comprising a support and a light receiving layer constituted by a photosensitive layer composed of amorphous material at least containing silicon atoms and a surface layer composed of amorphous material containing silicon atoms, and at least one of elements selected from oxygen atoms, carbon atoms and nitrogen atoms, wherein optical band gaps are matched at the interface between the photosensitive layer and the surface layer, and the support has a surface provided with irregularities composed of a plurality of spherical dimples each of which has an inside face provided with minute irregularities.

A still further aspect of this invention resides in a light receiving member comprising a support and a light receiving layer constituted by a photosensitive material composed of amorphous material at least containing silicon atoms and a surface layer, wherein the surface layer has a multi-layered structure containing an abrasion-resistant layer at the outermost side and at least a reflection preventive layer to the inside, and the support has a surface provided with irregularities composed of a plurality of spherical dimples each of which having an inside face provided with minute irregularities.

Now, the findings regarding the surface shape of the support as described above is based on the facts obtained by various experiments attempted by the present inventors.

For better understanding the above-mentioned facts, the following explanation will be made referring to the drawings.

FIGS. 1(A) through 1(C) are schematic views illustrating typical examples of the layer structure of the light receiving member 100 pertaining to this invention. In all of the cases, the light receiving member is made up of the support 101 and the light receiving layer formed thereon. The support 101 has irregularities resembling a plurality of fine spherical dimples each of which having an inside face provided minute irregularities on the surface thereof. The light receiving layer is formed along the slopes of the irregularities, in which FIG. 1(A) is a schematic view illustrating a first typical example of the layer structure of the light receiving member 100 according to this invention, in which are shown the support 101, a light receiving layer 102, a first layer 102', a second layer 102'' and a free surface 103 of the light receiving layer 102;

FIG. 1(B) is a schematic view illustrating a second typical example of the layer structure of the light receiving member 100 according to this invention, in which are shown the support 101, a photosensitive layer 104, a surface layer 105 and a free surface 103 of the surface layer 105; and

FIG. 1(C) is a schematic view illustrating a third typical example of the layer structure of the light receiving member 100 according to this invention, in

which are shown the support 101, a photosensitive layer 104', a surface layer 105' and a free surface 103 of the surface layer 105'.

FIGS. 2 and 3 are views explaining how the problem of interference fringe pattern is solved in the light receiving member of this invention.

FIG. 3 is an enlarged view of a portion of a conventional light receiving member in which a light receiving layer of a multi-layered structure is deposited on a support the surface of which is regularly roughened. In the drawing, a first layer 301, a second layer 302, a free surface 303 and an interface 304 between the first and the second layers are shown respectively. As shown in FIG. 3, in the case of merely roughening the surface of the support regularly by grinding or like other means, since the light receiving layer is usually formed along the uneven shape at the surface of the support, the inclined surface of the unevenness at the surface of the support and the inclined surface of the unevenness of the light receiving layer are in parallel with each other.

Owing to the parallelism, the following problems always occur, for example, in a light receiving member of a multi-layered structure in which the light receiving layer comprises two layers, that is, a first layer 301 and the second layer 302. Since the interface 304 between the first layer and the second layer is in parallel with the free surface 303, the direction of the reflection light  $R_1$  at the interface 304 and that of the reflection light  $R_2$  at the free surface coincide with each other and, accordingly, an interference fringe is formed depending on the thickness of the second layer.

FIG. 2 is an enlarged view for a portion shown in FIG. 1. As shown in FIG. 2, an uneven shape composed of a plurality of fine spherical dimples are formed at the surface of the support in the light receiving member according to this invention and the light receiving layer thereover is deposited along the uneven shape. Therefore, in the light receiving member of the multi-layered structure, for example, in which the light receiving layer comprises a first layer 201 and a second layer 202, the interface 204 between the first layer 201 and the second layer 202 and the free surface 203 are respectively formed with the uneven shape composed of the spherical dimples along the uneven shape at the surface of the support. Assuming the radius of curvature of the spherical dimples formed at the interface 204 and  $R_1$  and the radius of curvature of the spherical dimples formed at the free surface as  $R_2$ , since  $R_1$  is not identical with  $R_2$ , the reflection light at the interface 204 and the reflection light at the free surface 203 have reflection angles different from each other, that is,  $\theta_1$  is not identical with  $\theta_2$  in FIG. 2 and the direction of their reflection lights are different. In addition, the deviation of the wavelength represented by  $l_1 + l_2 - l_3$  by using  $l_1$ ,  $l_2$ , and  $l_3$  shown in FIG. 2 is not constant but variable, by which a sharing interference corresponding to the so-called Newton ring phenomenon occurs and the interference fringe is dispersed within the dimples. Then, if the interference ring should appear in the microscopic point of view in the images caused by way of the light receiving member, it is not visually recognized.

That is, in a light receiving member having a light receiving layer of multi-layered structure formed on the support having such a surface shape, the fringe pattern resulting in the images due to the interference between lights passing through the light receiving layer and reflecting on the layer interface and at the surface of the

support permits one to obtain a light receiving member capable of forming excellent images.

By the way, the radius of curvature  $R$  and the width  $D$  of the uneven shape formed by the spherical dimples, at the surface of the support of the light receiving member according to this invention constitute an important factor for effectively attaining the advantageous effect of preventing the occurrence of the interference fringe in the light receiving member according to this invention. The present inventors carried out various experiments and, as a result, discovered the following facts.

That is, if the radius of curvature  $R$  and the width  $D$  satisfy the following equation:

$$D/R \geq 0.035$$

0.5 or more Newton rings due to the sharing interference are present in each of the dimples. Further, if they satisfy the following equation:

$$D/R \geq 0.055$$

one or more Newton rings due to the sharing interference are present in each of the dimples.

From the foregoing, it is preferred that the ratio  $D/R$  is greater than 0.035 and, preferably, greater than 0.055 for dispersing the interference fringes which result throughout the light receiving member in each of the dimples, thereby preventing the occurrence of the interference fringe in the light receiving member.

Further, it is desired that the width  $D$  of the unevenness formed by the scraped dimple is about 500  $\mu\text{m}$  at the maximum, preferably, less than 200  $\mu\text{m}$  and, more preferably less than 100  $\mu\text{m}$ .

In addition, it is desired that the height of a minute irregularity to be formed with the inside face of a spherical dimple of the support, namely the surface roughness  $\gamma_{\max}$  of the inside face of the spherical dimple lies in the range of 0.5 to 20  $\mu\text{m}$ . That is, in the case where said  $\gamma_{\max}$  is less than 0.5  $\mu\text{m}$ , a sufficient scattering effect is not provided. And in the case where it exceeds 20  $\mu\text{m}$ , the magnitude of the minute irregularity becomes undesirably greater in comparison with that of the spherical dimple to prevent the spherical dimple from being formed in a desired spherical form which results in a light receiving member that does not prevent sufficiently the occurrence of the interference fringe. In addition to this, when a light receiving layer is deposited on such support, the light receiving member which results, has an undesirably enhanced unevenness which is apt to invite defects in visible images to be formed.

This invention has been completed on the basis of the above-mentioned findings.

The light receiving members according to this invention will now be explained more specifically referring to the drawings.

FIG. 1(A) is a schematic view illustrating a typical layer structure of the light receiving member 100 that embodies the first feature of this invention, in which are shown a support 101 which has a surface provided with irregularities composed of a plurality of spherical dimples each of which having an inside face provided with irregularities, a light receiving layer 102, a first layer 102', a second layer 102'' and a free surface 103. Explanation will be made for the support 101 and the light receiving layer 102.

## SUPPORT 101

The support 101 in the light receiving member according to this invention has a surface with fine unevenness smaller than the resolution power required for the light receiving member and the unevenness is composed of a plurality of spherical dimples each of which having an inside face provided with minute irregularities.

the shape of the surface of the support and an example of the preferred methods of preparing the shape are specifically explained referring to FIGS. 4 and 5 but it should be noted that the shape of the support in the light receiving member of this invention and the method of preparing the same are no way limited only thereto.

15 FIG. 4 is a schematic view for a typical example of the shape at the surface of the support in the light receiving member according to this invention, in which a portion of the uneven shape is enlarged.

In FIG. 4, are shown a support 401, a support surface 402, an irregular shape due to a spherical dimple (spherical cavity pit 403, an inside face of the spherical dimple provided with minute irregularities 404, and a rigid sphere 403' of which surface has irregularities 404'.

20 FIG. 4 also shows an example of the preferred methods of preparing the surface shape of the support. That is, the rigid sphere 403' is caused to fall gravitationally from a position at a predetermined height above the support surface 402 and collides against the support surface 402 thereby forming the spherical dimple having the inside face provided with minute irregularities 404. And a plurality of the spherical dimples 403 each substantially of an almost identical radius of curvature  $R$  and of an almost identical width  $D$  can be formed to the support surface 402 by causing a plurality of the rigid spheres 403' substantially of an identical diameter of curvature  $R'$  to fall from identical height  $h$  simultaneously or sequentially.

25 FIGS. 5(A) through 5(C) show typical embodiments of supports formed with the uneven shape composed of a plurality of spherical dimples each of which having an inside surface provided with minute irregularities at the surface as described above.

30 In FIGS. 5(A) through 5(C), are shown a support 501, a support surface 502, a spherical dimple (spherical cavity pit) having an inside face provided with minute irregularities (not shown) 504 or 504' and a rigid sphere of which surface has minute irregularities (not shown) 503 or 503'.

35 In the embodiment shown in FIG. 5(A), a plurality of dimples (spherical cavity pits) 503, 503, . . . of an almost identical radius of curvature and of an almost identical width are formed while being closely overlapped with each other thereby forming an uneven shape regularly by causing to fall a plurality of spheres 503', 503' . . . regularly

40 from an identical height to different positions at the support surface 502 of the support 501. In this case, it is naturally required for forming the dimples 503, 503, . . . overlapped with each other that the spheres 503', 503', . . . are gravitationally dropped such that the times of collision of the respective spheres 503', 503', . . . to the support surface 502 are displaced from each other.

45 Further, in the embodiment shown in FIG. 5(B), a plurality of dimples 504, 504', . . . having two kinds of diameter of curvature and two kinds of width are formed being densely overlapped with each other to the surface 502 of the support 501 thereby forming an unevenness with irregular height at the surface by dropping two kinds of spheres 503, 503', . . . of different

diameters from the heights identical with or different from each other.

Furthermore, in the embodiment shown in FIG. 5(C) (front elevational and cross-sectional views for the support surface), a plurality of dimples 504, 504, . . . of an almost identical diameter of curvature and plural kinds of width are formed while being overlapped with each other thereby forming an irregular unevenness by causing to fall a plurality of spheres 503, 503, . . . of an identical diameter from the identical height irregularly to the surface 502 of the support 501.

As described above, the uneven shape of the support surface composed of the spherical dimples each of which having an inside face provided with irregularities can be formed preferably by dropping the rigid spheres respectively of a surface provided with minute irregularities to the support surface. In this case, a plurality of spherical dimples having desired radius of curvature and width can be formed at a predetermined density on the support surface by properly selecting various conditions such as the diameter of the rigid spheres, falling height, hardness for the rigid sphere and the support surface or the amount of the fallen spheres. That is, the height and the pitch of the uneven shape formed for the support surface can optionally be adjusted depending on the given purpose by selecting various conditions as described above thereby enabling one to obtain a support having a desired uneven shape with the support surface.

For making the surface of the support into an uneven shape in the light receiving member, a method of forming such a shape by the grinding work by means of a diamond cutting tool using lathe, milling cutter, etc. has been proposed, which will be effective to some extent. However, the method leads to problems in that it requires the use of cutting oils, removal of cutting dusts inevitably resulting during cutting work and removal of the cutting oils remaining on the cut surface, which complicates the fabrication and reduce the working efficiency. In this invention, since the uneven surface shape of the support is formed by the spherical dimples as described above, a support having the surface with a desired uneven shape can conveniently be prepared with no problems as described above at all.

The support 101 for use in this invention may either be electroconductive or insulative. The electroconductive support can include, for example, metals such as NiCr, stainless steels, Al, Cr, Mo, Au, Nb, Ta, V, Ti, Pt and Pb or the alloys thereof.

The electrically insulative support can include, for example, films or sheets of synthetic resins such as polyester, polyethylene, polycarbonate, cellulose acetate, polypropylene, polyvinyl chloride, polyvinylidene chloride, polystyrene, and polyamide, glass, ceramic and paper. It is preferred that the electrically insulative support is applied with electroconductive treatment to at least one of the surfaces thereof and disposed with a light receiving layer on the thus treated surface.

In the case of glass, for instance, electroconductivity is applied by disposing, at the surface thereof, a thin film made of NiCr, Al, Cr, Mo, Au, Ir, Nb, Ta, V, Ti, Pt, Pd,  $In_2O_3$ ,  $SnO_2$ , ITO( $In_2O_3 + SnO_2$ ), etc. In the case of the synthetic resin film such as a polyester film, the electroconductivity is provided to the surface by disposing a thin film of metal such as NiCr, Al, Ag, Pv, Zn, Ni, Au, Cr, Mo, Ir, Nb, Ta, V, Tl and Pt by means of vacuum deposition, electron beam vapor deposition, sputtering, etc. or applying lamination with the metal to the sur-

face. The support may be of any configuration such as cylindrical, belt-like or plate-like shape, which can be properly determined depending on the application uses. For instance, in the case of using one of the light receiving members as shown in FIGS. 1(A) through 2(C) as image forming member for use in electronic photography, it is desirably configured into an endless belt or cylindrical form in the case of continuous high speed reproduction. The thickness of the support member is properly determined so that the light receiving member as desired can be formed. In the case flexibility is required for the light receiving member, it can be made as thin as possible within a range capable of sufficiently providing a function as the support. However, the thickness is usually greater than 10  $\mu m$  in view of the fabrication and handling or mechanical strength of the support.

Explanation will then be made to one embodiment of a device for preparing the support surface in the case of using the light receiving member according to this invention as the light receiving member for use in electronic photography while referring to FIGS. 6(A) and 6(B). But this invention is no way limited only thereto.

In the case of the support for the light receiving member for use in electrophotography, a cylindrical substrate is prepared as a drawn tube obtained by applying usual extruding work to aluminum alloy or the like other material into a boat hall tube or a mandrel tube and further applying drawing work, followed by optical heat treatment or tempering. Then, an uneven shape is formed at the surface of the support as the cylindrical substrate by using the fabrication device as shown in FIG. 6(A) and 6(B). The rigid sphere to be used for forming the uneven shape as described above at the support surface can include, for example, various kinds of rigid spheres made of stainless steels, aluminum, steels, nickel and brass and like other metals, ceramics and plastics. Among all, rigid spheres of stainless steels or steels are preferred in view of the durability and the reduced cost. The hardness of such sphere may be higher or lower than that of the support.

However, in the case of the rigid sphere repeatedly used, it is desired that the hardness is higher than that of the support.

In order to form the particular shape as above mentioned for the support surface, it is necessary to use a rigid sphere of a surface provided with minute irregularities.

Such rigid sphere may be prepared properly in accordance with a mechanical treatment method such as a method utilizing plastic processing treatment such as embossing and wave adding and a surface roughening method such as satin finishing or a chemical treatment method such as acid etching or alkali etching.

And the shape (height) or the hardness of the irregularities as formed on the surface of the rigid sphere may be adjusted properly by subjecting the rigid sphere to the surface treatment in accordance with electropolishing, chemical polishing or finish polishing, or anodic oxidation coating, chemical coating, planting, vitreous enameling, painting, evaporation film forming or CVD film forming.

FIGS. 6(A) and 6(B) are schematic cross-sectional views for the entire fabrication device, in which are shown an aluminum cylinder 601 for preparing a support, and the cylinder 601 may previously be finished at the surface to an appropriate smoothness. The cylinder 601 is supported by a rotating shaft 602, driven by an

appropriate drive means 603 such as a motor and made rotatable around the axial center. The rotating speed is properly determined and controlled while considering the density of the spherical dimples to be formed and the amount of rigid spheres supplied.

A rotating vessel 604 is supported by the rotating shaft 602 and rotates in the same direction as the cylinder 601 does. The rotating vessel 604 contains a plurality of rigid spheres each of which having a surface provided with minute irregularities 605, 605, . . . . The rigid spheres are held by plural projected ribs 606, 606, . . . being disposed on the inner wall of the rotating vessel 604 and transported to the upper position by the rotating action of the rotating vessel 604. The rigid spheres 605, 605, . . . then continuously fall down and collide against the surface of the cylinder 601 thereby forming a plurality of spherical dimples each of which having an inside face provided with irregularities when the revolution speed of the rotating vessel 605 is maintained at an appropriate rate.

The fabrication device can be structured in the following way. That is, the circumferential wall of the rotating vessel 604 are uniformly perforated so as to allow the passage of a washing liquid to be jetting-like supplied from one or more of a showering pipe 607 being placed outside the rotating vessel 604 thereby having the cylinder 601, the rigid spheres 605, 605, . . . and also the inside of the rotating vessel 604 washed with the washing liquid.

In that case, extraneous matter caused due to a static electricity generated by contacts between the rigid spheres or between the rigid spheres and the inside part of the rotating vessel can be washed away to form a desirable shape to the surface of the cylinder being free from such extraneous matter. As the washing liquid, it is necessary to use such that does not give any dry unevenness or any residue. In this respect, a fixed oil itself or a mixture of it with a washing liquid such as trichloroethane or trichloroethylene are preferable.

#### LIGHT RECEIVING LAYER 102

The light receiving layer 102 is a layer disposed on the support 102 as described above and it comprises an amorphous material based on silicon atoms and, particularly preferably, an amorphous material containing silicon atoms (Si) and at least one of hydrogen atoms(H) and halogen atoms(X) (hereinafter referred to as "a-Si(H,X)") and also, optionally, containing electroconductive substances. The light receiving layer 102 in the light receiving member according to this invention has a multi-layered structure. For instance, in the embodiment shown in FIG. 1(A), it comprises a first layer 102' and a second layer 102" and has a free surface 103 on the side of the light receiving layer opposite to the support.

The halogen atom(X) contained in the light receiving layer includes, specifically, fluorine, chlorine, bromine with iodine, fluorine and chlorine being particularly preferred. The amount of the hydrogen atoms(H), the amount of the halogen atoms(X) or the sum of the amounts for the hydrogen atoms and the halogen atoms (H+X) contained in the light receiving layer 102 is usually from 1 to 40 atm% and, preferably, from 5 to 30 atm%.

In the light receiving member according to this invention, the thickness of the light receiving layer is one of the important factors for effectively attaining the purpose of this invention and a sufficient care has to be

taken therefor upon designing the light receiving member so as to provide the member with desired performances. The layer thickness is usually from 1 to 10  $\mu\text{m}$ , preferably, from 1 to 80  $\mu\text{m}$  and, more preferably, from 5 to 50  $\mu\text{m}$ .

By the way, at least one of the elements selected from oxygen atoms, carbon atoms, nitrogen atoms is contained in the light receiving layer of the light receiving member according to this invention mainly with a purpose of increasing the photosensitivity and the dark resistance of the light receiving member, as well as improving the close bondability between the support and the light receiving layer.

In the case of incorporating at least one of the elements selected from the oxygen atoms, carbon atoms and nitrogen atoms into the light receiving layer 102, it is contained at a uniform distribution or not uniform distribution in the direction of the layer thickness depending on the purpose or the expected effects as described above and, accordingly, the content is also varied depending on them.

That is, in the case of increasing the photosensitivity and dark resistance of the light receiving member, the element is contained at a uniform distribution over the entire layer region of the light receiving layer. In this case, the amount of at least one of the elements selected from carbon atoms, oxygen atoms and nitrogen atoms contained in the light receiving layer may be a relatively small amount.

In the case of improving the close bondability between the support and the light receiving layer, at least one of the elements selected from the carbon atoms, oxygen atoms and nitrogen atoms is contained uniformly in a portion of the layer region at the end of the light receiving layer on the side of the support or the element is contained such that the distribution density of at least one of the elements selected from the carbon atoms, oxygen atoms and nitrogen atoms is higher at the end of the light receiving layer on the side of the support. In this case, the amount of at least one of the elements selected from the oxygen atoms, carbon atoms and nitrogen atoms is made relatively great in order to ensure the improvement for the close bondability with the support.

On the other hand, the amount of at least one of the elements selected from the oxygen atoms, carbon atoms and nitrogen atoms contained in the light receiving layer of the light receiving member according to this invention is also determined while considering the organic relationship such as the performance at the interface in contact with the support, in addition to the performances required for the light receiving layer as described above and it is usually from 0.001 to 50 atm%, preferably, from 0.002 to 40 atm% and, most suitably, from 0.003 to 30 atm%. By the way, in the case of incorporating the element in the entire layer region of the photosensitive layer or the proportion of the layer thickness of the layer region incorporated with the element is greater in the layer thickness of the light receiving layer, the upper limit for the content is made smaller. That is, if the thickness of the layer region incorporated with the element is 2/5 of the thickness for the light receiving layer, the content is usually less than 30 atm%, preferably, less than 20 atm% and, most suitably, less than 10 atm%.

Then, several examples are explained referring to FIGS. 7 through 15 in which a relatively large amount of at least one of the elements selected from oxygen

atoms, carbon atoms and nitrogen atoms are contained in the light receiving layer according to this invention on the side of the support, then the amount is gradually decreased from the end on the side of the support to the end on the side of the free surface and decreased further to a relatively small amount or substantially zero near the end of the light receiving layer on the side of the free surface. However, this invention is no way limited only to these examples. At least one of the elements selected from carbon atoms, oxygen atoms, and nitrogen atoms is referred to hereinafter as "atoms(O,C,N)".

In FIGS. 7 through 15, the abscissa represents the distribution density C of the atoms(O,C,N), the ordinate represent the thickness of the light receiving layer,  $t_B$  represents the position of the interface between the support and the light receiving layer and  $t_T$  represents the position for the free surface of the light receiving layer.

FIG. 7 shows the first typical embodiment of the distribution state of the atoms(O,C,N) contained in the light receiving layer in the direction of the layer thickness. In this embodiment, the distribution density of the atoms (O,C,N) is at a constant value  $C_1$  from the interface position  $t_B$  between the light receiving layer and the support to the position  $t_1$ , the distribution density C is continuously decreased from the density  $C_2$  from the position  $t_1$  to the position  $t_T$  at the free surface and then the distribution density C of the atoms(O,C,N) is decreased to  $C_3$  at the position  $t_T$ .

In another typical embodiment shown in FIG. 8, the distribution density C of the atoms(O,C,N) contained in the light receiving layer is such that the density  $C_4$  is continuously decreased from the position  $t_B$  to the position  $t_T$  where it attains  $C_5$ .

In the embodiment shown in FIG. 9, the distribution density C of the atoms(O,C,N) is kept at a constant value  $C_6$  from the position  $t_B$  to the position  $t_2$ , the distribution density C of the atoms(O,C,N) is continuously decreased gradually from the density  $C_7$  from the position  $t_2$  to the position  $t_T$  and the distribution density C of the atoms(O,C,N) is substantially zero at the position  $t_T$ .

In the embodiment shown in FIG. 10, the distribution density C of the atoms(O,C,N) is continuously decreased from  $C_8$  gradually from the position  $t_B$  to the position  $t_T$  and the distribution density C of the atoms(O,C,N) at the position  $t_T$  is substantially zero.

In the embodiment shown in FIG. 11, the distribution density C of the atoms(O,C,N) is at a constant density  $C_9$  between the position  $t_B$  and the position  $t_3$  and the density is decreased linearly from the density  $C_9$  to a density  $C_{10}$  between the position  $t_3$  and the position  $t_T$ .

In the embodiment shown in FIG. 12, the distribution density C of the atoms(O,C,N) is at constant density  $C_{11}$  from the position  $t_B$  to the position  $t_4$  and the density is decreased linearly from the density  $C_{12}$  to the density  $C_{13}$  between the position  $t_4$  and the position  $t_T$ .

In the embodiment FIG. 13, the distribution density C of the atoms(O,C,N) is decreased along linearly till the density  $C_{14}$  is decreased to substantially zero from the position  $t_B$  to the position  $t_T$ .

In the embodiment shown in FIG. 14, the distribution density C of the atoms(O,C,N) is decreased linearly till the density  $C_{15}$  is decreased to the density  $C_{16}$  and from the position  $t_B$  to the position  $t_5$  then kept at a constant density  $C_{16}$  from the position  $t_5$  to the position  $t_T$ .

Finally in the embodiment shown in FIG. 15, the distribution density C of the atoms(O,C,N) is at a den-

sity  $C_{17}$  at the position  $t_B$ , gradually decreased initially from the density  $C_{17}$  and rapidly decreased to a density  $C_{18}$  near the position  $t_6$  and then decreased at the position  $t$  (from the position  $t_5$  to the position  $t_6$ ). Then, from the position  $t_6$  to the position  $t_7$ , the density is initially decreased rapidly and, thereafter, gradually decreased slowly to a density  $C_{19}$  at the position  $t_7$ . Further, between the position  $t_7$  and the position  $t_8$ , the density is decreased extremely gradually to a density  $C_{20}$  at the position  $t_8$ . Further, the density is gradually decreased from the density  $C_{20}$  substantially to zero from the position  $t_6$  to the position  $t_T$ .

As shown by the embodiments shown in FIGS. 7 through 15, in the case where the distribution density C of the atoms(O,C,N) is higher at the end of the light receiving layer on the side of the support, while the distribution density C is considerably lower or substantially equal to zero at the end of the first layer on the side of the free surface, improvement in the close bondability between the support and the light receiving layer can be attained more effectively by disposing a localized region at the end of the light receiving layer on the side of the support where the distribution density of the atoms(O,C,N) is relatively higher and, preferably, by disposing the localized region at a position within 5 um from the interface position  $t_B$  between the support surface and the light receiving layer.

The localized region may be disposed partially or entirely at the end of the light receiving layer to be contained with the atoms(O,C,N) on the side of the support, which may be properly determined in accordance with the performances required for the light receiving layer to be formed. It is desired that the amount of the atoms(O,C,N) contained in the localized region is such that the maximum value of the distribution density C of the atoms(O,C,N) is greater than the 500 atm ppm, preferably, greater than 800 atm ppm and, most suitably, greater than 1000 atm ppm in the distribution.

In the light receiving member according to this invention, substance for controlling the electroconductivity may be contained to the light receiving layer 102 in a uniform or not-uniform distributed state to the entire or partial layer region.

As the substance for controlling the conductivity, so-called impurities in the field of the semiconductor can be mentioned and those usable herein can include atoms belonging to the group III of the periodical table that provide P-type conductivity (hereinafter simply referred to as "group III atom") or atoms belonging to the group V of the periodical table that provide n-type conductivity (hereinafter simply referred to as "group V atom"). Specifically, the group III atoms can include B (boron), Al (aluminum), Ga (gallium), In (indium) and Ti (thallium), B and Ga being particularly preferred. The group V atoms can include, for example, P (phosphor), As (arsenic), Sb (antimony) and Bi (bismuth), P and Sb being particularly preferred.

In the case of incorporating the group III or group V atoms as the substance for controlling the conductivity into the light receiving layer according to this invention, they are contained in the entire layer region or partial layer region depending on the purpose or the expected effects as described below and the content is also varied.

That is, if the main purpose resides in the control for the conduction type and/or conductivity of the light receiving layer, the substance is contained in the entire

layer region of the photosensitive layer, in which the content of group III or group V atoms may be relatively small and it is usually from  $1 \times 10^{-3}$  to  $1 \times 10^3$  atm ppm, preferably from  $5 \times 10^{-2}$  to  $5 \times 10^2$  atm ppm and, most suitably, from  $1 \times 10^{-1}$  to  $2 \times 10^2$  atm ppm.

In the case of incorporating the group III or group V atoms in a uniform distributed state to a portion of the layer region in contact with the support, or the atoms are contained such that the distribution density of the group III or group V atoms in the direction of the layer thickness is higher on the side adjacent with the support, a partial layer region containing such group III or group V atoms or the region containing them at a higher density functions as a charge injection inhibition layer. That is, in the case of incorporating the group III atoms, movement of electrons injected from the side of the support into the light receiving layer can effectively be inhibited upon applying the charging treatment of at positive polarity at the free surface of the light receiving layer. While on the other hand, in the case of incorporating the group III atoms, movement of positive holes injected from the side of the support into the light receiving layer can effectively be inhibited upon applying the charging treatment at negative polarity at the free surface of the light receiving layer. The content in this case is relatively great. Specifically, it is generally from 30 to  $5 \times 10^4$  atm ppm, preferably, from 50 to  $1 \times 10^4$  atm ppm and, most suitably, from  $1 \times 10^2$  to  $5 \times 10^3$  atm ppm. Then, for effectively attaining the foregoing effect, it is desirable that the relationship:  $t/t+t_0 \leq 0.4$  is established between the layer thickness  $t$  for the portion of the layer region or the layer region containing the substance at a high density and the layer thickness  $t_0$  for the photosensitive layer other than above. More preferably, the value for the relationship is less than 0.35 and, most suitably, less than 0.3. Further, the thickness of the layer region is generally from  $3 \times 10^{-3}$  to  $10\mu$ , preferably,  $4 \times 10^{-5}$  to  $8\mu$  and, most suitably, from  $5 \times 10^{-5}$  to  $5\mu$ .

Further, typical embodiments in which the group III or group V atoms incorporated into the light receiving layer is so distributed that the amount therefor is relatively great on the side of the support, decreased from the support toward the free surface and is relatively smaller or substantially equal to zero near the end on the side of the free surface can be explained by the same embodiments as those in FIGS. 7 through 15 that exemplify those cases of incorporating at least one of the elements selected from oxygen atoms, carbon atoms and nitrogen atoms to the light receiving layer as described above. However, this invention is no way limited only to these embodiments.

As shown in the embodiments of FIGS. 7 through 15, in the case where the distribution density C of the group III or group V atoms is higher at the portion of the light receiving layer near the side of the support, while the distribution density C is considerably lower or substantially reduced to zero in the portion of the light receiving layer on the side of the free surface, the foregoing effect that the layer region where the group III or group V atoms are distributed at a higher density can form the charge injection inhibition layer as described above more effectively, by disposing a localized region where the distribution density of the group III or group V atoms is relatively higher at the portion near the side of the support, preferably, by disposing the localized region at a position within  $5\mu$  from the interface position in adjacent with the support surface.

While the individual effects have been described above for the distribution state of the group III or group V atoms, the distribution state of the group III or group V atoms and the amount of the group III or group V atoms are, of course, combined properly as required for obtaining the light receiving member having performances capable of attaining a desired purpose. For instance, in the case of disposing the charge injection inhibition layer at the end of the light receiving layer on the side of the support, a substance for controlling the conductivity of a polarity different from that of the substance for controlling the conductivity contained in the charge injection inhibition layer may be contained in the light receiving layer other than the charge injection inhibition layer, or a substance for controlling the conductivity of the same polarity may be contained by an amount substantially smaller than that contained in the charge inhibition layer.

Further, in the light receiving member according to this invention, a so-called barrier layer composed of electrically insulating material may be disposed instead of the charge injection inhibition layer as the constituent layer disposed at the end on the side of the support, or both of the barrier layer and the charge injection inhibition layer may be disposed as the constituent layer. The material for constituting the barrier layer can include, for example, those inorganic electrically insulating materials such as  $\text{Al}_2\text{O}_3$ ,  $\text{SiO}_2$  and  $\text{Si}_3\text{N}_4$  or organic electrically insulating material such as polycarbonate.

FIG. 1(B) is a schematic view for illustrating the typical layer structure of the light receiving member that embodies the second aspect of this invention, in which are shown a light receiving member 100, a support 101, a free surface 103, a photosensitive layer 104 and a surface layer 105. As shown in FIG. 1(B), the light receiving member in this embodiment is different from the light receiving layer that embodies the first aspect of this invention shown in FIG. 1(A) as described above in that it comprises a light receiving layer having the photosensitive layer 104 and the surface layer 105 on the support 101 and identical with the embodiment shown in FIG. 1(A) with respect to the support 101.

Explanation will then be made to the photosensitive layer 104 and the surface layer 105.

#### PHOTOSENSITIVE LAYER 104

The photosensitive layer 104 is a layer disposed on the support 101 and it comprises an amorphous material based on silicon atoms and, preferably, an amorphous material containing silicon atoms (Si) and at least one of hydrogen atoms (H) or halogen atoms (X) (hereinafter referred to as "a-Si(H,X)"). The photosensitive layer 104 preferably contains further a substance for controlling the conductivity. The photosensitive layer 104 may be multilayered structure and, particularly preferably, it includes a so-called barrier layer composed of a charge injection inhibition layer and/or electrically insulating material containing a substance for controlling the conductivity as one of the constituent layers.

The halogen atoms and the substance for controlling the conductivity contained in the photosensitive layer 104 is the same as those contained in the light receiving layer 101 shown in FIG. 1(A). The photosensitive layer is the same as the light receiving layer 102 shown in FIG. 1(A) also with respect to the constitution in that a barrier layer composed of a charge injection inhibition

layer containing group III atoms or group V atoms at a high concentration and/or electrically insulating material is disposed to the photosensitive layer 104 on the side in adjacent with the support 101.

#### SURFACE LAYER 105

The surface layer 105 is disposed on the photosensitive layer 104 as described above and the surface layer is generally grouped into the following four types.

One of them is constituted with a-Si(H,X) containing oxygen atoms in a uniformly distributed state (that is a-SiO(H,X)).

The surface layer 104 is disposed to the light receiving layer according to this invention with an aim of improving the moisture-proofness, performance for continuous repeating use, electrical voltage withstanding property, circumstantial resistance property and durability, and these purposes can be attained by incorporating oxygen atoms in the amorphous material constituting the surface layer.

Further, in the light receiving member according to this invention, since each of the amorphous layers constituting the photosensitive layer 104 and the surface layer 105 contains common constituent atoms of silicon, a chemical stability can be ensured at the interface between the photosensitive layer 104 and the surface layer 105.

The oxygen atoms are contained in a uniformly distributed state in the surface layer 105, by which the foregoing various properties can be improved in accordance with the increase in the content of the oxygen atoms. However, if the content is excessive, the layer quality is reduced and electrical and mechanism properties are also degraded. In view of the above, the amount of the hydrogen atoms is usually from 0.001 to 90 atm%, preferably, from 1 to 90 atm% and, most suitably, from 10 to 80 atm%.

It is desired that either one of the hydrogen atoms or halogen atoms is contained also in the surface layer and the amount of the hydrogen atoms(H), the amount of the halogen atoms(X) or the sum of the amounts for the hydrogen and the halogen atoms(H+X) contained in the surface layer 105 is usually from 1 to 40 atm%, preferably, from 5 to 30 atm% and, most suitably, from 5 to 25 atm%.

The surface layer 105 has to be formed with an utmost care so as to obtain the properties as desired. That is, the state of the substance comprising silicon atoms, oxygen atoms and, further, hydrogen atoms and/or halogen atoms as the constituent atoms is from crystalline to amorphous state, the electrical property of the layer may vary from the conductive, to semiconductivity and insulating property and, further, the photoelectrical property of the layer may also vary from photoconductive to non-photoconductive property depending on the content of each of the constituent atoms and other conditions of preparation. Accordingly, it is essential to select the content for each of the constituent atoms and the preparation conditions such that the surface layer 105 having desired properties depending on the purpose can be formed.

For instance, in the case of disposing the surface layer 105 mainly for improving the electrical voltage withstanding property, the amorphous material constituting the surface layer 105 is formed such that it exhibits remarkable electrically insulating behavior under the working conditions. Further, in the case of disposing the surface layer 105 mainly for improving the proper-

ties in the continuous repeating use or the circumstantial-resistant property, the amorphous layer constituting the surface layer 105 is formed such that the layer has a photosensitivity to some extent to the irradiated light, although the degree of the electrically insulating property is somewhat moderated.

In this invention, the thickness of the surface layer is also one of the important factors for effectively attaining the purpose of this invention and it is properly determined depending on the desired purposes. It is, however, also necessary that the layer thickness is determined in view of relative and organic relationships in accordance with the amounts of the oxygen atoms, halogen atoms and hydrogen atoms contained in the layer or the properties required for the surface layer. Further, it should be determined also in economical point of view such as productivity or mass productivity. In view of the above, the thickness of the surface layer is usually from  $3 \times 10^{-3}$  to  $30\mu$ , preferably, from  $4 \times 10^{-3}$  to  $20\mu$  and, most preferably, from  $5 \times 10^{-3}$  to  $10\mu$ .

The second embodiment for the surface layer 105 comprises a-Si containing at least one of the elements selective from oxygen atoms(O), carbon atoms(C) and nitrogen(N) and, preferably, at least one of the elements of hydrogen atoms(H) and halogen atoms(X) (hereinafter referred to as "a-Si(O,C,N)(H,X)"), and it provides a function of reducing the reflection of the incident light at the free surface 103 of the light receiving member and increasing the transmission rate, as well as a function of improving various properties such as moisture proofness, property for continuous repeating use, electrical voltage withstanding property, circumstantial-resistant property and durability of the light receiving member.

In this case, it is necessary to constitute such that the optical band gap  $E_{opt}$  possessed by the surface layer and the optical band gap  $E_{opt}$  possessed by the photosensitive layer 104 directly disposed with the surface layer are matched at the interface between the surface layer 105 and the photosensitive layer 104, or such optical band gaps are matched to such an extent as capable of substantially preventing the reflection of the incident light at the interface between the surface layer 105 and the photosensitive layer 104.

Further, in addition to the conditions as described above, it is desirable to constitute such that the optical band gap  $E_{opt}$  possessed by the surface layer is sufficiently larger at the end of the surface layer 105 on the side of the free surface for ensuring a sufficient amount of the incident light reaching the photosensitive layer 104 disposed below the surface layer. Then, in the case of adapting the optical band gaps at the interface between the surface layer 105 and the photosensitive layer 104, as well as making the optical band gap  $E_{opt}$  sufficiently larger at the end of the surface layer on the side of the free surface, the optical band gap possessed by the surface layer is continuously varied in the direction of the thickness of the surface layer.

The value of the optical band gap  $E_{opt}$  of the surface layer in the direction of the layer thickness is controlled by controlling, the content of at least one of the elements selected from the oxygen atoms(O), carbon atoms(C) and nitrogen atoms(N) as the atoms for adjusting the optical band gaps contained in the surface layer is controlled.

Specifically, the content of at least one of the elements selected from oxygen atoms(O), carbon atoms(C) and nitrogen atoms(N) (hereinafter referred to as

"atoms(O,C,N)" is adjusted nearly or equal to zero at the end of the photosensitive layer in adjacent with the surface layer.

Then, the amount of the atoms(O,C,N) is continuously increased from the end of the surface layer on the side of the photosensitive layer to the end on the side of the free surface and a sufficient amount of atoms(O,C,N) to prevent the reflection of the incident light at the free surface is contained near the end on the side of the free surface. Hereinafter, several typical examples for the distributed state of the atoms(O,C,N) in the surface layer are explained referring to FIGS. 16 through 18, but this invention is no way limited only to these embodiments.

In FIGS. 16 through 18, the abscissa represents the distribution density C of the atoms(O,C,N) and silicon atoms and the ordinate represents the thickness t of the surface layer, in which  $t_7$  is the position for the interface between the photosensitive layer and the surface layer,  $t_F$  is a position for the free surface, the solid line represents the variation in the distribution density of the atoms(O,C,N) and the broken line shows the variation in the distribution density of the silicon atoms(Si).

FIG. 16 shows a first typical embodiment for the distribution state of the atoms(O,C,N) and the silicon atoms(Si) contained in the surface layer in the direction of the layer thickness. In this embodiment, the distribution density C of the atoms(O,C,N) is increased till the density is increased from zero to a density  $C_1$  from the interface position  $t_7$  to the position  $t_1$  linearly. While on the other hand, the distribution density of the silicon atoms is decreased linearly from a density  $C_2$  to a density  $C_3$  from the position  $t_1$  to the position  $t_F$ . The distribution density C for the atoms(O,C,N) and the silicon atoms are kept at constant density  $C_1$  and density  $C_3$  respectively.

In the embodiment shown in FIG. 17, the distribution density C of the atoms(O,C,N) is increased linearly from the density zero to a density  $C_4$  from the interface position  $t_7$  to the position  $t_3$ , while it is kept at a constant density  $C_4$  from the position  $t_3$  to the position  $t_F$ . While on the other hand, the distribution density C of the silicon atoms is decreased linearly from a density  $C_5$  to a density  $C_6$  from the position  $t_7$  to the position  $t_2$ , decreased linearly from the density  $C_6$  to a density  $C_7$  from the position  $t_2$  to the position  $t_3$ , and kept at the constant density  $C_7$  from the position  $t_3$  to the position  $t_F$ . In the case where the density of the silicon atoms is high at the initial stage of forming the surface layer, the film forming rate is increased. In this case, the film forming rate can be compensated by decreasing the distribution density of the silicon atoms in the two steps as in this embodiment.

In the embodiment shown in FIG. 18, the distribution density of the atoms(O,C,N) is continuously increased from zero to a density  $C_8$  from the position  $t_7$  to the position  $t_4$ , while the distribution density C of the silicon atoms(Si) is continuously decreased from a density  $C_9$  to a density  $C_{10}$ . The distribution density of the atoms(O,C,N) and the distribution density of the silicon atoms(Si) are kept at a constant density  $C_8$  and a constant density  $C_{10}$  respectively from the position  $t_4$  to the position  $t_F$ . In the case of continuously increasing the distribution density of the atoms(O,C,N) gradually as in this embodiment, the variation coefficient of the reflective rate in the direction of the layer thickness of the surface layer can be made substantially constant.

As shown in FIGS. 16 through 18, in the surface layer of the light receiving member according to this invention, it is desired to dispose a layer region in which the distribution density of the atoms(O,C,N) is made substantially zero at the end of the surface layer on the side of the photosensitive layer, increased continuously toward the free surface and made relatively high at the end of the surface layer on the side of the free surface. Then, the thickness of the layer region in this case is usually made greater than  $0.1 \mu\text{m}$  for providing a function as the reflection preventive layer and a function as the protecting layer.

It is desired that at least one of the hydrogen atoms and the halogen atoms are contained also in the surface layer, in which the amount of the hydrogen atoms(H), the amount of the halogen atoms(X) or the sum of the hydrogen atoms and the halogen atoms (H+X) are usually from 1 to 40 atm%, preferably, from 5 to 30 atm% and, most suitably, from 5 to 25 atm%.

Further, in this invention, the thickness of the surface layer is also one of the most important factors for effectively attaining the purpose of the invention, which is properly determined depending on the desired purposes. It is required that the layer thickness is determined in view of the relative and organic relationship in accordance with the amount of the oxygen atoms, carbon atoms, nitrogen atoms, halogen atoms and hydrogen atom contained in the surface layer or the properties required for the surface layer. Further, it should be determined also from the economical point of view such as productivity and mass productivity. In view of the above, the thickness of the surface layer is usually from  $3 \times 10^{-3}$  to  $30\mu$ , preferably, from  $4 \times 10^{-3}$  to  $20\mu$  and, particularly preferably, from  $5 \times 10^{-3}$  to  $10\mu$ .

The third embodiment of the surface layer 105 provides a function of reducing the reflection and increasing the transmission rate at the free surface 104 of the light receiving layer, that is, the reflection preventive function, as well as the function of improving various properties such as the moisture proofness, the property for continuous repeating use, electrical voltage withstanding property, circumstantial resistance and durability of the light receiving member.

Further, the material for forming the surface layer is required to satisfy various conditions in that it can provide the excellent reflection preventive function for the layer constituted therewith, and a function of improving the various properties as described above, as well as those conditions in that it does not give undesired effects on the photoconductivity of the light receiving member, provides an adequate electronic photographic property, for example, an electric resistance over a certain level, provide an excellent solvent resistance in the case of using the liquid developing process and it does not reduce the various properties of the first layer already formed. Those materials that can satisfy such various conditions and can be used effectively include, for example, at least one of materials selected from inorganic fluorides, inorganic oxides and inorganic sulfides such as  $\text{MgF}_2$ ,  $\text{Al}_2\text{O}_3$ ,  $\text{ZrO}_2$ ,  $\text{TiO}_2$ ,  $\text{ZnS}$ ,  $\text{CeO}_2$ ,  $\text{CeF}_3$ ,  $\text{Ta}_2\text{O}_5$ ,  $\text{AlF}_3$  and  $\text{NaF}$ .

Further, for effectively preventing the reflection prevention, it is desired to selectively use those materials capable of satisfying the conditions represented by the equation:

$$n = \sqrt{n_a}$$

where  $n$  represents the refractive index of the material for forming the surface layer and  $n_a$  represents the refractive index of the layer constituting the photosensitive layer laminated directly to the surface layer.

Several examples of the refractive indexes of inorganic fluorides, inorganic oxides and inorganic sulfide or the mixture thereof as described above will now be referred to. The refractive index is varied somewhat depending on the kinds of the layer to be prepared, conditions and the like. Numerical values in the parentheses represent the refractive index.

$ZrO_2$  (2.00),  $TiO_2$  (2.26),  $ZrO_2/TiO_2=6/1$  (2.08),  $TiO_2/ZrO_2=3/1$  (2.20),  $GeO_2$  (2.23),  $ZnS$  (2.24),  $Al_2O_3$  (1.63),  $CeF_3$  (1.60),  $Al_2O_3/ZrO_2=1/1$  (1.66),  $MgF_2$  (1.38).

Further, it is desirable that the thickness  $d$  of the surface layer can satisfy the conditions expressed by the following equation:

$$d = \frac{\lambda}{4n} \quad (n \text{ is a positive odd number})$$

where  $d$  represents the thickness of the surface layer,  $n$  represents the refractive index of the material constituting the surface layer and  $\lambda$  represents the wavelength of the irradiated light. Specifically, in the case where the wavelength of the exposing light is within the wavelength range from the near infrared to the visible rays the thickness  $d$  of the surface layer is preferably defined as from 0.05 to 2  $\mu m$ .

In the last embodiment of the surface layer 105, the surface layer is constituted as a multi-layered structure at least comprising an abrasion-resistant layer at the outermost side and the reflection preventive layer at the inside in order to overcome the problems of the interference fringe or uneven sensitivity resulted from the uneven thickness of the surface layer. That is, in the light receiving member comprising the surface layer of the multi-layered structure, since a plurality of interfaces are resulted in the surface layer and the reflections at the respective interfaces are offset with each other and, accordingly, the reflection at the interface between the surface layer and the light sensitive layer can be decreased, the problem in the prior art that the reflection rate is changed due to the uneven thickness of the surface layer can be overcome.

It is of course possible to constitute the abrasion resistant layer (outermost layer) and the reflection preventive layer (inner layer) for constituting the surface layer as a single layer structure or two or more multi-layered structure provided that the properties required for them can be satisfied.

For constituting the surface layer as such a multi-layered structure, the optical band gaps ( $E_{opt}$ ) of the layer constituting the abrasion-resistant layer (outermost layer) and the reflection preventive layer (inner layer) are made different. Specifically, it is adapted such that the refractive index of the abrasion-resistant layer (outermost layer), the refractive index of the reflection preventive layer (inner layer) and the refractive index of the photosensitive layer to which the surface layer is disposed directly are made different from each other.

Then, the reflection at the interface between the photosensitive layer and the surface layer can be reduced to zero by satisfying the relationship represented by the following equation:

$$n_3 = \sqrt{n_1 \cdot n_2}$$

(where  $n_1 < n_3 < n_2$ )

$$2n_3d = (1+m)\lambda$$

( $m$  represents an integer)

where  $n_1$  is the refractive index of the photosensitive layer,  $n_2$  is a refractive index of the abrasion-resistant layer constituting the surface layer,  $n_3$  is a refractive index of the reflection preventive layer,  $d$  is a thickness of the reflection preventive layer and  $\lambda$  is the wavelength of the incident light.

Although the relationship is defined as:  $n_1 < n_3 < n_2$  in the embodiment described above, the relation is not always limited only thereto but it may, for example, be defined as  $n_1 < n_2 < n_3$ .

Further, the material for forming the surface layer is required to satisfy conditions in that it can provide the function of reducing the reflection of the incident light to the light receiving member and increasing the transmission rate, and improving various properties of the light receiving member such as moisture proofness, property for the continuous repeating use, electrical voltage withstanding property, circumstantial resistance and durability, as well as those conditions in that it does not give undesired effects on the photoconductivity of the light receiving member, provides electro-photographic property, for example, an electrical resistance over a certain level, provides an excellent solvent resistance in the case of using the liquid developing process and it does not reduce the various properties of the photosensitive layer already formed. Those materials that can satisfy such various conditions and can be used effectively include amorphous materials containing silicon atoms(Si) and at least one of the elements selected from oxygen atoms(O), carbon atoms(C) and nitrogen atoms(N) and, preferably, further at least one of hydrogen atoms(H) and halogen atoms(X) (hereinafter referred to as "a-Si(O,C,N)(H,X)"), or at least one of the elements selected from inorganic fluorides, inorganic oxides and inorganic sulfides such as  $MgF_2$ ,  $Al_2O_3$ ,  $ZnS$ ,  $TiO_2$ ,  $ZrO_2$ ,  $CeO_2$ ,  $CeF_3$ ,  $AlF_3$  and  $NaF$ .

In the case of constituting the surface layer with an amorphous material containing silicon atoms, and at least one of the elements selected from oxygen atoms, carbon atoms or nitrogen atoms, the refractive indexes are made different by making the amount of oxygen atoms, carbon atoms or hydrogen atoms contained in the surface layer different between the abrasion-resistant layer and the reflection preventive layer. Specifically, in the case of constituting the photosensitive layer with a-SiH and the surface layer with a-SiCH, the amount of the carbon atoms contained in the abrasion-resistant layer is made greater than the amount of the carbon atoms contained in the reflection preventive layer and the refractive index  $n_1$  of the photosensitive layer, the refractive index  $n_3$  of the reflection preventive layer, the refractive index  $n_2$  of the abrasion-resistant layer and the thickness  $d$  of the abrasion-resistant layer are made as:  $n_1 \approx 2.0$ ,  $n_2 \approx 3.5$ ,  $n_3 \approx 2.65$  and  $d \approx 755 \text{ \AA}$  respectively. Further, by making the amount of the oxygen atoms, carbon atoms or nitrogen atoms contained in the surface layer different between the abrasion-resistant layer and the reflection preventive layer, the refractive indexes in each of the layers can be made different. Specifically, the abrasion-resistant layer can be formed with a-SiC(H,X) and the reflection preven-

tive layer can be formed with a-SiN(N,X) or a-SiO(H,X).

At least one of the elements selected from the oxygen atoms, carbon atoms and nitrogen atoms is contained in a uniformly distributed state in the abrasion-resistant layer and the reflection preventive layer constituting the surface layer. The foregoing various properties can be improved along with the increase in the amount of these atoms contained. However, if the amount is excessive, the layer quality is lowered and the electrical and mechanical properties are also degraded. In view of the above, the amount of these atoms contained in the surface layer is defined as usually from 0.001 to 90 atm%, preferably, from 1 to 90 atm% and, most suitably, from 10 to 80 atm%. Further, it is desirable that at least one of the hydrogen atoms and halogen atoms is contained in the surface layer, in which the amount of the hydrogen atoms(H), the amount of the halogen atoms(X) or the sum of the amounts of the hydrogen atoms and the halogen atoms(H+X) contained in the surface layer is usually from 1 to 40 atm%, preferably, from 5 to 30 atm% and, most suitably, from 5 to 25 atm%.

Furthermore, in the case of constituting the surface layer with at least one of the compounds selected from the inorganic fluorides, inorganic oxides and inorganic sulfides, they are selectively used such that the refractive indexes in each of the photosensitive layer, the abrasion-resistant layer and the reflection preventive layer are different and the foregoing conditions can be satisfied while considering the refractive indexes for each of the inorganic compounds exemplified above and the mixture thereof. Numerical values in the parentheses represent the refractive indexes of the inorganic compounds and the mixtures thereof.

ZrO<sub>2</sub> (2.00), TiO<sub>2</sub> (2.26), ZrO<sub>2</sub>/TiO<sub>2</sub>=6/1 (2.09), TiO<sub>2</sub>/ZrO<sub>2</sub>=3/1 (2.20), GeO<sub>2</sub> (2.23), ZnS (2.24), Al<sub>2</sub>O<sub>3</sub> (1.63), GeF<sub>3</sub> (1.60), Al<sub>2</sub>O<sub>3</sub>/ZrO<sub>2</sub>=1/1 (1.68), MgF<sub>2</sub> (1.38). These refractive indexes may of course vary somewhat depending on the kind of the layer prepared and the preparing conditions.

Furthermore, the thickness of the surface layer is one of the important factors for effectively attaining the purpose of this invention and the thickness is properly determined depending on the desired purposes. It is required that the thickness be determined while considering the relative and organic relationships depending on the amount of the oxygen atoms, carbon atoms, nitrogen atoms, halogen atoms and hydrogen atoms contained in the layer or the properties required for the surface layer. Further, the thickness has to be determined also from economical point of view such as the productivity and the mass productivity. In view of the above, the thickness of the surface layer is usually from  $3 \times 10^{-3}$  to  $30\mu$ , more preferably, from  $4 \times 10^{-3}$  to  $20\mu$  and, most preferably,  $5 \times 10^{-3}$  to  $10\mu$ .

FIG. 1(C) is a schematic view for illustrating the typical layer structure of the light receiving member that embodies the third aspect of this invention, in which are shown a light receiving member 100, a support 101, a free surface 103, a photosensitive layer 104' and a surface layer 105'.

As shown in FIG. 1(C), the light receiving member that embodies the third aspect of this invention is identical with the light receiving member illustrated in FIG. 1(B) as described above in that it comprises on the support 101 a light receiving layer having a photosensitive layer and a surface layer. Of course, the support 101 is identical with that shown in FIGS. 1(A) and (B), but the

constituent materials for the photosensitive layer 104' and the surface layer 105' are different from those for the photosensitive layer 104 and the surface layer 105' described above. Explanation will then be made to the photosensitive layer 104' and the surface layer 105'.

#### PHOTOSENSITIVE LAYER 104'

The photosensitive layer 104' is a layer disposed on the support 101 and it comprises an amorphous material containing silicon atoms and at least one of the elements selected from oxygen atoms, carbon atoms and nitrogen atoms and, further preferably, containing either one of hydrogen atoms or halogen atoms (hereinafter referred to as "a-Si (O,C,N)(H,X)") and it further contains, as required, a substance for controlling the conductivity. The photosensitive layer 104' may have a multi-layered structure and, particularly preferably, it comprises a charge injection inhibition layer containing a substance for controlling the conductivity as one of the constituent layers and/or a barrier layer as one of the constituent layers.

The halogen atoms and the content thereof that can be incorporated into the photosensitive layer 104' are the same as those in the case of the light receiving layer 102 and the photosensitive layer 104 as described above. Further, the amount for at least one of the elements selected from oxygen atoms, carbon atoms and nitrogen atoms that can be contained in the light sensitive layer 104' (hereinafter referred to as "atoms(O,C,N)") and the distribution state of the atoms(O,C,N) are identical with the case in the light receiving layer 102 as described above. That is, the atoms (O,C,N) may be contained uniformly in the entire or partial region layer of the photosensitive layer 104' or, alternatively, they may be contained not uniformly to the entire or a partial layer region of the photosensitive layer 104', specifically, as shown in FIGS. 7 through 16 for instance.

Further, the amount of the substance for controlling the conductivity that can be incorporated into the photosensitive layer 104', that is, the amount of the group III atoms or group V atoms, as well as the distribution state thereof are identical as those in the case of the light receiving layer 102 and the photosensitive layer 104.

Furthermore, a charge injection inhibition layer containing the group III atoms or group V atoms at a high density and/or a barrier layer comprising an electrically insulating material can also be disposed to the photosensitive layer 104' on the side of the support in the same way as in the light receiving layer 102 shown in FIG. 1(A) and the photosensitive layer 104 shown in FIG. 1(B).

#### SURFACE LAYER 105'

The surface layer 105' is a layer disposed on the photosensitive layer 104' as described above and the surface layer 105' can generally be divided into the following four types.

The first embodiment comprises an amorphous silicon containing at least one of the elements selected from oxygen atoms, carbon atoms or nitrogen atoms not contained in the first layer in a uniformly distributed state (hereinafter referred to as "a-Si(O,C,N)(H,X)"). The surface layer 105' is disposed for improving the moisture-proofness property for continuous repeating use, electrical voltage withstanding property, circumstantial resistance and durability. These purposes can be attained by incorporating at least one of the oxygen

atoms, carbon atoms or nitrogen atoms into the amorphous material constituting the surface layer.

Since each of the amorphous materials constituting the surface layer 105' and the photosensitive layer 104' comprises common constituent atoms of silicon, a chemical stability can be ensured at the interface between the surface layer 105' and the photosensitive layer 104'.

The oxygen atoms, carbon atoms and nitrogen atoms are contained in a uniformly distributed state in the surface layer 105', in which the various properties as described above are improved along with the increase in the amount of these atoms contained. However, if the amount is excessive, the layer quality is lowered and electrical and mechanical properties are also degraded. In view of the above, the content of the atoms is defined usually from 0.001 to 90 atm%, preferably, from 1 to 90 atm% and, most suitably, from 10 to 80 atm%.

It is desired that at least one of the hydrogen atoms and halogen atoms is contained also in the surface layer 105', in which the amount of the hydrogen atoms(H), the amount of the halogen atoms(X) or the sum of the amounts of the hydrogen atoms and the halogen atoms (H+X) contained in the surface layer 105' is usually from 1 to 40 atm%, preferably, from 5 to 30 atm% and, most suitably, from 5 to 25 atm%.

The surface layer has to be formed with an utmost care so that properties can be obtained as desired. That is, since the material comprising silicon atoms and at least one of the elements selected from oxygen atoms, carbon atoms and nitrogen atom and, further, hydrogen atoms and/or halogen atoms as the constituent atoms varies from the crystalline to amorphous state in the form, from the conductive to semiconductive or insulating property in the electrical property and from the photoconductive to non-photoconductive property in the photoconductive property respectively. Accordingly, it is important to select the content for each of the constituent atoms and the preparing conditions so that a surface layer having desired properties depending on the purposes can be formed.

For instance, in the case of disposing the surface layer mainly for improving the electrical voltage withstanding property, the amorphous material constituting the surface layer 105' is formed as showing remarkable electrical insulating behaviors under the working conditions. Further, in the case of disposing the surface layer mainly for improving the property of the continuous repeating use or the circumstantial resistance the amorphous material constituting the surface layer 105' is formed so as to provide a certain level of photosensitivity to the irradiated light, while the degree of the electrical insulating property described above is moderated to some extent.

Furthermore, the thickness of the surface layer 105' is also one of the important factors for effectively attaining the purpose of this invention and it is properly determined depending on the desired purposes. It should also be determined under the relative and organic relationship in accordance with the amount of the oxygen atoms, carbon atoms, nitrogen atoms, halogen atoms and hydrogen atoms or the properties required for the surface layer. In view of the above, the thickness for the surface layer is usually from  $3 \times 10^{-5}$  to  $30\mu$ , more preferably, from  $4 \times 10^{-5}$  to  $20\mu$  and, particularly preferably, from  $5 \times 10^{-5}$  to  $10\mu$ .

The second embodiment of the surface layer 105' comprises an a-Si containing at least one of the elements

selected from oxygen atoms(O), carbon atoms(C) and nitrogen atoms(N) and, further preferably, at least one of the elements selected from hydrogen atoms(H) and halogen atoms(X) (hereinafter referred to as "a-Si(O,C,N)(H,X)'"), which provides a function of decreasing the incident light and increasing the transmission rate at the free surface 103 of the various properties such as receiving member, as well as a function of improving the moisture proofness, property for continuous repeating use, electrical voltage withstanding property, circumstantial resistance and durability of the light receiving member.

In this case, it has to be constituted such that the optical band gap Eopt possessed by the surface layer 105 and the optical band gap Eopt possessed by the photosensitive layer 104' to which the surface layer is directly disposed are matched with each other at the interface between the surface layer 105' and the photosensitive layer 104', or the optical band gaps are matched to such an extent as the reflection of the incident light at the interface between the surface layer 105' and the photosensitive layer 104' can be prevented substantially.

Furthermore, in addition to the conditions described above, it is desired to constitute such that the optical band gap Eopt possessed by the surface layer is made sufficiently greater at the end of the surface layer 105' on the side of the free surface for sufficiently insuring the amount of the incident light reaching the photosensitive layer 104' disposed below the surface layer at the end of the surface layer 105' on the side of the free surface. Then, it is constituted such that the optical band gap Eopt is matched at the interface between the surface layer 105' and the photosensitive layer 104', as well as the optical band gap varies continuously in the direction of the thickness of the surface layer in the case of adapting the optical band gap Eopt to be sufficiently greater at the end of the surface layer on the side of the free surface.

The value of the optical band gap Eopt of the surface layer in the direction of the layer thickness is controlled as described above by controlling the amount of at least one element selected from oxygen atoms(O), carbon atoms(C) and nitrogen atoms(N) to be contained in the surface layer as the adjusting atoms for the optical band gap.

Specifically, in the case where at least one of the elements selected from the oxygen atoms(O), the carbon atoms(C) and the nitrogen atoms(N) (hereinafter referred to as "atoms(O,C,N)") are not contained at the end of the photosensitive layer 104' on the side in adjacent with the surface layer 105', the content of the atoms(O,C,N) at the end of the surface layer in adjacent with the light sensitive layer is made equal or near to zero. While on the other hand, in the case that the atoms(O,C,N) are contained at the end of the photosensitive layer 104' in adjacent with the surface layer 105', the content of the atoms(O,C,N) at the end of the surface layer in adjacent with the light sensitive layer and the content of the atoms(O,C,N) at the end of the photosensitive layer on the side in adjacent with the surface layer are made equal or substantially equal with each other. Then, the amount of the atoms(O,C,N) is continuously increased from the end of the surface layer on the side of the photosensitive layer to the end on the side of the surface layer, and a sufficient amount of atoms(O,C,N) to prevent the reflection of the incident light at the free surface is contained near the end on the

side of the free surface. Several examples of the distribution state of the atoms(O,C,N) in the surface layer will now be explained referring to FIGS. 16 through 18, but this invention is no way limited only to these examples.

In FIGS. 16 through 18, the abscissa represents the distribution density C of the atoms(O,C,N) and the silicon atoms, while the ordinate represents the thickness t of the surface layer, in which,  $t_T$  is an interface position between the photosensitive layer and the surface layer,  $t_F$  is a free surface position, the solid line represents the variation in the distribution density of the atoms(O,C,N) and the broken line shows the variation in the distribution density of the silicon atoms(Si).

FIG. 16 shows a first typical embodiment of the distribution state of the atoms(O,C,N) and the silicon atoms (Si) contained in the surface layer in the direction of the layer thickness. In this embodiment, the distribution density C of the atoms(O,C,N) is increased linearly from zero to a density  $C_1$  from the interface position  $t_T$  to the position  $t_1$ , while the distribution density of the silicon atoms is decreased linearly from a density  $C_1$  to a density  $C_3$ . From the position  $t_1$  to the position  $t_F$ , the distribution density C for the atoms(O,C,N) and the silicon atoms are kept at constant density  $C_1$  and density  $C_3$  respectively.

In the embodiment shown in FIG. 17, the distribution density C for the atoms(O,C,N) is increased linearly from the density zero to a density  $C_4$  from the interface position  $t_T$  to the position  $t_3$  and it is kept at a constant density  $C_4$  from the position  $t_3$  to the position  $t_F$ . While on the other hand, the distribution density C of the silicon atoms is increased linearly from a density  $C_5$  to a density  $C_6$  from the position  $t_T$  to the position  $t_2$ , decreased linearly from the density  $C_6$  to a density  $C_7$  from the position  $t_2$  to the position  $t_3$  and kept at a constant density  $C_7$  from the position  $t_3$  to the position  $t_F$ . In the case where the density of the silicon atoms is higher at the initial stage of forming the surface layer, the film-forming speed is increased. In this case, the film-forming speed can be compensated by decreasing the distribution density for the silicon atoms in two steps as in this embodiment.

In the embodiment shown in FIG. 18, the distribution density of the atoms(O,C,N) is continuously increased from the density zero to a density  $C_8$ , while the distribution density C of the silicon atoms(Si) is continuously decreased from a density  $C_9$  to the density  $C_{10}$  from the position  $t_T$  to the position  $t_4$ . The distribution density of the atoms(O,C,N) and the distribution density of the silicon atoms(Si) kept at constant density  $C_8$  and the density  $C_{10}$  respectively from the position  $t_4$  to the position  $t_F$ . As in this embodiment, in the case of continuously increasing the distribution density of the atoms-(O,C,N) gradually, the variation coefficient for the refractive index in the thickness in the direction of the thickness of the surface layer can be made substantially constant.

In the surface layer 105', it is desirable as shown in FIGS. 16 through 18 that the distribution density of the atoms(O,C,N) is substantially reduced to zero at the end of the surface layer on the side of photosensitive layer, which is continuously increased toward the free surface, and a region layer at a relatively high density is disposed at the end of the surface layer on the side of the free surface. Then, the thickness of the layer region in this case is usually defined so as to be greater than 0.1  $\mu\text{m}$  so as to provide a function as a reflection preventive layer and the function as the protecting layer.

It is desired that at least one of hydrogne atoms and halogen atoms in contained also in the surface layer, in which the amount of the hydrogen atoms(H), the amount of the halogen atoms(X) or the sum of the amounts for the hydrogen atoms and the halogen atoms (H+X) is usually from the 1 to 40 atm%, preferably, 5 to 30 atom% and, most suitably, 5 to 25 atm%.

The thickness of the surface layer 105' is also one of the important factors for effectively attaining the purpose of this invention and it is properly determined depending on the desired purposes. It is also necessary that the thickness is defined under relative and organic relationships depending on the amount of the oxygen atoms, carbon atoms, nitrogen atoms, halogen atoms and hydrogen atoms contained in the layer or depending on the properties required for the surface layer. Further, it should be determined also from the economical point of veiw such as the productivity and the mass productivity.

In view of the above, the thickness for the surface layer is usually from  $3 \times 10^{-3}$  to  $30\mu$ , more preferably, from  $4 \times 10^{-3}$  to  $20\mu$  and, particularly preferably, from  $5 \times 10^{-3}$  to  $10\mu$ .

As the third and the fourth embodiment as the surface layer 105', the third and the fourth embodiment of the surface layer 105 in the photoreceiving member shown in FIG. 1(B) can be used as they are. That is, the third embodiment has a surface layer having a function of preventing reflection and the fourth embodiment provides a surface layer of a multi-layered structure at least comprising an abrasion-resistant layer at the outermost side and a reflection preventive layer to the inside.

By adapting the layer structure of the light receiving member according to this invention as described above, all of the various problems in the light receiving members comprising a light receiving layer constituted with amorphous silicon as described above can be overcome. Particularly, in a case of using the coherent laser beams as an optical source, it is possible to remarkably prevent the occurrence of the interference fringe pattern upon forming images due to the interference phenomenon thereby enabling to obtain reproduced image at high quality.

Further, since the light receiving member according to this invention has a high photosensitivity in the entire visible ray region and, further, since it is excellent in the photosensitive property on the side of the longer wavelength, it is suitable for the matching property, particularly, with a semiconductor laser, exhibits a rapid optical response and shows more excellent electrical, optical and electroconductive natures, electrical voltage withstand property and resistance to working circumstances.

Particularly, in the case of applying the light receiving member to the electrophotography, it gives no undesired effects at all of the residual potential to the image formation, stable electrical properties high sensitivity and high S/N ratio, excellent light fastness and property for repeating use, high image density and clear half tone and can provide high quality image with high resolution power repeatedly.

The method of forming the light receiving layer according to this invention will now be explained.

The amorphous material constituting the light receiving layer in this invention is prepared by vacuum depositing method utilizing the discharging phenomena such as glow discharging, sputtering and ion plating processes. These production processes are properly used

selectively depending on the factors such as the manufacturing conditions, the installation cost required, production scale and properties required for the light receiving members to be prepared. A glow discharging process or sputtering process is suitable since the control for the condition upon preparing the light receiving members having desired properties are relatively easy and carbon atoms and hydrogen atoms can be introduced easily together with silicon atoms. The glow discharging process and the sputtering process may be used together in one identical system.

Basically, when a layer constituted with a-Si(H,X) is formed for example, by the glow discharging process, gaseous starting material for supplying Si capable of supplying silicon atoms(Si) and introduced together with gaseous starting material for introducing hydrogen atoms(H) and/or halogen atoms(X) into a deposition chamber the inside pressure of which can be reduced, glow discharge is generated in the deposition chamber and a layer composed of a-Si(H,X) is formed on the surface of a predetermined support disposed previously at a predetermined position.

The gaseous starting material for supplying Si can include gaseous or gasifiable silicon hydrides (silanes) such as SiH<sub>4</sub>, Si<sub>2</sub>H<sub>6</sub>, Si<sub>3</sub>H<sub>8</sub>, Si<sub>4</sub>H<sub>10</sub>, etc., SiH<sub>4</sub> and Si<sub>2</sub>H<sub>6</sub> being particularly preferred in view of the easy layer forming work and the good efficiency for the supply of Si.

Further, various halogen compounds can be mentioned as the gaseous starting material for introducing the halogen atoms and gaseous or gasifiable halogen compounds, for example, gaseous halogen, halides, inter-halogen compounds and halogen-substituted silane derivatives are preferred. Specifically, they can include halogen gas such as of fluorine, chlorine, bromine and iodine, inter-halogen compounds such as BrF, ClF, ClF<sub>3</sub>, BrF<sub>2</sub>, BrF<sub>3</sub>, IF<sub>7</sub>, ICl, IBr, etc., and silicon halides such as SiF<sub>4</sub>, Si<sub>2</sub>H<sub>6</sub>, SiCl<sub>4</sub>, SiBr<sub>4</sub>. The use of the gaseous or gasifiable silicon halide as described above is particularly advantageous since the layer constituted with halogen atom-containing a-Si can be formed with no additional use of the gaseous starting material for supplying Si.

The gaseous starting material usable for supplying hydrogen atoms can include those gaseous or gasifiable materials, for example, hydrogen gas, halides such as H<sub>2</sub>F, HCl, HBr and HI, silicon hydrides such as SiH<sub>4</sub>, Si<sub>2</sub>H<sub>6</sub>, Si<sub>3</sub>H<sub>8</sub> and Si<sub>4</sub>H<sub>10</sub> or halogen-substituted silicon hydrides such as SiH<sub>2</sub>F<sub>2</sub>, SiH<sub>2</sub>I<sub>2</sub>, SiH<sub>2</sub>Cl<sub>2</sub>, SiHCl<sub>3</sub>, SiH<sub>2</sub>Br<sub>2</sub>, SiHBr<sub>3</sub>. The use of these gaseous starting material is advantageous since the content of the hydrogen atoms(H), which are extremely effective in view of the control for the electrical or photoelectronic properties, can be controlled with ease. Then, the use of the hydrogen halide or the halogen-substituted silicon hydride as described above is particularly advantageous since the hydrogen atoms(H) are also introduced together with the introduction of the halogen atoms.

Further, the amount of the hydrogen atoms(H) and/or halogen atoms(X) contained in the a-Si layer is controlled, for example, by controlling the temperature of the support, the amount of introducing the starting material into the deposition chamber used for introducing the hydrogen atoms (H) and/or halogen atoms(X) and the electrical power for discharging.

In the case of forming layer comprising a-Si(H,X) by means of the reactive sputtering process or ion plating process, for example, by the sputtering process, the

halogen atoms are introduced by introducing gaseous halogen compounds or halogen atom-containing silicon compounds into a deposition chamber thereby forming a plasma atmosphere with the gas.

Further, in the case of introducing the hydrogen atoms, the gaseous starting material for introducing the hydrogen atoms, for example, H<sub>2</sub> or gaseous silanes as described above are introduced into the sputtering deposition chamber thereby forming a plasma atmosphere with the gas.

For instance, in the case of the reactive sputtering process, a layer comprising a-Si(H,X) is formed on a support by using a Si target and by introducing a halogen atom introducing gas and H<sub>2</sub> gas together with an inert gas such as He or Ar as required into a deposition chamber thereby forming a plasma atmosphere and then sputtering the Si target. In the case of forming a layer constituted with an amorphous material composed of a-Si(H,X) further incorporated with group III atoms or group V atoms, nitrogen atoms, oxygen atoms or carbon atoms by using a glow discharging, sputtering or ion plating process, starting material for introducing group III or group V atoms, starting material for introducing nitrogen gas, starting material for introducing oxygen gas or starting material for introducing carbon atoms is used together with the starting material for forming a-Si(H,X) upon forming the a-Si(H,X) layer while controlling the amount of them in the layer to be formed. For instance, in the case of forming a layer or layer region constituted with a-Si(H,X) containing the group III or group V atoms by using the glow discharging, sputtering or ion plating process, the starting material for introducing the group III or group V atoms are used together with the starting material for forming a-Si(H,X) upon forming the layer constituted with a-Si(H,X) as described above and they are incorporated while controlling the amount of them into the layer to be formed.

Referring specifically to the boron atom introducing materials as the starting material for introducing the group III atoms, they can include boron hydrides such as B<sub>2</sub>H<sub>6</sub>, B<sub>4</sub>H<sub>10</sub>, B<sub>5</sub>H<sub>9</sub>, B<sub>5</sub>H<sub>11</sub>, B<sub>6</sub>H<sub>10</sub>, B<sub>6</sub>H<sub>12</sub> and B<sub>6</sub>H<sub>14</sub> and boron halides such as BF<sub>3</sub>, BC<sub>13</sub> and BBr<sub>3</sub>. In addition, AlCl<sub>3</sub>, CaCl<sub>3</sub>, Ga(CH<sub>3</sub>)<sub>2</sub>, InCl<sub>3</sub>, TiCl<sub>3</sub> and the like can also be mentioned.

Referring to the starting material for introducing the group V atoms and, specifically to, the phosphor atom introducing materials, they can include, for example, phosphor hydrides such as PH<sub>3</sub> and P<sub>2</sub>H<sub>6</sub> and phosphor halide such as PH<sub>4</sub>I, PF<sub>3</sub>, PF<sub>5</sub>, PCl<sub>3</sub>, PCl<sub>5</sub>, PBr<sub>3</sub>, PBr<sub>5</sub> and PI<sub>3</sub>. In addition, AsH<sub>3</sub>, AsF<sub>5</sub>, AsCl<sub>3</sub>, AsBr<sub>3</sub>, AsF<sub>3</sub>, SbH<sub>3</sub>, SbF<sub>3</sub>, SbF<sub>5</sub>, SbCl<sub>3</sub>, SbCl<sub>5</sub>, BiH<sub>3</sub>, SiCl<sub>3</sub> and BiBr<sub>3</sub> can also be mentioned to as the effective starting material for introducing the group V atoms.

In the case of using the glow discharging process for forming the layer or layer region containing oxygen atoms, starting material for introducing the oxygen atoms is added to those selected from the group of the starting material as desired above for forming the light receiving layer. As the starting material for introducing the oxygen atoms, most of those gaseous or gasifiable materials can be used that comprise at least oxygen atoms as the constituted atoms.

For instance, it is possible to use a mixture of gaseous starting material comprising silicon atoms(Si) as the constituent atoms, gaseous starting material comprising oxygen atoms(O) as the constituent atom and, as required, gaseous starting material comprising hydrogen

atoms(H) and/or halogen atoms(X) as the constituent atoms in a desired mixing ratio, a mixture of gaseous starting material comprising silicon atoms(Si) as the constituent atoms and gaseous starting material comprising oxygen atoms(O) and hydrogen atoms(H) as the constituent atoms in a desired mixing ratio, or a mixture of gaseous starting material comprising silicon atoms(Si) as the constituent atoms and gaseous starting material comprising silicon atoms(Si), oxygen atoms(O) and hydrogen atoms(H) as the constituent atoms.

Further, it is also possible to use a mixture of gaseous starting material comprising silicon atoms(Si) and hydrogen atoms(H) as the constituent atoms and gaseous starting material comprising oxygen atoms(C) as the constituent atoms.

Specifically, there can be mentioned, for example, oxygen(O<sub>2</sub>), ozone(O<sub>3</sub>), nitrogen monoxide(NO), nitrogen dioxide(NO<sub>2</sub>), dinitrogen oxide(N<sub>2</sub>O), dinitrogen trioxide(N<sub>2</sub>O<sub>3</sub>), dinitrogen tetraoxide(N<sub>2</sub>O<sub>4</sub>), dinitrogen pentoxide(N<sub>2</sub>O<sub>5</sub>), nitrogen trioxide(NO<sub>3</sub>), lower siloxanes comprising silicon atoms(Si), oxygen atoms(O) and hydrogen atoms(H) as the constituent atoms, for example, disiloxane(H<sub>3</sub>SiOSiH<sub>3</sub>) and trisiloxane(H<sub>3</sub>SiOSiH<sub>2</sub>OSiH<sub>3</sub>), etc.

In the case of forming the layer or layer region containing oxygen atoms by way of the sputtering process, it may be carried out by sputtering a single crystal or polycrystalline Si wafer or SiO<sub>2</sub> wafer, or a wafer containing Si and SiO<sub>2</sub> in admixture is used as a target and sputtered in various gas atmospheres.

For instance, in the case of using the Si wafer as the target, a gaseous starting material for introducing oxygen atoms and, optionally, hydrogen atoms and/or halogen atoms is diluted as required with a dilution gas, introduced into a sputtering deposition chamber, gas plasmas with these gases are formed and the Si wafer is sputtered.

Alternatively, sputtering may be carried out in the atmosphere of a dilution gas or in a gas atmosphere containing at least hydrogen atoms(H) and/or halogen atoms(X) as constituent atoms as a sputtering gas by using individually Si and SiO<sub>2</sub> targets or a single Si and SiO<sub>2</sub> mixed target. As the gaseous starting material for introducing the oxygen atoms, the gaseous starting material for introducing the oxygen atoms shown in the examples for the glow discharging process as described above can be used as the effective gas also in the sputtering.

In the case of using the glow discharging process for forming the layer or the layer region containing the nitrogen atoms, starting material for introducing nitrogen atoms is added to the material selected as required from the starting materials for forming the light receiving layer as described above. As the starting material for introducing the nitrogen atoms, most of gaseous or 50 gasifiable materials can be used that comprise at least nitrogen atoms as the constituent atoms.

For instance, it is possible to use a mixture of gaseous starting material comprising silicon atoms(Si) as the constituent atoms, gaseous starting material comprising nitrogen atoms(N) as the constituent atoms and, optionally, gaseous starting material comprising hydrogen atoms(H) and/or halogen atoms(X) as the constituent atoms mixed in a desired mixing ratio, or a mixture of starting gaseous material comprising silicon atoms(Si) as the constituent atoms and gaseous starting material comprising nitrogen atoms(N) and hydrogen atoms(H) as the constituent atoms also in a desired mixing ratio.

Alternatively, it is also possible to use a mixture of gaseous starting material comprising nitrogen atoms(N) as the constituent atoms gaseous starting material comprising silicon atoms(Si) and hydrogen atoms(H) as the constituent atoms.

The starting material that can be used effectively as the gaseous starting material for introducing the nitrogen atoms(N) used upon forming the layer or layer region containing nitrogen atoms can include gaseous or gasifiable nitrogen, nitrides and nitrogen compounds such as azide compounds comprising N as the constituent atoms or N and H as the constituent atoms, for example, nitrogen(N<sub>2</sub>), ammonia(NH<sub>3</sub>), hydrazine(H<sub>2</sub>NNH<sub>2</sub>), hydrogen azide(HN<sub>3</sub>) and ammonium azide(NH<sub>4</sub>N<sub>3</sub>). In addition, nitrogen halide compounds such as nitrogen trifluoride(F<sub>3</sub>N) and nitrogen tetrafluoride(F<sub>4</sub>N<sub>2</sub>) can also be mentioned in that they can also introduce halogen atoms(X) in addition to the introduction of nitrogen atoms(N).

The layer or layer region containing the nitrogen atoms may be formed through the sputtering process by using a single crystal or polycrystalline Si wafer or Si<sub>3</sub>N<sub>4</sub> wafer or a wafer containing Si and Si<sub>3</sub>N<sub>4</sub> in admixture as a target and sputtering them in various gas atmospheres.

In the case of using a Si wafer as a target, for instance, gaseous starting material for introducing nitrogen atoms and, as required, hydrogen atoms and/or halogen atoms is diluted optionally with a dilution gas, introduced into a sputtering deposition chamber to form gas plasmas with these gases and the Si wafer is sputtered.

Alternatively, Si and Si<sub>3</sub>N<sub>4</sub> may be used as individual targets or as a single target comprising Si and Si<sub>3</sub>N<sub>4</sub> in admixture and then sputtered in the atmosphere of a dilution gas or in a gaseous atmosphere containing at least hydrogen atoms(H) and/or halogen atoms(X) as the constituent atoms as for the sputtering gas. As the gaseous starting material for introducing nitrogen atoms, those gaseous starting materials for introducing the nitrogen atoms described previously shown in the example of the glow discharging can be used as the effective gas also in the case of the sputtering.

The light receiving layer containing carbon atoms, for example, may be formed through the glow discharging process, by using a mixture of gaseous starting material comprising silicon atoms(Si) as the constituent atoms, gaseous starting material comprising carbon atoms(C) as the constituent atoms and, optionally, gaseous starting material comprising hydrogen atoms(H) and/or halogen atoms(X) as the constituent atoms in a desired mixing ratio, a mixture of gaseous starting material comprising silicon atoms(Si) as the constituent atoms and gaseous starting material comprising carbon atoms(C) and hydrogen atoms(H) as the constituent atoms also in a desired mixing ratio, a mixture of gaseous starting material comprising silicon atoms(Si) as the constituent atoms and gaseous starting material comprising silicon atoms(Si), carbon atoms(C) and hydrogen atoms(H) as the constituent atoms, or a mixture of gaseous starting material comprising silicon atoms(Si) and hydrogen atoms(H) as the constituent atoms and gaseous starting material comprising carbon atoms(C) as constituent atoms.

The layer or layer region constituted with a SiC(H,X) may be formed through the sputtering process by using a single crystal or polycrystalline Si wafer, a C (graphite) wafer or a wafer containing a mixture of

Si and C as a target and sputtering them in a desired gas atmosphere.

In the case of using, for example a Si wafer as a target, gaseous starting material for introducing carbon atoms, and hydrogen atoms and/or halogen atoms is introduced while being optionally diluted with a dilution gas such as Ar and He into a sputtering deposition chamber thereby forming gas plasmas with these gases and sputtering the Si wafer.

Alternatively, in the case of using Si and C as individual targets or as a single target comprising Si and C in admixture, gaseous starting material for introducing hydrogen atoms and/or halogen atoms as the sputtering gas is optionally diluted with a dilution gas, introduced into a sputtering deposition chamber thereby forming gas plasmas and sputtering is carried out. As the gaseous starting material for introducing each of the atoms used in the sputtering process, those gaseous starting materials used in the glow discharging process as described above may be used as they are.

The gaseous starting materials that are effectively usable herein can include gaseous silicon hydrides comprising C and H as the constituent atoms, such as silanes, for example,  $\text{SiH}_4$ ,  $\text{Si}_2\text{H}_6$ ,  $\text{Si}_3\text{H}_8$  and  $\text{Si}_4\text{H}_{10}$ , as well as those comprising C and H as the constituent atoms, for example, saturated hydrocarbons of 1 to 4 carbon atoms, ethylenic hydrocarbons of 2 to 4 carbon atoms and acetylenic hydrocarbons of 2 to 3 carbon atoms.

Specifically, the saturated hydrocarbons can include 30 methane( $\text{CH}_4$ ), ethane( $\text{C}_2\text{H}_6$ ), propane( $\text{C}_3\text{H}_8$ ), n-butane( $n\text{-C}_4\text{H}_{10}$ ) and pentane( $\text{C}_5\text{H}_{12}$ ), the ethylenic hydrocarbons can include ethylene( $\text{C}_2\text{H}_4$ ), propylene( $\text{C}_3\text{H}_6$ ), butene-1( $\text{C}_4\text{H}_8$ ), butene-2( $\text{C}_4\text{H}_8$ ), isobutylene( $\text{C}_4\text{H}_8$ ) and pentene( $\text{C}_5\text{H}_{10}$ ) and the acetylenic hydrocarbons can include acetylene( $\text{C}_2\text{H}_2$ ), methylacetylene( $\text{C}_3\text{H}_4$ ) and butene( $\text{C}_4\text{H}_6$ ).

The gaseous starting material comprising Si, C and H as the constituent atoms can include silicided alkyls, for example,  $\text{Si}(\text{CH}_3)_4$  and  $\text{Si}(\text{C}_2\text{H}_5)_4$ . In addition to these gaseous starting materials,  $\text{H}_2$  can of course be used as the gaseous starting material for introducing H.

In the case of forming the light receiving layer according to this invention by means of the glow discharging, sputtering or ion plating process, the content of the oxygen atoms, carbon atoms, nitrogen atoms and the group III or V atoms introduced into a-Si(H,X) is controlled by controlling the gas flow rate and the ratio of the gas flow rate of the starting materials entered in the deposition chamber.

The conditions upon forming the light receiving layer, for example, the temperature of the support, the gas pressure in the deposition chamber and the electric discharging power are important factors for obtaining a light receiving member having desired properties and they are properly selected while considering the function of the layer to be formed. Further, since these layer forming conditions may be varied depending on the kind and the amount of each of the atoms contained in the light receiving layer, the conditions have to be determined also taking the kind or the amount of the atoms to be contained into consideration.

Specifically, the temperature of the support is usually from 50° to 350° C. and, more preferably, from 50° to 250° C. The gas pressure in the deposition chamber is usually from 0.01 to 1 Torr and, particularly preferably, from 0.1 to 0.5 Torr. Further, the electrical discharging power is usually from 0.005 to 50 W/cm<sup>2</sup>, more prefera-

bly, from 0.01 to 30 W/cm<sup>2</sup> and, particularly preferably, from 0.01 to 20 W/cm<sup>2</sup>.

However, the actual conditions for forming the layer such as temperature of the support, discharging power and the gas pressure in the deposition chamber can not usually be determined with ease independent of each other. Accordingly, the conditions optimal to the layer formation are desirably determined based on relative and organic relationships for forming the amorphous material layer having desired properties.

By the way, it is necessary that the foregoing various conditions are kept constant upon forming the light receiving layer for unifying the distribution state of the oxygen atoms, carbon atoms, nitrogen atoms, group III or V atoms, or hydrogen atoms and/or halogen atoms to be contained in the light receiving layer according to this invention.

Further, in the case of forming a photosensitive layer comprising oxygen atoms, carbon atoms, nitrogen atoms, or group III or group V atoms contained in the light receiving layer at a desired distributed state in the direction of the layer thickness by varying their distribution densities in the direction of the layer thickness upon forming the light receiving layer in this invention, 20 the layer is formed, for example, in the case of the glow discharging process, by properly varying the gas flow rate of gaseous starting material for introducing the oxygen atoms, carbon atoms, nitrogen atoms, or group III or group V atoms upon introducing into the deposition chamber in accordance with a desired variation coefficient while maintaining other conditions constant. Then, the gas flow rate may be varied, specifically, by gradually changing the opening degree of a predetermined needle valve disposed to the midway of the gas flow system, for example, manually or any of other means usually employed such as an externally driving motor. In this case, the variation of the flow rate may not necessarily be linear but a desired content curve may be obtained, for example, by controlling the flow rate along with a previously designed variation coefficient curve by using a microcomputer or the like.

Further, in the case of forming the light receiving layer by means of the sputtering process, a desired distributed state of the oxygen atoms, carbon atoms, nitrogen atoms or group III or group V atoms in the direction of the layer thickness may be formed with the distribution density being varied in the direction of the layer thickness by using gaseous starting material for introducing the oxygen atoms, carbon atoms, nitrogen atoms, or group III or group V atoms and varying the gas flow rate upon introducing these gases into the deposition chamber in accordance with a desired variation coefficient in the same manner as the case of using the flow discharging process.

Further, in the case of constituting the surface layer in this invention with at least one of the elements selected from the inorganic fluorides, inorganic oxides and inorganic sulfides, since it is also necessary to control the layer thickness at an optical level for forming such a surface layer, vapor deposition, sputtering, gas phase plasma, optical CVD, heat CVD process or the like may be used. These forming processes are, of course, properly selected while considering those factors such as the kind of the forming materials for the surface layer, production conditions, installation cost required and production scale.

By the way, in view of the easy operations, easy setting for the conditions and the likes, sputtering pro-

cess may preferably be employed in the case of using the inorganic compounds for forming the surface layer. That is, the inorganic compound for forming the surface layer is used as a target and Ar gas is used as a sputtering gas, and the surface layer is deposited by causing glow discharging and sputtering the inorganic compounds.

#### PREFERRED EMBODIMENTS OF THE INVENTION

This invention will now be described more specifically while referring to examples 1 through 66 but this invention is in no way limited only to these examples.

In each of the examples, the photosensitive layer is formed by using the glow discharging process, while the surface layer is formed by using the glow discharging or sputtering process. FIG. 19 shows a device for preparing a light receiving member according to this invention by means of the glow discharging process.

Gas reservoirs 1092, 1093, 1094, 1095 and 1096 illustrated in the figure are charged with gaseous starting materials for forming the respective layers in this invention, that is, for instance, SiH<sub>4</sub> gas (99.999% purity) in the reservoir 1092, B<sub>2</sub>H<sub>6</sub> gas diluted with H<sub>2</sub> (99.999% purity, hereinafter simply referred to as B<sub>2</sub>H<sub>6</sub>/H<sub>2</sub>) in the reservoir 1093, CH<sub>4</sub> gas (99.999% purity) in the reservoir 1094, NH<sub>3</sub> gas (99.999% purity) in the reservoir 1095 and H<sub>2</sub> gas (99.999% purity) in the reservoir 1096.

Prior to the entrance of these gases into a reaction chamber 1901, it is confirmed that valves 1922-1926 for the gas reservoirs 1092-1096 and a leak valve 1935 are closed and that inlet valves 1912-1916, exit valves 1917-1921, and sub-valves 1932 and 1933 are opened. Then, a main valve 1934 is at first opened to evacuate the inside of the reaction chamber 1901 and gas pipe-ways. Then, when the reading on a vacuum gauge 1936 reaches about  $5 \times 10^{-6}$  Torr, the sub-valves 1932 and 1933, as well as the exit valves 1917-1921 are closed.

Reference is then made to an example in the case of forming a light receiving layer on a substrate cylinder 1937. SiH<sub>4</sub> gas from the gas reservoir 1092 and B<sub>2</sub>H<sub>6</sub>/H<sub>2</sub> gas from the gas reservoir 1093 are caused to flow into mass flow controllers 1907 and 1908 respectively by opening the valves 1922 and 1923, controlling the pressure of exit pressure gauges 1927 and 1928 to 1 kg/cm<sup>2</sup> and gradually opening the inlet valves 1912 and 1913. Subsequently, the exit valves 1917 and 1918 and the sub-valve 1932 are gradually opened to enter the gases into the reaction chamber 1901. In this case, the exit valves 1917 and 1918 are adjusted so as to attain a desired value for the ratio between the SiH<sub>4</sub> gas flow rate and the B<sub>2</sub>H<sub>6</sub>/H<sub>2</sub> gas flow rate, and the opening of the main valve 1934 is adjusted while observing the reading on the vacuum gauge 1936 so as to obtain a desired value for the pressure inside the reaction chamber 1901. Then, after confirming that the temperature of the substrate cylinder 1937 has been set by a heater 1938 within a range from 50° to 400° C., a power source 1940 is set to a predetermined electrical power to cause glow discharging in the reaction chamber 1901 while controlling the B<sub>2</sub>H<sub>6</sub>/H<sub>2</sub> gas flow rate and the SiH<sub>4</sub> gas flow rate in accordance with a previously designed variation coefficient curve by using a microcomputer (not illustrated), thereby forming, at first, a photosensitive layer constituted with a-Si(H,X) containing boron atoms on the substrate cylinder 1937.

Then, a surface layer is formed on the photosensitive layer. Subsequent to the procedures as described above, SiH<sub>4</sub> gas and CH<sub>4</sub> gas, for instance, are optionally di-

luted with a dilution gas such as He, Ar and H<sub>2</sub> respectively, entered at a desired gas flow rates into the reaction chamber 1901 while controlling the gas flow rate for the SiH<sub>4</sub> gas and the CH<sub>4</sub> gas in accordance with a previously designed variation coefficient curve by using a microcomputer (not illustrated), by which a surface layer constituted with a-Si(H,X) containing carbon atoms is formed.

When the photosensitive layer and the surface layer are formed, the flow rates for the gaseous starting materials are controlled by using the microcomputer or the like, in which the gas pressure in the reaction chamber 1901 can be stabilized to ensure a stable film-forming conditions by using a dilution gas together with the gaseous starting materials for introducing each of the atoms.

All of the exit valves other than those required for upon forming the respective layers are of course closed. Further, upon forming the respective layers, the inside of the system is once evacuated to a high vacuum degree as required by closing the exit valves 1917-1921 while opening the sub-valves 1932 and 1933 and fully opening the main valve 1934 for avoiding that the gases having been used for forming the previous layers are left in the reaction chamber 1901 and in the gas pipe-ways from the exit valves 1917-1921 to the inside of the reaction chamber 1901.

#### TEST EXAMPLE 1

Rigid spheres of 0.6 mm diameter made of SUS stainless steel were chemically etched to form an unevenness to the surface of each of the rigid spheres.

Usable as the etching agent are an acid such as hydrochloric acid, hydrofluoric acid, sulfuric acid and chromic acid and an alkali such as caustic soda.

In this example, an aqueous solution prepared by admixing 1.0 volumetric part of concentrated hydrochloric acid to 1.0 to 4.0 volumetric part of distilled water was used, and the period of time for the rigid spheres to be immersed in the aqueous solution, the acid concentration of the aqueous solution and other necessary conditions were appropriately adjusted to form a desired unevenness to the surface of each of the rigid spheres.

#### TEST EXAMPLE 2

In the device as shown in FIGS. 6(A) and 6(B), the surface of an aluminum alloy cylinder (diameter: 60 mm, length: 298 mm) was treated by using the rigid spheres each of which having a surface provided with appropriate minute irregularities (average height of the irregularities  $\gamma_{max}=5 \mu\text{m}$ ) which was obtained in Test Example 1 to have an appropriate uneven shape composed of dimples each of which having an inside face provided with irregularities.

When examining the relationship for the diameter R' of the rigid sphere, the falling height h, the radius of curvature R and the width D for the dimple, it was confirmed that the radius of curvature R and the width D of the dimple was determined depending on the conditions such as the diameter R' for the rigid sphere, the falling height h and the like. It was also confirmed that the pitch between each of the dimples (density of the dimples or the pitch for the unevenness) could be adjusted to a desired pitch by controlling the rotating speed or the rotation number of the cylinder, or the falling amount of the rigid sphere.

Further, the following matters were confirmed as a result of the studies about the magnitude of  $R$  and of  $D$ ; it is not preferred for  $R$  to be less than 0.1 mm because the rigid spheres to be employed in that case are to be lighter and smaller, that results in making it difficult to control the formation of the dimples as expected. Then, it is not preferred for  $R$  to be more than 2.0 mm because the rigid spheres to be employed in that case are to be heavier and the falling height is to be extremely lower, for instance, in the case where  $D$  is desired to be relatively smaller in order to adjust the falling height, that results in making it also difficult to control the formation of the dimples as expected. Further, it is not preferred for  $D$  to be less than 0.02 mm because the rigid spheres to be employed in that case are to be of a 15 smaller size and to be lighter in order to secure their falling height, that results in making it also difficult to control the formation of the dimples as expected. Further in addition, when examining the dimples as formed, it was confirmed that the inside face of each of the 20 dimples as formed was provided with appropriate min-

FIG. 20(A) is a schematic plan view illustrating the entire exposing device, and FIG. 20(B) is a schematic side elevational view for the entire device. In the figures, are shown a light receiving member 2001, a semiconductor laser 2002,  $f\theta$  lens 2003 and a polygonal mirror 2004.

Then, as a comparison, a light receiving member was manufactured in the same manner as described above by using an aluminum alloy cylinder, the surface of which 10 was treated with a conventional cutting tool (60 mm diameter, 298 mm length, 100  $\mu\text{m}$  unevenness pitch and 3  $\mu\text{m}$  unevenness depth) (cylinder No. 107). When observing the thus obtained light receiving member under an electron microscope, the layer interface between the support surface and the light receiving layer and the surface of the light receiving layer were in parallel with each other. Images were formed in the same manner as above by using this light receiving member and the thus obtained images were evaluated in the same manner as described above. The results are as shown in the lower column of Table 1A.

TABLE 1A

| Cylinder No.                      | 101          | 102          | 103          | 104          | 105          | 106          | 107 |
|-----------------------------------|--------------|--------------|--------------|--------------|--------------|--------------|-----|
| $D$ ( $\mu\text{m}$ )             | 450 $\pm$ 50 | 450 $\pm$ 50 | 450 $\pm$ 50 | 450 $\pm$ 50 | 450 $\pm$ 50 | 450 $\pm$ 50 | —   |
| $\frac{D}{R}$                     | 0.02         | 0.03         | 0.04         | 0.05         | 0.06         | 0.07         | —   |
| Occurrence of interference fringe | x            | Δ            | ○            | ○            | ◎            | ◎            | x   |

Actual usability:

x: not usable

Δ: usable

○: preferably usable

◎: particularly preferably usable

ute irregularities.

### EXAMPLE 1

The surface of an aluminum alloy cylinder was treated in the same manner as in the Test Example 2 to obtain a cylindrical Al support having diameter  $D$  and ratio  $D/R$  (cylinder Nos. 101-106) as shown in the upper column of Table 1A.

Then, a light receiving layer was formed on the Al support (cylinder Nos. 101-106) under the conditions shown in Table 1B below using the fabrication device shown in FIG. 19.

Boron atoms contained in the layer were so introduced to provide a ratio:  $\text{B}_2\text{H}_6/\text{SiF}_4 = 100$  ppm and that they were doped to about 200 ppm over the entire layer.

These light receiving members were subjected to imagewise exposure by irradiating laser beams at 780 nm wavelength and with 80  $\mu\text{m}$  of spot diameter using an image exposing device shown in FIG. 20 and images were obtained by subsequent development and transfer.

The state of the occurrence of interference fringe on the thus obtained images were as shown in the lower column of Table 1A.

TABLE 1B

| Layer preparing step | Gas used                          | Flow rate (SCCM)                        | Discharging power ( $\text{W}/\text{cm}^2$ ) | Layer thickness ( $\mu$ ) |
|----------------------|-----------------------------------|-----------------------------------------|----------------------------------------------|---------------------------|
| First step           | $\text{SiF}_4$                    | $\text{SiF}_4 = 300$                    | 300                                          | 2                         |
|                      | $\text{B}_2\text{H}_6/\text{H}_2$ | $\text{B}_2\text{H}_6/\text{H}_2 = 180$ |                                              |                           |
|                      | $\text{H}_2$                      | $\text{H}_2 = 120$                      |                                              |                           |
|                      | $\text{CH}_4$                     | $\text{CH}_4 = 5$                       |                                              |                           |
| Second step          | $\text{SiF}_4$                    | $\text{SiF}_4 = 300$                    | 300                                          | 23                        |
|                      | $\text{H}_2$                      | $\text{H}_2 = 300$                      |                                              |                           |
|                      | $\text{CH}_4$                     | $\text{CH}_4 = 5$                       |                                              |                           |

Al substrate temperature: 250°C.

Discharging frequency: 13.56 MHz

### EXAMPLE 2

A light receiving layer was formed on Al supports (cylinder Nos. 101-107) in the same manner as in Example 1 except for forming these light receiving layers in accordance with the layer forming conditions shown in Table 2B.

When forming the images on the thus obtained light receiving members in the same manner as in Example 1, the state of occurrence of the interference fringe in the obtained images were as shown in the lower column of Table 2A.

TABLE 2A

| Cylinder No.               | 101          | 102          | 103          | 104          | 105          | 106          | 107 |
|----------------------------|--------------|--------------|--------------|--------------|--------------|--------------|-----|
| $D$ ( $\mu\text{m}$ )      | 450 $\pm$ 50 | 450 $\pm$ 50 | 450 $\pm$ 50 | 450 $\pm$ 50 | 450 $\pm$ 50 | 450 $\pm$ 50 | —   |
| $\frac{D}{R}$              | 0.02         | 0.03         | 0.04         | 0.05         | 0.06         | 0.07         | —   |
| Occurrence of interference | x            | Δ            | ○            | ○            | ◎            | ◎            | x   |

TABLE 2A-continued

| Cylinder No. | 101 | 102 | 103 | 104 | 105 | 106 | 107 |
|--------------|-----|-----|-----|-----|-----|-----|-----|
| fringe       |     |     |     |     |     |     |     |

x: not usable

Δ: usable

○: preferably usable

◎: particularly preferably usable

TABLE 2B

| Layer preparing step | Gas used         | Flow rate (SCCM)       | Discharging power (W/cm <sup>2</sup> ) | Layer thickness (μm) |
|----------------------|------------------|------------------------|----------------------------------------|----------------------|
| First step           | SiF <sub>4</sub> | SiF <sub>4</sub> = 350 | 300                                    | 3                    |
|                      | NO               | NO = 10                |                                        |                      |
|                      | H <sub>2</sub>   | H <sub>2</sub> = 300   |                                        |                      |
| Second step          | SiF <sub>4</sub> | SiF <sub>4</sub> = 350 | 300                                    | 22                   |
|                      | H <sub>2</sub>   | H <sub>2</sub> = 300   |                                        |                      |

Al substrate temperature: 250° C.

Discharging frequency: 13.56 MHz

## EXAMPLES 3-7

Light receiving members were prepared on Al supports (cylinder Nos. 103-106) of Example 1 in the same manner as in Example 1 except for forming these light receiving layers in accordance with the layer forming conditions shown in Tables 3 through 7. In the examples 3 through 7, the flow rates for the gases used upon forming the light receiving layers were automatically adjusted under the microcomputer control in accordance with the flow rate variation curves shown in FIGS. 21-25 respectively. The boron atoms to be contained in the light receiving layers in each of the examples were introduced under the same conditions as those in Example 1.

Images were formed on the thus obtained light receiving members in the same manner as in Example 1.

Occurrence of interference fringe was not observed in any of the thus obtained images and the image quality was extremely high.

TABLE 3

| (Variation chart: FIG. 21) |                                               |                                                     |                                        |                      |
|----------------------------|-----------------------------------------------|-----------------------------------------------------|----------------------------------------|----------------------|
| Layer preparing step       | Gas used                                      | Flow rate (SCCM)                                    | Discharging power (W/cm <sup>2</sup> ) | Layer thickness (μm) |
| First step                 | SiF <sub>4</sub>                              | SiF <sub>4</sub> = 350                              | 300                                    | 2                    |
|                            | H <sub>2</sub>                                | H <sub>2</sub> = 120                                |                                        |                      |
|                            | NH <sub>3</sub>                               | NH <sub>3</sub> = 10                                |                                        |                      |
| Second step                | B <sub>2</sub> H <sub>6</sub> /H <sub>2</sub> | B <sub>2</sub> H <sub>6</sub> /H <sub>2</sub> = 180 |                                        |                      |
|                            | SiF <sub>4</sub>                              | SiF <sub>4</sub> = 350                              | 300                                    | 2                    |
|                            | H <sub>2</sub>                                | H <sub>2</sub> = 120                                |                                        |                      |
| Third step                 | NH <sub>3</sub>                               | NH <sub>3</sub> = 10 → 0.5                          |                                        |                      |
|                            | B <sub>2</sub> H <sub>6</sub> /H <sub>2</sub> | B <sub>2</sub> H <sub>6</sub> /H <sub>2</sub> = 180 |                                        |                      |
|                            | SiF <sub>4</sub>                              | SiF <sub>4</sub> = 350                              | 300                                    | 17                   |
| Fourth step                | H <sub>2</sub>                                | H <sub>2</sub> = 300                                |                                        |                      |
|                            | NH <sub>3</sub>                               | NH <sub>3</sub> = 0.5                               |                                        |                      |
|                            | SiF <sub>4</sub>                              | SiF <sub>4</sub> = 350                              | 300                                    | 2                    |
| Fifth step                 | H <sub>2</sub>                                | H <sub>2</sub> = 300                                |                                        |                      |
|                            | NH <sub>3</sub>                               | NH <sub>3</sub> = 0.5 → 10                          |                                        |                      |
|                            | SiF <sub>4</sub>                              | SiF <sub>4</sub> = 350                              | 300                                    | 2                    |
| Sixth step                 | H <sub>2</sub>                                | H <sub>2</sub> = 300                                |                                        |                      |
|                            | NH <sub>3</sub>                               | NH <sub>3</sub> = 10                                |                                        |                      |

Al substrate temperature: 250° C.

Discharging frequency: 13.56 MHz

TABLE 4

(Variation chart: FIG. 22)

| Layer preparing step | Gas used                                      | Flow rate (SCCM)                                        | Discharging power (W/cm <sup>2</sup> ) | Layer thickness (μm) |
|----------------------|-----------------------------------------------|---------------------------------------------------------|----------------------------------------|----------------------|
| First step           | SiF <sub>4</sub>                              | SiF <sub>4</sub> = 350                                  | 300                                    | 3                    |
|                      | H <sub>2</sub>                                | H <sub>2</sub> = 120                                    |                                        |                      |
|                      | NO                                            | NO = 5                                                  |                                        |                      |
| Second step          | B <sub>2</sub> H <sub>6</sub> /H <sub>2</sub> | B <sub>2</sub> H <sub>6</sub> /H <sub>2</sub> = 180     |                                        |                      |
|                      | SiF <sub>4</sub>                              | SiF <sub>4</sub> = 350                                  | 300                                    | 1                    |
|                      | H <sub>2</sub>                                | H <sub>2</sub> = 120 → 300                              |                                        |                      |
| Third step           | NO                                            | NO = 5                                                  |                                        |                      |
|                      | B <sub>2</sub> H <sub>6</sub> /H <sub>2</sub> | B <sub>2</sub> H <sub>6</sub> /H <sub>2</sub> = 180 → 0 |                                        |                      |
|                      | SiF <sub>4</sub>                              | SiF <sub>4</sub> = 350                                  | 300                                    | 21                   |
| Fourth step          | H <sub>2</sub>                                | H <sub>2</sub> = 300                                    |                                        |                      |
|                      | NO                                            | NO = 5                                                  |                                        |                      |

Al substrate temperature: 250° C.

Discharging frequency: 13.56 MHz

TABLE 5

(Variation chart: FIG. 23)

| Layer preparing step | Gas used                                      | Flow rate (SCCM)                                        | Discharging power (W/cm <sup>2</sup> ) | Layer thickness (μm) |
|----------------------|-----------------------------------------------|---------------------------------------------------------|----------------------------------------|----------------------|
| First step           | SiH <sub>4</sub>                              | SiH <sub>4</sub> = 350                                  | 300                                    | 5                    |
|                      | H <sub>2</sub>                                | H <sub>2</sub> = 0 → 300                                |                                        |                      |
|                      | B <sub>2</sub> H <sub>6</sub> /H <sub>2</sub> | B <sub>2</sub> H <sub>6</sub> /H <sub>2</sub> = 300 → 0 |                                        |                      |
| Second step          | CH <sub>4</sub>                               | CH <sub>4</sub> = 10 → 0                                |                                        |                      |
|                      | SiH <sub>4</sub>                              | SiH <sub>4</sub> = 350                                  | 300                                    | 20                   |
| Third step           | H <sub>2</sub>                                | H <sub>2</sub> = 300                                    |                                        |                      |

Al substrate temperature: 250° C.

Discharging frequency: 13.56 MHz

TABLE 6

(Variation chart: FIG. 24)

| Layer preparing step | Gas used                                      | Flow rate (SCCM)                                        | Discharging power (W/cm <sup>2</sup> ) | Layer thickness (μm) |
|----------------------|-----------------------------------------------|---------------------------------------------------------|----------------------------------------|----------------------|
| First step           | SiF <sub>4</sub>                              | SiF <sub>4</sub> = 300                                  | 300                                    | 2                    |
|                      | H <sub>2</sub>                                | H <sub>2</sub> = 120                                    |                                        |                      |
|                      | B <sub>2</sub> H <sub>6</sub> /H <sub>2</sub> | B <sub>2</sub> H <sub>6</sub> /H <sub>2</sub> = 180     |                                        |                      |
| Second step          | NH <sub>3</sub>                               | NH <sub>3</sub> = 10                                    |                                        |                      |
|                      | SiF <sub>4</sub>                              | SiF <sub>4</sub> = 300                                  | 300                                    | 2                    |
|                      | H <sub>2</sub>                                | H <sub>2</sub> = 120 → 300                              |                                        |                      |
| Third step           | B <sub>2</sub> H <sub>6</sub> /H <sub>2</sub> | B <sub>2</sub> H <sub>6</sub> /H <sub>2</sub> = 180 → 0 |                                        |                      |
|                      | NH <sub>3</sub>                               | NH <sub>3</sub> = 10 → 0.5                              |                                        |                      |
|                      | SiF <sub>4</sub>                              | SiF <sub>4</sub> = 300                                  | 300                                    | 21                   |
| Fourth step          | H <sub>2</sub>                                | H <sub>2</sub> = 300                                    |                                        |                      |
|                      | NH <sub>3</sub>                               | NH <sub>3</sub> = 0.5                                   |                                        |                      |

Al substrate temperature: 250° C.

Discharging frequency: 13.56 MHz

TABLE 7

(Variation chart: FIG. 25)

| Layer preparing step | Gas used                                      | Flow rate (SCCM)                                    | Discharging power (W/cm <sup>2</sup> ) | Layer thickness (μm) |
|----------------------|-----------------------------------------------|-----------------------------------------------------|----------------------------------------|----------------------|
| First step           | SiH <sub>4</sub>                              | SiH <sub>4</sub> = 300                              | 300                                    | 1                    |
|                      | H <sub>2</sub>                                | H <sub>2</sub> = 300                                |                                        |                      |
|                      | B <sub>2</sub> H <sub>6</sub> /H <sub>2</sub> | B <sub>2</sub> H <sub>6</sub> /H <sub>2</sub> = 200 |                                        |                      |
| Second step          | NO                                            | NO = 10                                             |                                        |                      |

TABLE 7-continued

(Variation chart: FIG. 25)

| Layer preparing step | Gas used                                      | Flow rate (SCCM)                                        | Discharging power (W/cm <sup>2</sup> ) | Layer thickness (μm) |
|----------------------|-----------------------------------------------|---------------------------------------------------------|----------------------------------------|----------------------|
| Second step          | SiH <sub>4</sub>                              | SiH <sub>4</sub> = 300                                  | 300                                    | 2                    |
|                      | H <sub>2</sub>                                | H <sub>2</sub> = 300                                    |                                        |                      |
|                      | B <sub>2</sub> H <sub>6</sub> /H <sub>2</sub> | B <sub>2</sub> H <sub>6</sub> /H <sub>2</sub> = 200 → 0 |                                        |                      |

H<sub>2</sub> gas upon forming the light receiving layers were automatically adjusted under the microcomputer control in accordance with the flow rate variation curves shown in FIGS. 22-23 and 25 respectively.

5 Images were formed on the thus obtained light receiving members in the same manner as in Example 1.

Occurrence of interference fringe was not observed in any of the thus obtained images and the image quality was extremely high.

TABLE 8

| Layer constitution    | Layer preparing step | Gas used                                                                         | Flow rate (SCCM)                                                              | Discharging power (W) | Layer thickness (μm) |
|-----------------------|----------------------|----------------------------------------------------------------------------------|-------------------------------------------------------------------------------|-----------------------|----------------------|
| Photo-sensitive layer | First step           | SiF <sub>4</sub><br>B <sub>2</sub> H <sub>6</sub> /H <sub>2</sub><br>(=3000 ppm) | SiF <sub>4</sub> = 350<br>B <sub>2</sub> H <sub>6</sub> /H <sub>2</sub> = 180 | 300                   | 2                    |
| Photo-sensitive layer | Second step          | SiF <sub>4</sub><br>H <sub>2</sub>                                               | SiF <sub>4</sub> = 350<br>H <sub>2</sub> = 300                                | 300                   | 23                   |
| Surface layer         | Third step           | SiF <sub>4</sub><br>NO                                                           | SiF <sub>4</sub> = 100<br>NO = 500                                            | 200                   | 0.5                  |

Al substrate temperature: 250° C.  
Discharging frequency: 13.56 MHz

TABLE 9

| Layer constitution    | Layer preparing step | Gas used                                                           | Flow rate (SCCM)                                                | Discharging power (W) | Layer thickness (μm) |
|-----------------------|----------------------|--------------------------------------------------------------------|-----------------------------------------------------------------|-----------------------|----------------------|
| Photo-sensitive layer | First step           | SiF <sub>4</sub><br>PH <sub>3</sub> /H <sub>2</sub><br>(=3000 ppm) | SiF <sub>4</sub> = 300<br>PH <sub>3</sub> /H <sub>2</sub> = 180 | 300                   | 2                    |
| Photo-sensitive layer | Second step          | SiF <sub>4</sub><br>H <sub>2</sub>                                 | SiF <sub>4</sub> = 300<br>H <sub>2</sub> = 300                  | 300                   | 23                   |
| Surface layer         | Third step           | SiF <sub>4</sub><br>NO                                             | SiF <sub>4</sub> = 100<br>NO = 500                              | 200                   | 0.5                  |

Al substrate temperature: 250° C.  
Discharging frequency: 13.56 MHz

|            |                                          |                                                           |     |    |
|------------|------------------------------------------|-----------------------------------------------------------|-----|----|
| Third step | NO<br>SiH <sub>4</sub><br>H <sub>2</sub> | NO = 10<br>SiH <sub>4</sub> = 400<br>H <sub>2</sub> = 300 | 300 | 22 |
|------------|------------------------------------------|-----------------------------------------------------------|-----|----|

Al substrate temperature: 250° C.  
Discharging frequency: 13.56 MHz

## EXAMPLES 8-13

Light receiving members were prepared on Al supports (cylinder Nos. 103-106) of Example 1 in the same manner as in Example 1 except for forming these light receiving layers in accordance with the layer forming conditions shown in Tables 8 through 13. In the examples 11 through 13, the flow rates of B<sub>2</sub>H<sub>6</sub>/H<sub>2</sub> gas and

TABLE 10

| Layer constitution    | Layer preparing step | Gas used                           | Flow rate (SCCM)                               | Discharging power (W) | Layer thickness (μm) |
|-----------------------|----------------------|------------------------------------|------------------------------------------------|-----------------------|----------------------|
| Photo-sensitive layer | First step           | SiF <sub>4</sub><br>H <sub>2</sub> | SiF <sub>4</sub> = 350<br>H <sub>2</sub> = 300 | 300                   | 25                   |
| Surface layer         | Second step          | SiF <sub>4</sub><br>NO             | SiF <sub>4</sub> = 100<br>NO = 500             | 200                   | 0.5                  |

50 Al substrate temperature: 250° C.  
Discharging frequency: 13.56 MHz

TABLE 11

| Layer constitution    | Layer preparing step | Gas used                                                                         | Flow rate (SCCM)                                                                  | Discharging power (W) | Layer thickness (μm) |
|-----------------------|----------------------|----------------------------------------------------------------------------------|-----------------------------------------------------------------------------------|-----------------------|----------------------|
| Photo-sensitive layer | First step           | SiF <sub>4</sub><br>B <sub>2</sub> H <sub>6</sub> /H <sub>2</sub><br>(=3000 ppm) | SiF <sub>4</sub> = 300<br>B <sub>2</sub> H <sub>6</sub> /H <sub>2</sub> = 180     | 300                   | 3                    |
| Photo-sensitive layer | Second step          | SiF <sub>4</sub><br>B <sub>2</sub> H <sub>6</sub> /H <sub>2</sub><br>(=3000 ppm) | SiF <sub>4</sub> = 300<br>B <sub>2</sub> H <sub>6</sub> /H <sub>2</sub> = 180 → 0 | 300                   | 1                    |
| Photo-sensitive layer | Third step           | SiF <sub>4</sub><br>H <sub>2</sub>                                               | H <sub>2</sub> = 120 → 300                                                        | 300                   | 21                   |
| Surface               | Fourth               | SiF <sub>4</sub>                                                                 | SiF <sub>4</sub> = 100                                                            | 200                   | 0.5                  |

TABLE 11-continued

| Layer constitution |      | Layer preparing step |    | Flow rate (SCCM) | Discharging power (W) | Layer thickness (μm) |
|--------------------|------|----------------------|----|------------------|-----------------------|----------------------|
| layer              | step | Gas used             | NO | NO = 500         |                       |                      |

Al substrate temperature: 250° C.

Discharging frequency: 13.56 MHz

TABLE 12

| Layer constitution    |             | Layer preparing step |                                                                                  | Flow rate (SCCM)                                                                                              | Discharging power (W) | Layer thickness (μm) |
|-----------------------|-------------|----------------------|----------------------------------------------------------------------------------|---------------------------------------------------------------------------------------------------------------|-----------------------|----------------------|
| Photo-sensitive layer | step        | Gas used             | SiF <sub>4</sub><br>B <sub>2</sub> H <sub>6</sub> /H <sub>2</sub><br>(=3000 ppm) | SiF <sub>4</sub> = 300<br>B <sub>2</sub> H <sub>6</sub> /H <sub>2</sub> = 300 → 0<br>H <sub>2</sub> = 0 → 300 | 300                   | 5                    |
|                       | Second step | SiF <sub>4</sub>     | SiF <sub>4</sub> = 300<br>H <sub>2</sub> = 300                                   | 300                                                                                                           | 20                    |                      |
| Surface layer         | Third step  | SiF <sub>4</sub>     | SiF <sub>4</sub> = 100<br>NO = 500                                               | 200                                                                                                           | 0.5                   |                      |

Al substrate temperature: 250° C.

Discharging frequency: 13.56 MHz

TABLE 13

| Layer constitution    |             | Layer preparing step |                                                                                  | Flow rate (SCCM)                                                                                        | Discharging power (W) | Layer thickness (μm) |
|-----------------------|-------------|----------------------|----------------------------------------------------------------------------------|---------------------------------------------------------------------------------------------------------|-----------------------|----------------------|
| Photo-sensitive layer | step        | Gas used             | SiH <sub>4</sub><br>B <sub>2</sub> H <sub>6</sub> /H <sub>2</sub><br>(=3000 ppm) | SiH <sub>4</sub> = 300<br>B <sub>2</sub> H <sub>6</sub> /H <sub>2</sub> = 200 0<br>H <sub>2</sub> = 300 | 300                   | 3                    |
|                       | Second step | SiH <sub>4</sub>     | SiH <sub>4</sub> = 300<br>H <sub>2</sub> = 300                                   | 300                                                                                                     | 22                    |                      |
| Surface layer         | Third step  | SiH <sub>4</sub>     | SiH <sub>4</sub> = 100<br>NO = 500                                               | 200                                                                                                     | 0.5                   |                      |

Al substrate temperature: 250° C.

Discharging frequency: 13.56 MHz

## EXAMPLES 14-25

40

TABLE 14-continued

Light receiving members were prepared on Al supports (cylinder Nos. 103-106) of Example 1 in the same manner as in Example 1 except for forming these light receiving layers in accordance with the layer forming conditions shown in Tables 14 through 25.

In the examples 16-19 and 21-24, the flow rates for the gas used upon forming the light receiving layers were automatically adjusted under the microcomputer control in accordance with the flow rate variation curves shown in FIGS. 26, 22, 27, 24, 25, 28, 29 and 30 respectively.

The boron atoms to be contained in the light receiving layers were introduced under the same conditions as those in Example 1.

Images were formed on the thus obtained light receiving members in the same manner as in Example 1.

Occurrence of interference fringe was not observed in any of the thus obtained images and the image quality was extremely high.

TABLE 14

| Layer constitution | Layer preparing step | Gas used                            | Flow rate (SCCM)                              | Discharging power (W) | Layer thickness (μm) |
|--------------------|----------------------|-------------------------------------|-----------------------------------------------|-----------------------|----------------------|
| Photo-sensitive    | First step           | SiF <sub>4</sub><br>CH <sub>4</sub> | SiF <sub>4</sub> = 350<br>CH <sub>4</sub> = 5 | 300                   | 3                    |

45

55

TABLE 15

| Layer constitution    | Layer preparing step | Gas used                            | Flow rate (SCCM)                               | Discharging power (W) | Layer thickness (μm) |
|-----------------------|----------------------|-------------------------------------|------------------------------------------------|-----------------------|----------------------|
| photo-sensitive layer | Second step          | SiF <sub>4</sub><br>CH <sub>4</sub> | SiF <sub>4</sub> = 350<br>CH <sub>4</sub> = 5  | 300                   | 22                   |
| Surface layer         | Third step           | SiF <sub>4</sub><br>NH <sub>3</sub> | SiF <sub>4</sub> = 20<br>NH <sub>3</sub> = 600 | 200                   | 0.5                  |

Al substrate temperature: 250° C.

Discharging frequency: 13.56 MHz

60

65

| Layer constitution    | Layer preparing step | Gas used                           | Flow rate (SCCM)                               | Discharging power (W) | Layer thickness (μm) |
|-----------------------|----------------------|------------------------------------|------------------------------------------------|-----------------------|----------------------|
| photo-sensitive layer | First step           | SiF <sub>4</sub><br>H <sub>2</sub> | SiF <sub>4</sub> = 350<br>H <sub>2</sub> = 300 | 300                   | 3                    |
| Surface layer         | Second step          | SiF <sub>4</sub><br>H <sub>2</sub> | SiF <sub>4</sub> = 350<br>H <sub>2</sub> = 300 | 300                   | 22                   |

Al substrate temperature: 250° C.

Discharging frequency: 13.56 MHz

TABLE 16

(Variation Chart: FIG. 26)

| Layer constitution    | Layer preparing step | Gas used                                      | Flow rate (SCCM)                                    | Discharging power (W) | Layer thickness ( $\mu$ m) |
|-----------------------|----------------------|-----------------------------------------------|-----------------------------------------------------|-----------------------|----------------------------|
| Photo-sensitive layer | First step           | SiF <sub>4</sub>                              | SiF <sub>4</sub> = 350                              | 300                   | 2                          |
|                       |                      | H <sub>2</sub>                                | H <sub>2</sub> = 120                                |                       |                            |
|                       |                      | CH <sub>4</sub>                               | CH <sub>4</sub> = 10                                |                       |                            |
|                       |                      | B <sub>2</sub> H <sub>6</sub> /H <sub>2</sub> | B <sub>2</sub> H <sub>6</sub> /H <sub>2</sub> = 180 |                       |                            |
|                       | Second step          | SiF <sub>4</sub>                              | SiF <sub>4</sub> = 350                              | 300                   | 2                          |
|                       |                      | H <sub>2</sub>                                | H <sub>2</sub> = 120                                |                       |                            |
|                       |                      | CH <sub>4</sub>                               | CH <sub>4</sub> = 10 → 0.5                          |                       |                            |
|                       |                      | B <sub>2</sub> H <sub>6</sub> /H <sub>2</sub> | B <sub>2</sub> H <sub>6</sub> /H <sub>2</sub> = 180 |                       |                            |
|                       | Third step           | SiF <sub>4</sub>                              | SiF <sub>4</sub> = 350                              | 300                   | 17                         |
|                       |                      | H <sub>2</sub>                                | H <sub>2</sub> = 300                                |                       |                            |
|                       |                      | CH <sub>4</sub>                               | CH <sub>4</sub> = 0.5                               |                       |                            |
|                       | Fourth step          | SiF <sub>4</sub>                              | SiF <sub>4</sub> = 350                              | 300                   | 2                          |
|                       |                      | H <sub>2</sub>                                | H <sub>2</sub> = 300                                |                       |                            |
|                       |                      | CH <sub>4</sub>                               | CH <sub>4</sub> = 0.5 → 10                          |                       |                            |
|                       | Fifth step           | SiF <sub>4</sub>                              | SiF <sub>4</sub> = 350                              | 300                   | 2                          |
|                       |                      | H <sub>2</sub>                                | H <sub>2</sub> = 300                                |                       |                            |
|                       |                      | CH <sub>4</sub>                               | CH <sub>4</sub> = 10                                |                       |                            |
| Surface layer         | Sixth step           | SiF <sub>4</sub>                              | SiF <sub>4</sub> = 100                              | 200                   | 0.5                        |
|                       |                      | NO                                            | NO = 500                                            |                       |                            |

Al substrate temperature: 250° C.

Discharging frequency: 13.56 MHz

TABLE 17

(Variation chart: FIG. 22)

| Layer constitution    | Layer preparing step | Gas used                                      | Flow rate (SCCM)                                        | Discharging power (W) | Layer thickness ( $\mu$ ) |
|-----------------------|----------------------|-----------------------------------------------|---------------------------------------------------------|-----------------------|---------------------------|
| Photo-sensitive layer | First step           | SiF <sub>4</sub>                              | SiF <sub>4</sub> = 350                                  | 300                   | 3                         |
|                       |                      | H <sub>2</sub>                                | H <sub>2</sub> = 120                                    |                       |                           |
|                       |                      | NH <sub>3</sub>                               | NH <sub>3</sub> = 5                                     |                       |                           |
|                       |                      | B <sub>2</sub> H <sub>6</sub> /H <sub>2</sub> | B <sub>2</sub> H <sub>6</sub> /H <sub>2</sub> = 180     |                       |                           |
|                       | Second step          | SiF <sub>4</sub>                              | SiF <sub>4</sub> = 350                                  | 300                   | 1                         |
|                       |                      | H <sub>2</sub>                                | H <sub>2</sub> = 120 → 300                              |                       |                           |
|                       |                      | NH <sub>3</sub>                               | NH <sub>3</sub> = 5                                     |                       |                           |
|                       |                      | B <sub>2</sub> H <sub>6</sub> /H <sub>2</sub> | B <sub>2</sub> H <sub>6</sub> /H <sub>2</sub> = 180 → 0 |                       |                           |
|                       | Third step           | SiF <sub>4</sub>                              | SiF <sub>4</sub> = 350                                  | 300                   | 21                        |
|                       |                      | H <sub>2</sub>                                | H <sub>2</sub> = 300                                    |                       |                           |
|                       |                      | NH <sub>3</sub>                               | NH <sub>3</sub> = 5                                     |                       |                           |
| Surface layer         | Fourth step          | SiF <sub>4</sub>                              | SiF <sub>4</sub> = 10                                   | 200                   | 0.5                       |
|                       |                      | CH <sub>4</sub>                               | CH <sub>4</sub> = 600                                   |                       |                           |

Al substrate temperature: 250° C.

Discharging frequency: 13.56 MHz

TABLE 18

(Variation chart: FIG. 27)

| Layer constitution    | Layer preparing step | Gas used                                      | Flow rate (SCCM)                                        | Discharging power (W) | Layer thickness ( $\mu$ ) |
|-----------------------|----------------------|-----------------------------------------------|---------------------------------------------------------|-----------------------|---------------------------|
| Photo-sensitive layer | First step           | SiF <sub>4</sub>                              | SiF <sub>4</sub> = 350                                  | 300                   | 5                         |
|                       |                      | H <sub>2</sub>                                | H <sub>2</sub> = 0 → 300                                |                       |                           |
|                       |                      | B <sub>2</sub> H <sub>6</sub> /H <sub>2</sub> | B <sub>2</sub> H <sub>6</sub> /H <sub>2</sub> = 300 → 0 |                       |                           |
|                       |                      | NH <sub>3</sub>                               | NH <sub>3</sub> = 10 → 0                                |                       |                           |
|                       | Second step          | SiF <sub>4</sub>                              | SiF <sub>4</sub> = 350                                  | 300                   | 20                        |
|                       |                      | H <sub>2</sub>                                | H <sub>2</sub> = 300                                    |                       |                           |
|                       |                      | NH <sub>3</sub>                               | NH <sub>3</sub> = 10                                    |                       |                           |
|                       | Surface layer        | Third step                                    | SiF <sub>4</sub>                                        | SiF <sub>4</sub> = 10 | 200                       |
|                       |                      | CH <sub>4</sub>                               | CH <sub>4</sub> = 600                                   |                       | 0.5                       |

Al substrate temperature: 250° C.

Discharging frequency: 13.56 MHz

TABLE 19

(Variation chart: FIG. 24)

| Layer constitution    | Layer preparing step | Gas used                                      | Flow rate (SCCM)                                    | Discharging power (W) | Layer thickness ( $\mu$ ) |
|-----------------------|----------------------|-----------------------------------------------|-----------------------------------------------------|-----------------------|---------------------------|
| Photo-sensitive layer | First step           | SiF <sub>4</sub>                              | SiF <sub>4</sub> = 350                              | 300                   | 2                         |
|                       |                      | H <sub>2</sub>                                | H <sub>2</sub> = 120                                |                       |                           |
|                       |                      | B <sub>2</sub> H <sub>6</sub> /H <sub>2</sub> | B <sub>2</sub> H <sub>6</sub> /H <sub>2</sub> = 180 |                       |                           |
|                       |                      | NH <sub>3</sub>                               | NH <sub>3</sub> = 10                                |                       |                           |
|                       | Second step          | SiF <sub>4</sub>                              | SiF <sub>4</sub> = 350                              | 300                   | 2                         |
|                       |                      | H <sub>2</sub>                                | H <sub>2</sub> = 120 → 300                          |                       |                           |

TABLE 19-continued

| (Variation chart: FIG. 24) |                                               |                                                         |                  |                       |                           |
|----------------------------|-----------------------------------------------|---------------------------------------------------------|------------------|-----------------------|---------------------------|
| Layer constitution         | Layer preparing step                          | Gas used                                                | Flow rate (SCCM) | Discharging power (W) | Layer thickness ( $\mu$ ) |
| Third step                 | B <sub>2</sub> H <sub>5</sub> /H <sub>2</sub> | B <sub>2</sub> H <sub>6</sub> /H <sub>2</sub> = 180 → 0 |                  |                       |                           |
|                            | NH <sub>3</sub>                               | NH <sub>3</sub> = 10 → 0.5                              |                  |                       |                           |
|                            | SiF <sub>4</sub>                              | SiF <sub>4</sub> = 350                                  | 300              | 21                    |                           |
|                            | H <sub>2</sub>                                | H <sub>2</sub> = 300                                    |                  |                       |                           |
| Surface layer              | NH <sub>3</sub>                               | NH <sub>3</sub> = 0.5                                   |                  |                       |                           |
|                            | SiF <sub>4</sub>                              | SiF <sub>4</sub> = 10                                   | 200              | 0.5                   |                           |
|                            | CH <sub>4</sub>                               | CH <sub>4</sub> = 600                                   |                  |                       |                           |

Al substrate temperature: 250° C.

Discharging frequency: 13.56 MHz

TABLE 20

| Layer constitution    | Layer preparing step | Gas used                                      | Flow rate (SCCM)                                    | Discharging power (W) | Layer thickness ( $\mu$ ) |
|-----------------------|----------------------|-----------------------------------------------|-----------------------------------------------------|-----------------------|---------------------------|
| Photo-sensitive layer | First step           | SiF <sub>4</sub>                              | SiF <sub>4</sub> = 350                              | 300                   | 5                         |
|                       |                      | H <sub>2</sub>                                | H <sub>2</sub> = 120                                |                       |                           |
|                       |                      | B <sub>2</sub> H <sub>6</sub> /H <sub>2</sub> | B <sub>2</sub> H <sub>6</sub> /H <sub>2</sub> = 180 | 300                   | 22                        |
|                       |                      | NO                                            | NO = 5                                              |                       |                           |
| surface layer         | Second step          | SiF <sub>4</sub>                              | SiF <sub>4</sub> = 350                              | 300                   | 22                        |
|                       |                      | H <sub>2</sub>                                | H <sub>2</sub> = 300                                |                       |                           |
|                       |                      | NO                                            | NO = 5                                              |                       |                           |
| Third step            | SiF <sub>4</sub>     | SiF <sub>4</sub> = 10                         | 200                                                 | 0.5                   | 0.5                       |
|                       | CH <sub>4</sub>      | CH <sub>4</sub> = 600                         |                                                     |                       |                           |

Al substrate temperature: 250° C.

Discharging frequency: 13.56 MHz

TABLE 22

| (Variation chart: FIG. 28) |                      |                                               |                                                     |                       |                           |
|----------------------------|----------------------|-----------------------------------------------|-----------------------------------------------------|-----------------------|---------------------------|
| Layer constitution         | Layer preparing step | Gas used                                      | Flow rate (SCCM)                                    | Discharging power (W) | Layer thickness ( $\mu$ ) |
| Photo-sensitive layer      | First step           | SiH <sub>4</sub>                              | SiH <sub>4</sub> = 350                              | 300                   | 4                         |
|                            |                      | B <sub>2</sub> H <sub>6</sub> /H <sub>2</sub> | B <sub>2</sub> H <sub>6</sub> /H <sub>2</sub> = 200 |                       |                           |
| Second step                | SiH <sub>4</sub>     | SiH <sub>4</sub> = 350                        | 300                                                 | 21                    | 21                        |
|                            |                      | NO                                            | NO = 0.5                                            |                       |                           |
| Surface layer              | Third step           | SiF <sub>4</sub>                              | SiF <sub>4</sub> = 10                               | 200                   | 0.5                       |
|                            |                      | CH <sub>4</sub>                               | CH <sub>4</sub> = 600                               |                       |                           |

Al substrate temperature: 250° C.

Discharging frequency: 13.56 MHz

TABLE 21

| (Variation chart: FIG. 25) |                      |                                               |                                                         |                       |                           |
|----------------------------|----------------------|-----------------------------------------------|---------------------------------------------------------|-----------------------|---------------------------|
| Layer constitution         | Layer preparing step | Gas used                                      | Flow rate (SCCM)                                        | Discharging power (W) | Layer thickness ( $\mu$ ) |
| Photo-sensitive layer      | First step           | SiH <sub>4</sub>                              | SiH <sub>4</sub> = 350                                  | 300                   | 1                         |
|                            |                      | H <sub>2</sub>                                | H <sub>2</sub> = 300                                    |                       |                           |
|                            |                      | B <sub>2</sub> H <sub>6</sub> /H <sub>2</sub> | B <sub>2</sub> H <sub>6</sub> /H <sub>2</sub> = 200     | 300                   | 4                         |
|                            |                      | NO                                            | NO-10                                                   |                       |                           |
| Second step                | SiH <sub>4</sub>     | SiH <sub>4</sub> = 350                        | 300                                                     | 20                    | 20                        |
|                            |                      | H <sub>2</sub>                                | H <sub>2</sub> = 300                                    |                       |                           |
|                            |                      | B <sub>2</sub> H <sub>6</sub> /H <sub>2</sub> | B <sub>2</sub> H <sub>6</sub> /H <sub>2</sub> = 200 → 0 |                       |                           |
| Third step                 | SiH <sub>4</sub>     | SiH <sub>4</sub> = 350                        | 300                                                     | 20                    | 20                        |
|                            |                      | H <sub>2</sub>                                | H <sub>2</sub> = 300                                    |                       |                           |
|                            |                      | NO                                            | NO = 10 → 0                                             |                       |                           |
| Surface layer              | Fourth step          | SiF <sub>4</sub>                              | SiF <sub>4</sub> = 10                                   | 200                   | 0.5                       |
|                            |                      | CH <sub>4</sub>                               | CH <sub>4</sub> = 600                                   |                       |                           |

Al substrate temperature: 250° C.

Discharging frequency: 13.56 MHz

TABLE 23

| (Variation chart: FIG. 29) |                      |                                               |                                                         |                       |                           |
|----------------------------|----------------------|-----------------------------------------------|---------------------------------------------------------|-----------------------|---------------------------|
| Layer constitution         | Layer preparing step | Gas used                                      | Flow rate (SCCM)                                        | Discharging power (W) | Layer thickness ( $\mu$ ) |
| photo-sensitive layer      | First step           | SiH <sub>4</sub>                              | SiH <sub>4</sub> = 350                                  | 300                   | 3                         |
|                            |                      | H <sub>2</sub>                                | H <sub>2</sub> = 300                                    |                       |                           |
|                            |                      | B <sub>2</sub> H <sub>6</sub> /H <sub>2</sub> | B <sub>2</sub> H <sub>6</sub> /H <sub>2</sub> = 250 → 0 |                       |                           |
|                            |                      | CH <sub>4</sub>                               | CH <sub>4</sub> = 10                                    |                       |                           |
| Surface layer              | Second step          | SiH <sub>4</sub>                              | SiH <sub>4</sub> = 350                                  | 300                   | 22                        |
|                            |                      | H <sub>2</sub>                                | H <sub>2</sub> = 300                                    |                       |                           |
|                            |                      | NO                                            | NO = 500                                                |                       |                           |
| Third step                 | SiF <sub>4</sub>     | SiF <sub>4</sub> = 100                        | 200                                                     | 0.5                   | 0.5                       |
|                            |                      | CH <sub>4</sub>                               |                                                         |                       |                           |

Al substrate temperature: 250° C.

Discharging frequency: 13.56 MHz

TABLE 24

| (Variation chart: FIG. 30) |                      |                                               |                                                         |                           |
|----------------------------|----------------------|-----------------------------------------------|---------------------------------------------------------|---------------------------|
| Layer constitution         | Layer preparing step | Gas used                                      | Flow rate (SCCM)                                        | Discharging power (W)     |
|                            |                      |                                               |                                                         | Layer thickness ( $\mu$ ) |
| Photosensitive step        | First                | SiH <sub>4</sub>                              | SiH <sub>4</sub> = 400                                  | 300                       |
|                            |                      | B <sub>2</sub> H <sub>6</sub> /H <sub>2</sub> | B <sub>2</sub> H <sub>6</sub> /H <sub>2</sub> = 200 → 0 |                           |
|                            |                      | NH <sub>3</sub>                               | NH <sub>3</sub> = 10 → 0                                |                           |
| Surface layer step         | Second               | SiH <sub>4</sub>                              | SiH <sub>4</sub> = 400                                  | 300                       |
|                            |                      |                                               |                                                         | 21                        |
| Surface layer step         | Third                | SiF <sub>4</sub>                              | SiF <sub>4</sub> = 10                                   | 200                       |
|                            |                      | CH <sub>4</sub>                               | CH <sub>4</sub> = 600                                   | 0.5                       |

Al substrate temperature: 250° C.

Discharging frequency: 13.56 MHz

TABLE 25

| Layer constitution   | Gas used         | Flow rate (SCCM)       | Discharging Power (W) | Layer thickness ( $\mu$ ) |
|----------------------|------------------|------------------------|-----------------------|---------------------------|
| Photosensitive layer | SiF <sub>4</sub> | SiF <sub>4</sub> = 350 | 300                   | 25                        |
|                      | H <sub>2</sub>   | H <sub>2</sub> = 300   |                       |                           |
|                      | CH <sub>4</sub>  | CH <sub>4</sub> = 5    |                       |                           |
| Surface layer        | SiF <sub>4</sub> | SiF <sub>4</sub> = 20  | 200                   | 0.5                       |
|                      | NH <sub>3</sub>  | NH <sub>3</sub> = 600  |                       |                           |

25

Al substrate temperature: 250° C.

Discharging frequency: 13.56 MHz

## EXAMPLES 26-35

Light receiving members were prepared on Al supports (cylinder Nos. 103-106) of Example 1 in the same manner as in Example 1 except for forming these light receiving layers in accordance with the layer forming conditions shown in Tables 26 through 35. In the examples each of the examples, the flow rates for the gases used upon forming the layers and upon forming the surface layers were automatically adjusted under the microcomputer control in accordance with the flow rate variation chart described in Table A.

The boron atoms to be contained in the photosensitive layer were so-introduced that B<sub>2</sub>H<sub>6</sub>SiF<sub>4</sub>=100 ppm and the atoms were doped to about 200 ppm over the entire layer.

TABLE 26

| Layer constitution   | Layer preparing step | Gas used         | Flow rate (SCCM)            | Discharging power (W) | Layer thickness ( $\mu$ ) |
|----------------------|----------------------|------------------|-----------------------------|-----------------------|---------------------------|
| Photosensitive layer | First                | SiH <sub>4</sub> | SiH <sub>4</sub> = 350      | 300                   | 25                        |
|                      |                      | H <sub>2</sub>   | H <sub>2</sub> = 300        |                       |                           |
| Surface layer        | Second               | SiF <sub>4</sub> | SiF <sub>4</sub> = 350 → 10 | 300 → 200             | 1.5                       |
|                      |                      | H <sub>2</sub>   | H <sub>2</sub> = 300 → 0    |                       |                           |
|                      |                      | CH <sub>4</sub>  | CH <sub>4</sub> = 0 → 600   |                       |                           |

Al substrate temperature: 250° C.

Discharging frequency: 13.56 MHz

TABLE 27

| Layer constitution   | Layer preparing step | Gas used                                      | Flow rate (SCCM)                                    | Discharging power (W) | Layer thickness ( $\mu$ ) |
|----------------------|----------------------|-----------------------------------------------|-----------------------------------------------------|-----------------------|---------------------------|
| Photosensitive layer | First                | SiF <sub>4</sub>                              | SiF <sub>4</sub> = 350                              | 300                   | 3                         |
|                      |                      | H <sub>2</sub>                                | H <sub>2</sub> = 120                                |                       |                           |
|                      |                      | B <sub>2</sub> H <sub>6</sub> /H <sub>2</sub> | B <sub>2</sub> H <sub>6</sub> /H <sub>2</sub> = 180 |                       |                           |
| Surface layer        | Second               | SiF <sub>4</sub>                              | SiF <sub>4</sub> = 350                              | 300                   | 23                        |
|                      |                      | H <sub>2</sub>                                | H <sub>2</sub> = 300                                |                       |                           |
|                      |                      | SiF <sub>4</sub>                              | SiF <sub>4</sub> = 350 → 10                         | 300 → 200             | 1.5                       |
|                      |                      | H <sub>2</sub>                                | H <sub>2</sub> = 300 → 0                            |                       |                           |
|                      |                      | CH <sub>4</sub>                               | CH <sub>4</sub> = 0 → 600                           |                       |                           |

50

55

55

60

65

TABLE 27-continued

| Layer constitution | Layer preparing step | Gas used        | Flow rate (SCCM)          | Discharging power (W) | Layer thickness ( $\mu$ ) |
|--------------------|----------------------|-----------------|---------------------------|-----------------------|---------------------------|
|                    |                      | NH <sub>3</sub> | NH <sub>3</sub> = 0 → 600 |                       |                           |

Al substrate temperature: 250° C.

Discharging frequency: 13.56 MHz

TABLE 28

| Layer constitution   | Layer preparing step | Gas used                                     | Flow rate (SCCM)                        | Discharging power (W) | Layer thickness ( $\mu$ ) |
|----------------------|----------------------|----------------------------------------------|-----------------------------------------|-----------------------|---------------------------|
| Photosensitive layer | First                | SiF <sub>4</sub>                             | SiF <sub>4</sub> = 350                  | 300                   | 5                         |
|                      |                      | H <sub>2</sub>                               | H <sub>2</sub> = 0 → 300                |                       |                           |
|                      |                      | B <sub>2</sub> H <sub>6</sub> H <sub>2</sub> | B <sub>2</sub> H <sub>6</sub> = 300 → 0 |                       |                           |
| Surface layer        | Second               | SiF <sub>4</sub>                             | SiF <sub>4</sub> = 350                  | 300                   | 20                        |
|                      |                      | H <sub>2</sub>                               | H <sub>2</sub> = 300                    |                       |                           |
| Surface layer        | Third                | SiF <sub>4</sub>                             | SiF <sub>4</sub> = 350 → 100            | 300 →                 | 1.5                       |
|                      |                      | H <sub>2</sub>                               | H <sub>2</sub> = 300 → 0                | 200                   |                           |
|                      |                      | NO                                           | NO = 0 → 500                            |                       |                           |

Al substrate temperature: 250° C.

Discharging frequency: 13.56 MHz

TABLE 29

| Layer constitution   | Layer preparing step | Gas used                                      | Flow rate (SCCM)                        | Discharging power (W) | Layer thickness ( $\mu$ ) |
|----------------------|----------------------|-----------------------------------------------|-----------------------------------------|-----------------------|---------------------------|
| Photosensitive layer | First                | SiF <sub>4</sub>                              | SiF <sub>4</sub> = 300                  | 300                   | 3                         |
|                      |                      | H <sub>2</sub>                                | H <sub>2</sub> = 120                    |                       |                           |
|                      |                      | B <sub>2</sub> H <sub>6</sub> /H <sub>2</sub> | B <sub>2</sub> H <sub>6</sub> = 180     |                       |                           |
| Surface layer        | Second               | SiF <sub>4</sub>                              | SiF <sub>4</sub> = 300                  | 300                   | 1                         |
|                      |                      | H <sub>2</sub>                                | H <sub>2</sub> = 120 → 300              |                       |                           |
|                      |                      | B <sub>2</sub> H <sub>6</sub> H <sub>2</sub>  | B <sub>2</sub> H <sub>6</sub> = 180 → 0 |                       |                           |
| Surface layer        | Third                | SiF <sub>4</sub>                              | SiF <sub>4</sub> = 300                  | 300                   | 21                        |
|                      |                      | H <sub>2</sub>                                | H <sub>2</sub> = 300                    |                       |                           |
| Surface layer        | Fourth               | SiF <sub>4</sub>                              | SiF <sub>4</sub> = 300 → 10             | 300 →                 | 1.5                       |
|                      |                      | H <sub>2</sub>                                | H <sub>2</sub> = 300 → 0                | 200                   |                           |
|                      |                      | NH <sub>3</sub>                               | NH <sub>3</sub> = 0 → 600               |                       |                           |

Al substrate temperature: 250° C.

Discharging frequency: 13.56 MHz

TABLE 30

| Layer constitution   | Layer preparing step | Gas used         | Flow rate (SCCM)            | Discharging power (W) | Layer thickness ( $\mu$ ) |
|----------------------|----------------------|------------------|-----------------------------|-----------------------|---------------------------|
| Photosensitive layer | First                | SiF <sub>4</sub> | SiF <sub>4</sub> = 300      | 300                   | 25                        |
|                      |                      | H <sub>2</sub>   | H <sub>2</sub> = 300        |                       |                           |
|                      |                      | CH <sub>4</sub>  | CH <sub>4</sub> = 5         |                       |                           |
| Surface layer        | Second               | SiF <sub>4</sub> | SiF <sub>4</sub> = 300 → 10 | 300 →                 | 1.5                       |
|                      |                      | H <sub>2</sub>   | H <sub>2</sub> = 300 → 0    | 200                   |                           |

TABLE 30-continued

| Layer<br>constitu-<br>tion | Layer<br>pre-<br>paring<br>step | Gas<br>used     | Flow rate<br>(SCCM)       | Discharg-<br>ing power<br>(W) | Layer<br>thick-<br>ness<br>( $\mu$ ) |
|----------------------------|---------------------------------|-----------------|---------------------------|-------------------------------|--------------------------------------|
|                            |                                 | CH <sub>4</sub> | CH <sub>4</sub> = 5 → 600 |                               |                                      |

Al substrate temperature: 250° C.

Discharging frequency: 13.56 MHz

TABLE 31

| Layer<br>constitu-<br>tion   | Layer<br>pre-<br>paring<br>step | Gas<br>used      | Flow rate<br>(SCCM)    | Discharg-<br>ing power<br>(W) | Layer<br>thick-<br>ness<br>( $\mu$ ) |
|------------------------------|---------------------------------|------------------|------------------------|-------------------------------|--------------------------------------|
| Photo-<br>sensitive<br>layer | First<br>step                   | SiF <sub>4</sub> | SiF <sub>4</sub> = 350 | 300                           | 3                                    |
|                              | Second<br>step                  | H <sub>2</sub>   | H <sub>2</sub> = 300   | 300                           | 23                                   |
| Surface<br>layer             | Third<br>step                   | CH <sub>4</sub>  | CH <sub>4</sub> = 10   |                               |                                      |
|                              |                                 | SiF <sub>4</sub> | SiF <sub>4</sub> = 350 | 300 → 200                     | 1.5                                  |

Al substrate temperature: 250° C.

Discharging frequency: 13.56 MHz

TABLE 32

| Layer<br>constitu-<br>tion | Layer<br>pre-<br>paring<br>step | Gas<br>used      | Flow rate<br>(SCCM)    | Discharg-<br>ing power<br>(W) | Layer<br>thick-<br>ness<br>( $\mu$ ) |
|----------------------------|---------------------------------|------------------|------------------------|-------------------------------|--------------------------------------|
| Photo-                     | First                           | SiF <sub>4</sub> | SiF <sub>4</sub> = 350 | 300                           | 2                                    |

| Layer<br>constitu-<br>tion | Layer<br>pre-<br>paring<br>step | Gas<br>used    | Flow rate<br>(SCCM)  | Discharg-<br>ing power<br>(W) | Layer<br>thick-<br>ness<br>( $\mu$ ) |
|----------------------------|---------------------------------|----------------|----------------------|-------------------------------|--------------------------------------|
|                            | step                            | H <sub>2</sub> | H <sub>2</sub> = 300 |                               |                                      |

Al substrate temperature: 250° C.

Discharging frequency: 13.56 MHz

TABLE 33

| Layer<br>constitu-<br>tion        | Layer<br>pre-<br>paring<br>step | Gas<br>used                                   | Flow rate<br>(SCCM)                                 | Discharg-<br>ing power<br>(W) | Layer<br>thick-<br>ness<br>( $\mu$ ) |
|-----------------------------------|---------------------------------|-----------------------------------------------|-----------------------------------------------------|-------------------------------|--------------------------------------|
| Photo-<br>sensi-<br>tive<br>layer | First<br>step                   | SiF <sub>4</sub>                              | SiF <sub>4</sub> = 300                              | 300                           | 3                                    |
|                                   | Second<br>step                  | H <sub>2</sub>                                | H <sub>2</sub> = 120                                |                               |                                      |
| Sur-<br>face<br>layer             | Third<br>step                   | NH <sub>3</sub>                               | NH <sub>3</sub> = 5                                 |                               |                                      |
|                                   |                                 | B <sub>2</sub> H <sub>6</sub> /H <sub>2</sub> | B <sub>2</sub> H <sub>6</sub> /H <sub>2</sub> = 180 |                               |                                      |
| Sur-<br>face<br>layer             | Second<br>step                  | SiF <sub>4</sub>                              | SiF <sub>4</sub> = 300                              | 300                           | 22                                   |
|                                   |                                 | H <sub>2</sub>                                | H <sub>2</sub> = 300                                |                               |                                      |
| Sur-<br>face<br>layer             | Third<br>step                   | NH <sub>3</sub>                               | NH <sub>3</sub> = 5                                 |                               |                                      |
|                                   |                                 | SiF <sub>4</sub>                              | SiF <sub>4</sub> = 300 → 10                         | 300 → 200                     | 1.5                                  |

Al substrate temperature: 250° C.

Discharging frequency: 13.56 MHz

TABLE 34

| Layer<br>constitu-<br>tion   | Layer<br>pre-<br>paring<br>step | Gas<br>used                                   | Flow rate<br>(SCCM)                                     | Discharg-<br>ing power<br>(W) | Layer<br>thick-<br>ness<br>( $\mu$ ) |
|------------------------------|---------------------------------|-----------------------------------------------|---------------------------------------------------------|-------------------------------|--------------------------------------|
| Photo-<br>sensitive<br>layer | First<br>step                   | SiF <sub>4</sub>                              | SiF <sub>4</sub> = 350                                  | 300                           | 3                                    |
|                              |                                 | H <sub>2</sub>                                | H <sub>2</sub> = 120                                    |                               |                                      |
|                              |                                 | NH <sub>3</sub>                               | NH <sub>3</sub> = 10                                    |                               |                                      |
| Sur-<br>face<br>layer        | Second<br>step                  | B <sub>2</sub> H <sub>6</sub> /H <sub>2</sub> | B <sub>2</sub> H <sub>6</sub> /H <sub>2</sub> = 180     |                               |                                      |
|                              |                                 | SiF <sub>4</sub>                              | SiF <sub>4</sub> = 350                                  | 300                           | 2                                    |
| Sur-<br>face<br>layer        | Third<br>step                   | H <sub>2</sub>                                | H <sub>2</sub> = 120 → 300                              |                               |                                      |
|                              |                                 | B <sub>2</sub> H <sub>6</sub> /H <sub>2</sub> | B <sub>2</sub> H <sub>6</sub> /H <sub>2</sub> = 180 → 0 |                               |                                      |
| Sur-<br>face<br>layer        | Fourth<br>step                  | SiF <sub>4</sub>                              | SiF <sub>4</sub> = 350                                  | 300                           | 20                                   |
|                              |                                 | H <sub>2</sub>                                | H <sub>2</sub> = 300                                    |                               |                                      |

Al substrate temperature: 250° C.

Discharging frequency: 13.56 MHz

| Layer<br>constitu-<br>tion | Layer<br>pre-<br>paring<br>step | Gas<br>used     | Flow rate<br>(SCCM)  | Discharg-<br>ing power<br>(W) | Layer<br>thick-<br>ness<br>( $\mu$ ) |
|----------------------------|---------------------------------|-----------------|----------------------|-------------------------------|--------------------------------------|
| sensi-<br>tive<br>layer    | step                            | H <sub>2</sub>  | H <sub>2</sub> = 300 |                               |                                      |
|                            | Second                          | CH <sub>4</sub> | CH <sub>4</sub> = 10 |                               |                                      |

Second SiF<sub>4</sub> SiF<sub>4</sub> = 350

| Layer<br>constitu-<br>tion   | Layer<br>pre-<br>paring<br>step | Gas<br>used                                   | Flow rate<br>(SCCM)                                 | Discharg-<br>ing power<br>(W) | Layer<br>thick-<br>ness<br>( $\mu$ ) |
|------------------------------|---------------------------------|-----------------------------------------------|-----------------------------------------------------|-------------------------------|--------------------------------------|
| Photo-<br>sensitive<br>layer | First<br>step                   | SiF <sub>4</sub>                              | SiF <sub>4</sub> = 300                              | 300                           | 3                                    |
|                              |                                 | H <sub>2</sub>                                | H <sub>2</sub> = 120                                |                               |                                      |
|                              |                                 | NO                                            | NO = 10                                             |                               |                                      |
| Sur-<br>face<br>layer        | Second<br>step                  | B <sub>2</sub> H <sub>6</sub> /H <sub>2</sub> | B <sub>2</sub> H <sub>6</sub> /H <sub>2</sub> = 180 |                               |                                      |
|                              |                                 | SiF <sub>4</sub>                              | SiF <sub>4</sub> = 300                              | 300                           | 1                                    |
| Sur-<br>face<br>layer        | Third<br>step                   | H <sub>2</sub>                                | H <sub>2</sub> = 300                                |                               | 21                                   |
|                              |                                 | SiF <sub>4</sub>                              | SiF <sub>4</sub> = 300                              | 300                           | 1.5                                  |

Al substrate temperature: 250° C.

Discharging frequency: 13.56 MHz

TABLE A

| Example No. | Chart showing the flow rate change of gas used in forming photosensitive layer | Chart showing the flow rate change of gas used in forming surface layer |
|-------------|--------------------------------------------------------------------------------|-------------------------------------------------------------------------|
| 26          | —                                                                              | FIG. 31                                                                 |
| 27          | —                                                                              | FIG. 32                                                                 |
| 28          | FIG. 33                                                                        | FIG. 34                                                                 |
| 29          | FIG. 22                                                                        | FIG. 35                                                                 |
| 30          | —                                                                              | FIG. 36                                                                 |
| 31          | —                                                                              | FIG. 37                                                                 |
| 32          | FIG. 38                                                                        | FIG. 39                                                                 |
| 33          | —                                                                              | FIG. 40                                                                 |
| 34          | FIG. 41                                                                        | FIG. 42                                                                 |
| 35          | FIG. 43                                                                        | FIG. 37                                                                 |

## EXAMPLES 36-46

Photosensitive layers were formed on Al supports (cylinder Nos. 103-106) used in Example 1 in accordance with layer forming conditions shown in each of Tables 36 through 46.

Subsequently, surface layers were formed by means of sputtering process using surface layer forming materials (1-20) shown in the upper column of Table B to the layer thickness shown in the lower column of Table B in Examples 36 and 36, while the surface layers were formed by means of sputtering process using layer constituent materials shown in the upper column of Table C to the layer thickness shown in the lower column of Table C in Examples 38-46.

In the Examples 36, 37, 42, 43, 45 and 46, the gases used when forming the photosensitive layers were automatically adjusted in accordance with the flow rate variation curves shown in each of FIGS. 33, 22, 38, 44, 45 and 41 under the control of a microcomputer. Further, boron atoms contained in the photosensitive layers were introduced in each of the examples under the same conditions as those in Example 1.

When images were formed on these light receiving members in the same manner as in Example 1, same satisfactory results as in Example 1 were obtained.

TABLE 36

| (Variation chart: FIG. 33) |                      |                                                                                     |                                                                                               |                                        |                     |
|----------------------------|----------------------|-------------------------------------------------------------------------------------|-----------------------------------------------------------------------------------------------|----------------------------------------|---------------------|
| Layer constituting step    | Layer preparing step | Gas used                                                                            | Flow rate (SCCM)                                                                              | Discharging power (W/cm <sup>2</sup> ) | Layer thickness (μ) |
| Photosensitive layer       | First step           | SiF <sub>4</sub><br>H <sub>2</sub><br>B <sub>2</sub> H <sub>6</sub> /H <sub>2</sub> | SiF <sub>4</sub> = 350<br>H <sub>2</sub> = 0 → 300<br>B <sub>2</sub> H <sub>6</sub> = 300 → 0 | 300                                    | 5                   |
|                            | Second step          | SiF <sub>4</sub><br>H <sub>2</sub>                                                  | SiF <sub>4</sub> = 350<br>H <sub>2</sub> = 300                                                | 300                                    | 20                  |

Al substrate temperature: 250° C.

Discharging frequency: 13.56 MHz

TABLE 37

| (Variation chart: FIG. 22) |                      |                                                                                     |                                                                                                                 |                                        |                     |
|----------------------------|----------------------|-------------------------------------------------------------------------------------|-----------------------------------------------------------------------------------------------------------------|----------------------------------------|---------------------|
| Layer constituting step    | Layer preparing step | Gas used                                                                            | Flow rate (SCCM)                                                                                                | Discharging power (W/cm <sup>2</sup> ) | Layer thickness (μ) |
| Photosensitive             | First step           | SiF <sub>4</sub><br>H <sub>2</sub><br>B <sub>2</sub> H <sub>6</sub> /H <sub>2</sub> | SiF <sub>4</sub> = 300<br>H <sub>2</sub> = 120<br>B <sub>2</sub> H <sub>6</sub> = 180                           | 300                                    | 3                   |
|                            | Second step          | SiF <sub>4</sub><br>H <sub>2</sub>                                                  | SiF <sub>4</sub> = 300<br>H <sub>2</sub> = 120 → 300<br>B <sub>2</sub> H <sub>6</sub> /H <sub>2</sub> = 180 → 0 | 300                                    | 1                   |
|                            | Third step           | SiF <sub>4</sub>                                                                    | SiF <sub>4</sub> = 300                                                                                          | 300                                    | 21                  |

TABLE 37-continued

| (Variation chart: FIG. 22) |                      |                |                      |                                        |                     |
|----------------------------|----------------------|----------------|----------------------|----------------------------------------|---------------------|
| Layer constituting step    | Layer preparing step | Gas used       | Flow rate (SCCM)     | Discharging power (W/cm <sup>2</sup> ) | Layer thickness (μ) |
| 5                          | step                 | H <sub>2</sub> | H <sub>2</sub> = 300 |                                        |                     |

Al substrate temperature: 250° C.  
Discharging frequency: 13.56 MHz

TABLE 38

| Layer constituting step | Layer preparing step  | Gas used   | Flow rate (SCCM)                   | Discharging power (W/cm <sup>2</sup> )         | Layer thickness (μ) |
|-------------------------|-----------------------|------------|------------------------------------|------------------------------------------------|---------------------|
| 15                      | Photo-sensitive layer | First step | SiF <sub>4</sub><br>H <sub>2</sub> | SiF <sub>4</sub> = 350<br>H <sub>2</sub> = 300 | 300                 |

Al substrate temperature: 250° C.  
Discharging frequency: 13.56 MHz

TABLE 39

| Layer constituting step | Layer preparing step  | Gas used    | Flow rate (SCCM)                                                                    | Discharging power (W/cm <sup>2</sup> )                                                                | Layer thickness (μ) |
|-------------------------|-----------------------|-------------|-------------------------------------------------------------------------------------|-------------------------------------------------------------------------------------------------------|---------------------|
| 25                      | Photo-sensitive layer | First step  | SiF <sub>4</sub><br>H <sub>2</sub><br>B <sub>2</sub> H <sub>6</sub> /H <sub>2</sub> | SiF <sub>4</sub> = 350<br>H <sub>2</sub> = 120<br>B <sub>2</sub> H <sub>6</sub> /H <sub>2</sub> = 180 | 300                 |
|                         |                       | Second step | SiF <sub>4</sub><br>H <sub>2</sub>                                                  | SiF <sub>4</sub> = 350<br>H <sub>2</sub> = 300                                                        | 23                  |
| 30                      |                       |             |                                                                                     |                                                                                                       |                     |

Al substrate temperature: 250° C.  
Discharging frequency: 13.56 MHz

TABLE 40

| Layer constituting step | Layer preparing step  | Gas used   | Flow rate (SCCM)                                      | Discharging power (W/cm <sup>2</sup> )                                | Layer thickness (μ) |
|-------------------------|-----------------------|------------|-------------------------------------------------------|-----------------------------------------------------------------------|---------------------|
| 35                      | Photo-sensitive layer | First step | SiF <sub>4</sub><br>H <sub>2</sub><br>CH <sub>4</sub> | SiF <sub>4</sub> = 300<br>H <sub>2</sub> = 300<br>CH <sub>4</sub> = 5 | 25                  |
|                         |                       |            |                                                       |                                                                       |                     |

Al substrate temperature: 250° C.  
Discharging frequency: 13.56 MHz

TABLE 41

| Layer constituting step | Layer preparing step  | Gas used    | Flow rate (SCCM)                                      | Discharging power (W/cm <sup>2</sup> )                                 | Layer thickness (μ) |
|-------------------------|-----------------------|-------------|-------------------------------------------------------|------------------------------------------------------------------------|---------------------|
| 45                      | Photo-sensitive layer | First step  | SiF <sub>4</sub><br>H <sub>2</sub><br>CH <sub>4</sub> | SiF <sub>4</sub> = 350<br>H <sub>2</sub> = 300<br>CH <sub>4</sub> = 10 | 3                   |
|                         |                       | Second step | SiF <sub>4</sub><br>H <sub>2</sub>                    | SiF <sub>4</sub> = 350<br>H <sub>2</sub> = 300                         | 23                  |
| 50                      |                       |             |                                                       |                                                                        |                     |

Al substrate temperature: 250° C.  
Discharging frequency: 13.56 MHz

55

TABLE 42

| Layer constituting step | Layer preparing step  | Gas used    | Flow rate (SCCM)                                      | Discharging power (W/cm <sup>2</sup> )                                       | Layer thickness (μ) |
|-------------------------|-----------------------|-------------|-------------------------------------------------------|------------------------------------------------------------------------------|---------------------|
| 60                      | Photo-sensitive layer | First step  | SiF <sub>4</sub><br>H <sub>2</sub><br>CH <sub>4</sub> | SiF <sub>4</sub> = 350<br>H <sub>2</sub> = 300<br>CH <sub>4</sub> = 10       | 2                   |
|                         |                       | Second step | SiF <sub>4</sub><br>H <sub>2</sub><br>CH <sub>4</sub> | SiF <sub>4</sub> = 350<br>H <sub>2</sub> = 300<br>CH <sub>4</sub> = 10 → 0.5 | 2                   |
| 65                      |                       | Third step  | SiF <sub>4</sub><br>H <sub>2</sub>                    | SiF <sub>4</sub> = 350<br>H <sub>2</sub> = 300                               | 21                  |

TABLE 42-continued

(Variation chart: FIG. 38)

| Layer constitution | Layer preparing step | Gas used        | Flow rate (SCCM)      | Discharging power (W/cm <sup>2</sup> ) | Layer thickness (μ) |
|--------------------|----------------------|-----------------|-----------------------|----------------------------------------|---------------------|
|                    |                      | CH <sub>4</sub> | CH <sub>4</sub> = 0.5 |                                        |                     |

Al substrate temperature: 250° C.

Discharging frequency: 13.56 MHz

TABLE 43-continued

(Variation chart: FIG. 44)

| Layer constitution | Layer preparing step | Gas used         | Flow rate (SCCM)       | Discharging power (W/cm <sup>2</sup> ) | Layer thickness (μ) |
|--------------------|----------------------|------------------|------------------------|----------------------------------------|---------------------|
|                    | Fifth step           | SiF <sub>4</sub> | SiF <sub>4</sub> = 100 | 300 → 200                              | 3                   |

Al substrate temperature: 250° C.

Discharging frequency: 13.56 MHz

TABLE 43

TABLE 44

| Layer constitution    | Layer preparing step | Gas used                                      | Flow rate (SCCM)                                    | Discharging power (W/cm <sup>2</sup> ) | Layer thickness (μ) |
|-----------------------|----------------------|-----------------------------------------------|-----------------------------------------------------|----------------------------------------|---------------------|
| Photo-sensitive layer | First step           | SiF <sub>4</sub>                              | SiF <sub>4</sub> = 300                              | 300                                    | 3                   |
|                       |                      | H <sub>2</sub>                                | H <sub>2</sub> = 120                                |                                        |                     |
|                       |                      | NH <sub>3</sub>                               | NH <sub>3</sub> = 5                                 |                                        |                     |
|                       |                      | B <sub>2</sub> H <sub>6</sub> /H <sub>2</sub> | B <sub>2</sub> H <sub>6</sub> /H <sub>2</sub> = 180 |                                        |                     |
|                       | Second step          | SiF <sub>4</sub>                              | SiF <sub>4</sub> = 300                              | 300                                    | 22                  |
|                       |                      | H <sub>2</sub>                                | H <sub>2</sub> = 300                                |                                        |                     |
|                       |                      | NH <sub>3</sub>                               | NH <sub>3</sub> = 5                                 |                                        |                     |

Al substrate temperature: 250° C.

Discharging frequency: 13.56 MHz

TABLE 45

(Variation chart: FIG. 45)

| Layer constitution    | Layer preparing step | Gas used                                      | Flow rate (SCCM)                    | Discharging power (W/cm <sup>2</sup> ) | Layer thickness (μ) |
|-----------------------|----------------------|-----------------------------------------------|-------------------------------------|----------------------------------------|---------------------|
| Photo-sensitive layer | First step           | SiF <sub>4</sub>                              | SiF <sub>4</sub> = 300              | 300                                    | 3                   |
|                       |                      | H <sub>2</sub>                                | H <sub>2</sub> = 120                |                                        |                     |
|                       |                      | NO                                            | NO = 10                             |                                        |                     |
|                       |                      | B <sub>2</sub> H <sub>6</sub> /H <sub>2</sub> | B <sub>2</sub> H <sub>4</sub> = 180 |                                        |                     |
|                       | Second step          | SiF <sub>4</sub>                              | SiF <sub>4</sub> = 300              | 300                                    | 1                   |
|                       |                      | H <sub>2</sub>                                | H <sub>2</sub> = 300                |                                        |                     |
|                       |                      | NO                                            | NO = 10 → 0                         |                                        |                     |
|                       | Third step           | SiF <sub>4</sub>                              | SiF <sub>4</sub> = 300              | 300                                    | 15                  |
|                       |                      | H <sub>2</sub>                                | H <sub>2</sub> = 300                |                                        |                     |
|                       | Fourth step          | SiF <sub>4</sub>                              | SiF <sub>4</sub> = 300 → 20         | 300 → 20                               | 2                   |
|                       |                      | H <sub>2</sub>                                | H <sub>2</sub> = 300 → 0            |                                        |                     |
|                       |                      | CH <sub>4</sub>                               | CH <sub>4</sub> = 0 → 600           |                                        |                     |
|                       | Fifth step           | SiF <sub>4</sub>                              | SiF <sub>4</sub> = 20               | 300 → 200                              | 3                   |
|                       |                      | CH <sub>4</sub>                               | CH <sub>4</sub> = 600               |                                        |                     |

Al substrate temperature: 250° C.

Discharging frequency: 13.56 MHz

(Variation chart: FIG. 44)

| Layer constitution    | Layer preparing step | Gas used         | Flow rate (SCCM)             | Discharging power (W/cm <sup>2</sup> ) | Layer thickness (μ) |
|-----------------------|----------------------|------------------|------------------------------|----------------------------------------|---------------------|
| Photo-sensitive layer | First step           | SiF <sub>4</sub> | SiF <sub>4</sub> = 300       | 300                                    | 3                   |
|                       |                      | H <sub>2</sub>   | H <sub>2</sub> = 300         |                                        |                     |
|                       |                      | CH <sub>4</sub>  | CH <sub>4</sub> = 10         |                                        |                     |
|                       | Second step          | SiF <sub>4</sub> | SiF <sub>4</sub> = 300       | 300                                    | 2                   |
|                       |                      | H <sub>2</sub>   | H <sub>2</sub> = 300         |                                        |                     |
|                       |                      | CH <sub>4</sub>  | CH <sub>4</sub> = 10 → 0     |                                        |                     |
|                       | Third step           | SiF <sub>4</sub> | SiF <sub>4</sub> = 300       | 300                                    | 15                  |
|                       |                      | H <sub>2</sub>   | H <sub>2</sub> = 300         |                                        |                     |
|                       | Fourth step          | SiF <sub>4</sub> | SiF <sub>4</sub> = 300 → 100 | 300 → 200                              | 2                   |
|                       |                      | H <sub>2</sub>   | H <sub>2</sub> = 300 → 0     |                                        |                     |
|                       |                      | CH <sub>4</sub>  | CH <sub>4</sub> = 0 → 500    |                                        |                     |

TABLE 46

(Variation chart: FIG. 41)

| Layer constitution    | Layer preparing step | Gas used                                      | Flow rate (SCCM)                                        | Layer thickness (μ) |
|-----------------------|----------------------|-----------------------------------------------|---------------------------------------------------------|---------------------|
| Photo-sensitive layer | First step           | SiF <sub>4</sub>                              | SiF <sub>4</sub> = 350                                  | 3                   |
|                       |                      | H <sub>2</sub>                                | H <sub>2</sub> = 120                                    |                     |
|                       |                      | NH <sub>3</sub>                               | NH <sub>3</sub> = 10                                    |                     |
|                       |                      | B <sub>2</sub> H <sub>6</sub> /H <sub>2</sub> | B <sub>2</sub> H <sub>6</sub> /H <sub>2</sub> = 180     |                     |
|                       | Second step          | SiF <sub>4</sub>                              | SiF <sub>4</sub> = 350                                  | 2                   |
|                       |                      | H <sub>2</sub>                                | H <sub>2</sub> = 120 → 300                              |                     |
|                       |                      | B <sub>2</sub> H <sub>6</sub> /H <sub>2</sub> | B <sub>2</sub> H <sub>6</sub> /H <sub>2</sub> = 180 → 0 |                     |
|                       | Third step           | SiF <sub>4</sub>                              | SiF <sub>4</sub> = 350                                  | 20                  |
|                       |                      | H <sub>2</sub>                                | H <sub>2</sub> = 300                                    |                     |

Al substrate temperature: 250° C.

Discharging frequency: 13.56 MHz

TABLE B

| Condition No.                                          | 1                | 2 | 3                | 4 | 5                                                      | 6 | 7                                                | 8 | 9                | 10 |
|--------------------------------------------------------|------------------|---|------------------|---|--------------------------------------------------------|---|--------------------------------------------------|---|------------------|----|
| Constituent condition for surface layer (mixing ratio) | ZrO <sub>2</sub> |   | TiO <sub>2</sub> |   | ZrO <sub>2</sub> /Ti <sub>2</sub> O <sub>5</sub> = 6/1 |   | TiO <sub>2</sub> /Zr <sub>2</sub> O <sub>7</sub> |   | CeO <sub>2</sub> |    |
| Refractive index                                       | 2.00             |   | 2.26             |   | 2.09                                                   |   | 2.20                                             |   | 2.23             |    |

TABLE B-continued

| Layer thickness (μm)                                   | 0.0975 | 0.293 | 0.0863                         | 0.259 | 0.0933           | 0.280 | 0.0886                                                 | 0.266 | 0.0874           | 0.262 |
|--------------------------------------------------------|--------|-------|--------------------------------|-------|------------------|-------|--------------------------------------------------------|-------|------------------|-------|
| Condition No.                                          | 11     | 12    | 13                             | 14    | 15               | 16    | 17                                                     | 18    | 19               | 20    |
| Constituent condition for surface layer (mixing ratio) | ZnS    |       | Al <sub>2</sub> O <sub>3</sub> |       | CeF <sub>3</sub> |       | Al <sub>2</sub> O <sub>3</sub> /ZrO <sub>2</sub> = 1/1 |       | MgF <sub>2</sub> |       |
| Refractive index                                       | 2.24   |       | 1.63                           |       | 1.60             |       | 1.68                                                   |       | 1.38             |       |
| Layer thickness (μm)                                   | 0.0871 | 0.261 | 0.120                          | 0.359 | 0.123            | 0.366 | 0.116                                                  | 0.348 | 0.141            | 0.424 |

TABLE C

| Example No.                                            | 38,39            | 40               | 41                                       | 42               | 43    | 44                             | 45               | 46    |
|--------------------------------------------------------|------------------|------------------|------------------------------------------|------------------|-------|--------------------------------|------------------|-------|
| Constituent condition for surface layer (mixing ratio) | ZrO <sub>2</sub> | TiO <sub>2</sub> | ZrO <sub>2</sub> /TiO <sub>2</sub> = 6/1 | CeO <sub>2</sub> | ZnS   | Al <sub>2</sub> O <sub>3</sub> | CeF <sub>3</sub> | MgF   |
| Refractive index                                       | 2.00             | 2.26             | 2.09                                     | 2.23             | 2.24  | 1.63                           | 1.60             | 1.38  |
| Layer thickness (μm)                                   | 0.293            | 0.256            | 0.280                                    | 0.262            | 0.261 | 0.359                          | 0.366            | 0.424 |

## EXAMPLES 47-66

Light receiving layers were formed on Al supports (sample Nos. 103-106) used in Example 1 under the layer preparing conditions shown in Tables D and E.

When forming images on the light receiving members thus obtained in the same manner as in Example 1, occurrence of interference fringe was not observed in any of the thus obtained images and the image quality was extremely good.

TABLE D

| Example No. | Photosensitive layer inhibition layer | Surface layer                                                           |              |             |                          |
|-------------|---------------------------------------|-------------------------------------------------------------------------|--------------|-------------|--------------------------|
|             |                                       | Reflection preventive layer (inside layer) from the side of the support |              |             | Abrasion-resistant layer |
|             |                                       | First layer                                                             | Second layer | Third layer | (outermost layer)        |
| 47          | —                                     | 19                                                                      | 2            | —           | 3                        |
| 48          | —                                     | 19                                                                      | 8            | —           | 5                        |
| 49          | —                                     | 20                                                                      | 12           | —           | 5                        |
| 50          | —                                     | 20                                                                      | 12           | —           | 16                       |
| 51          | —                                     | 20                                                                      | 12           | 13          | 3                        |

Numerals in the table represent the layer No. shown in Table B.

TABLE D-continued

| Example No. | Photosensitive layer inhibition layer | Surface layer          |                                                                         |             | Abrasion-resistant layer |             |    |
|-------------|---------------------------------------|------------------------|-------------------------------------------------------------------------|-------------|--------------------------|-------------|----|
|             |                                       | Charge injection layer | Reflection preventive layer (inside layer) from the side of the support | First layer | Second layer             | Third layer |    |
| 52          | —                                     | —                      | 20                                                                      | 12          | 13                       | 4           | 1  |
| 53          | —                                     | —                      | 17                                                                      | 4           | —                        | —           | 1  |
| 54          | —                                     | —                      | 18                                                                      | 4           | —                        | —           | 1  |
| 55          | —                                     | 23                     | 20                                                                      | 6           | —                        | —           | 7  |
| 56          | —                                     | 24                     | 20                                                                      | 4           | —                        | —           | 9  |
| 57          | —                                     | 25                     | 20                                                                      | 4           | —                        | —           | 10 |
| 58          | —                                     | —                      | 20                                                                      | 4           | —                        | —           | 11 |
| 59          | —                                     | 23                     | 20                                                                      | 13          | —                        | —           | 2  |
| 60          | —                                     | 23                     | 20                                                                      | 14          | —                        | —           | 2  |
| 61          | —                                     | 23                     | 20                                                                      | 15          | —                        | —           | 2  |
| 62          | —                                     | 23                     | 20                                                                      | 14          | 15                       | —           | 2  |
| 63          | —                                     | 23                     | 20                                                                      | 14          | 15                       | 4           | 2  |
| 64          | —                                     | —                      | 21                                                                      | 4           | —                        | —           | 1  |
| 65          | —                                     | 26                     | 21                                                                      | 4           | —                        | —           | 1  |
| 66          | —                                     | 27                     | 22                                                                      | 4           | —                        | —           | 1  |

TABLE E

| Name of layer | Layer No. | Preparing Method<br>GD: Glow discharge<br>SP: Sputter-ing | Layer constituent material | Preparing Condition                                           |                 |                      |       |
|---------------|-----------|-----------------------------------------------------------|----------------------------|---------------------------------------------------------------|-----------------|----------------------|-------|
|               |           |                                                           |                            | Gas used and flow rate, or target and sputter gas used (SCCM) |                 | Layer thickness (μm) |       |
|               |           |                                                           |                            | SiH <sub>4</sub>                                              | CH <sub>4</sub> | SiH <sub>4</sub>     |       |
| Surface layer | 1         | GD                                                        | a-SiCH                     | SiH <sub>4</sub>                                              | gas             | 10                   | 2     |
|               | 2         | GD                                                        | a-SiCH                     | CH <sub>4</sub>                                               | gas             | 600                  | 0.14  |
|               | 3         | GD                                                        | a-SiCH                     | SiH <sub>4</sub>                                              | gas             | 100                  | 3     |
|               | 4         | GD                                                        | a-SiCH                     | CH <sub>4</sub>                                               | gas             | 300                  | 0.076 |
|               | 5         | GD                                                        | a-SiCHF                    | SiH <sub>4</sub>                                              | gas             | 10                   | 1     |
|               | 6         | GD                                                        | a-SiCHF                    | SiF <sub>4</sub>                                              | gas             | 10                   |       |
|               | 7         | GD                                                        | a-SiCHF                    | CH <sub>4</sub>                                               | gas             | 700                  | 0.12  |
|               | 8         | GD                                                        | a-SiNOH                    | SiH <sub>4</sub>                                              | gas             | 70                   | 1.5   |
|               | 9         | GD                                                        | a-SiNOH                    | SiF <sub>4</sub>                                              | gas             | 70                   |       |
|               | 10        | GD                                                        | a-SiNH                     | CH <sub>4</sub>                                               | gas             | 300                  | 0.11  |
|               | 11        | GD                                                        | a-SiNH                     | SiH <sub>4</sub>                                              | gas             | 150                  | 2.5   |
|               |           |                                                           |                            | N <sub>2</sub> O                                              | gas             | 300                  |       |
|               |           |                                                           |                            | SiH <sub>4</sub>                                              | gas             | 100                  | 2     |
|               |           |                                                           |                            | NH <sub>3</sub>                                               | gas             | 300                  |       |
|               |           |                                                           |                            | SiF <sub>4</sub>                                              | gas             | 70                   | 2     |
|               |           |                                                           |                            | SiH <sub>4</sub>                                              | gas             | 70                   |       |

TABLE E-continued

| Name of layer                     | Layer No. | Preparing Method<br>GD: Glow<br>discharge<br>SP: Sputter-<br>ing | Layer constituent material                             | Preparing Condition                                                                      |                                                                                |      |
|-----------------------------------|-----------|------------------------------------------------------------------|--------------------------------------------------------|------------------------------------------------------------------------------------------|--------------------------------------------------------------------------------|------|
|                                   |           |                                                                  |                                                        | Gas used and flow rate, or target and sputter gas used (SCCM)                            | Layer thickness (μm)                                                           |      |
| Photosensitive layer              | 12        | SP                                                               | Al <sub>2</sub> O <sub>3</sub>                         | NH <sub>3</sub><br>Al <sub>2</sub> O <sub>3</sub><br>Ar                                  | gas 250                                                                        | 0.36 |
|                                   | 13        | SP                                                               | SiO <sub>2</sub>                                       | SiO <sub>2</sub><br>Ar                                                                   | gas 360                                                                        | 0.39 |
|                                   | 14        | SP                                                               | Al <sub>2</sub> O <sub>3</sub> /ZrO <sub>2</sub> = 1/1 | Al <sub>2</sub> O <sub>3</sub> /ZrO <sub>2</sub> = 1/1<br>Ar                             | gas 360                                                                        | 0.35 |
|                                   | 15        | SP                                                               | TiO <sub>2</sub>                                       | TiO <sub>2</sub><br>Ar                                                                   | gas 360                                                                        | 0.26 |
|                                   | 16        | SP                                                               | SiO <sub>2</sub>                                       | SiO <sub>2</sub><br>Ar                                                                   | gas 360                                                                        | 1    |
|                                   | 17        | GD                                                               | a-SiH                                                  | SiH <sub>4</sub><br>H <sub>2</sub>                                                       | gas 300<br>gas 360                                                             | 25   |
|                                   | 18        | GD                                                               | a-SiHF                                                 | SiH <sub>4</sub><br>SiF <sub>4</sub>                                                     | gas 200<br>gas 150                                                             | 20   |
|                                   | 19        | GD                                                               | a-SiHB                                                 | H <sub>2</sub><br>SiH <sub>4</sub><br>H <sub>2</sub>                                     | gas 350<br>gas 350<br>gas 360                                                  | 18   |
|                                   | 20        | GD                                                               | a-SiHFB                                                | B <sub>2</sub> H <sub>6</sub><br>SiF <sub>4</sub><br>H <sub>2</sub>                      | 3.5 × 10 <sup>-4</sup><br>gas 300<br>gas 250                                   | 15   |
|                                   | 21        | GD                                                               | a-SiNHB                                                | BF <sub>3</sub><br>SiH <sub>2</sub><br>H <sub>2</sub>                                    | gas 3.5 × 10 <sup>-4</sup><br>gas 300<br>gas 250                               | 15   |
| Charge injection inhibition layer | 22        | GD                                                               | a-SiNOHB                                               | NH <sub>4</sub><br>B <sub>2</sub> H <sub>6</sub><br>SiH <sub>4</sub><br>H <sub>2</sub>   | gas 2.5 × 10 <sup>-1</sup><br>gas 3.5 × 10 <sup>-4</sup><br>gas 300<br>gas 250 | 15   |
|                                   | 23        | GD                                                               | a-SiHB                                                 | NO<br>B <sub>2</sub> H <sub>6</sub><br>SiH <sub>4</sub><br>H <sub>2</sub>                | gas 2.5 × 10 <sup>-1</sup><br>gas 3.5 × 10 <sup>-4</sup><br>gas 350<br>gas 360 | 5    |
|                                   | 24        | GD                                                               | a-SiHFB                                                | B <sub>2</sub> H <sub>6</sub><br>SiH <sub>4</sub><br>SiF <sub>4</sub><br>H <sub>2</sub>  | gas 4.0 × 10 <sup>-2</sup><br>gas 300<br>gas 100<br>gas 150                    | 3    |
|                                   | 25        | GD                                                               | a-SiHFB                                                | B <sub>2</sub> H <sub>6</sub><br>SiH <sub>4</sub><br>SiF <sub>4</sub><br>BF <sub>3</sub> | gas 6.0 × 10 <sup>-2</sup><br>gas 250<br>gas 150<br>gas 6.0 × 10 <sup>-2</sup> | 3.5  |
|                                   | 26        | GD                                                               | a-SiNHB                                                | SiH <sub>4</sub><br>H <sub>2</sub><br>NH <sub>4</sub><br>B <sub>2</sub> H <sub>6</sub>   | gas 350<br>gas 360<br>gas 10<br>gas 4.0 × 10 <sup>-2</sup>                     | 5    |
|                                   | 27        | GD                                                               | a-SiNOHB                                               | SiH <sub>4</sub><br>H <sub>2</sub><br>NO<br>B <sub>2</sub> H <sub>6</sub>                | gas 350<br>gas 360<br>gas 10<br>gas 4.0 × 10 <sup>-2</sup>                     | 5    |

What is claimed is:

1. A light receiving member comprising a support and a light receiving layer of a multi-layered structure having at least a photosensitive layer composed of an amorphous material containing silicon atoms and at least one of the elements selected from oxygen atoms, carbon atoms and nitrogen atoms, said support having a surface provided with irregularities composed of spherical dimples, each of which having an inside face provided with minute irregularities.

2. A light receiving member as defined in claim 1, wherein the irregularities on the surface of the support are composed of spherical dimples having the same diameter of curvature.

3. A light receiving member as defined in claim 1, wherein the irregularities on the surface of the support are composed of spherical dimples having the same diameter of curvature and the same width.

4. A light receiving member as defined in claim 1, wherein the irregularities on the surface of the support are those which are formed by a plurality of rigid

50 spheres each of which having a surface provided with minute irregularities falling spontaneously on the surface of the support.

55 5. A light receiving member as defined in claim 4, wherein the irregularities on the surface of the support are those which are formed by the rigid spheres of almost the same diameter falling spontaneously on the surface of the support from almost the same height.

60 6. A light receiving member as defined in claim 1, wherein the spherical dimples have the radius of curvature R and the width D which satisfy the following equation

$$0.035 \leq (D/R) \leq 0.5.$$

65 7. A light receiving member as defined in claim 6, wherein the spherical dimple has the width D which satisfies the following equation

$D \leq 0.5 \text{ mm.}$ 

8. A light receiving member as defined in claim 1, wherein the minute irregularity has the height  $h$  which satisfies the following equation

$$0.5 \mu\text{m} \leq h \leq 20 \mu\text{m.}$$

9. A light receiving member as defined in claim 1, wherein the support is a metal member.

10. A light receiving member as defined in claim 1, wherein the photosensitive layer contains a substance for controlling the conductivity.

11. A light receiving member as defined in claim 1, wherein the light receiving layer comprises a charge injection inhibition layer containing a substance for controlling the conductivity as one of the constituent layers.

12. A light receiving member as defined in claim 1, wherein the light receiving layer comprises a barrier layer as one of the constituent layers.

13. A light receiving member comprising a support and, a light receiving layer having a photosensitive layer composed of an amorphous material based on silicon atoms and a surface layer, said support having a surface provided with irregularities composed of spherical dimples, each of which having an inside face provided with minute irregularities.

14. A light receiving member as in claim 13, wherein the irregularities on the surface of the support are composed of spherical dimples having the same radius of curvature.

15. A light receiving member as set forth in claim 13, wherein the irregularities on the surface of the support are composed of spherical dimples having the same radius of curvature and the same width.

16. A light receiving member as set forth in claim 13, wherein the irregularities on the surface of the support are those which are formed by a plurality of rigid spheres each of which having a surface provided with minute irregularities falling spontaneously on the surface of the support.

17. A light receiving member as defined in claim 16, wherein the irregularities on the surface of the support are those which are formed by the rigid spheres of almost the same diameter falling spontaneously on the surface of the support from almost the same height.

18. A light receiving member as defined in claim 13, wherein the spherical dimples have the radius of curvature  $R$  and the width  $D$  which satisfy the following equation

$$0.035 \leq D/R \leq 0.5.$$

19. A light receiving member as defined in claim 18, wherein the spherical dimple has the width  $D$  which satisfies the following equation

$$D \leq 0.5 \text{ mm.}$$

20. A light receiving member as defined in claim 13, wherein the minute irregularity has the height  $h$  which satisfies the following equation

$$0.5 \mu\text{m} \leq h \leq 20 \mu\text{m.}$$

21. A light receiving member as defined in claim 13, wherein the support is a metal member.

22. A light receiving member as defined in claim 13, wherein the photosensitive layer contains a substance for controlling the conductivity.

23. A light receiving member as defined in claim 13, wherein the light receiving layer comprises a charge injection inhibition layer containing a substance for controlling the conductivity as one of the constituent layers.

24. A light receiving member as defined in claim 13, wherein the light receiving layer comprises a barrier layer as one of the constituent layers.

25. A light receiving member as defined in claim 13, wherein the surface layer is composed of an amorphous material containing silicon atoms and oxygen atoms.

26. A light receiving member as defined in claim 13, wherein the surface layer is composed of an amorphous material containing silicon atoms and at least one of the elements selected from oxygen atoms, carbon atoms and nitrogen atoms, and optical band gaps are matched at the interface between the photosensitive layer and the surface layer.

27. A light receiving member as defined in claim 13, wherein the surface layer has a reflection preventive function.

28. A light receiving member as defined in claim 27, wherein the surface layer is composed of at least one of the elements selected from inorganic fluorides, inorganic oxides and inorganic sulfides.

29. A light receiving member as defined in claim 28, wherein the thickness  $d$  of the surface layer satisfies the following equation:

$$d = \frac{\lambda}{4n} \text{ m } (m \text{ is a positive odd number})$$

where  $n$  is a refractive index of the substance constituting the surface layer and  $\lambda$  is the wavelength of the irradiation light.

30. A light receiving member as defined in claim 28, wherein the refractive index  $n$  of the substance constituting the surface layer and the refractive index  $n_a$  of the amorphous material constituting the photosensitive layer in adjacent with the surface layer satisfies the following equation:

$$N = \sqrt{n_a}$$

31. A light receiving member as defined in claim 13, wherein the surface layer is constituted as a multi-layered structure comprising an abrasion-resistant layer at the outermost side and a reflection preventive layer in the inside.

32. A light receiving member as defined in claim 31, wherein the surface layer is composed of an amorphous layer containing silicon atoms and at least one of the elements selected from oxygen atoms, carbon atoms and nitrogen atoms.

33. A light receiving member as defined in claim 31, wherein the surface layer is composed of material selected from inorganic fluorides, inorganic oxides and inorganic sulfides.

34. A light receiving member comprising a support and a light receiving layer having a photosensitive layer composed of an amorphous material containing silicon atoms and at least one of the elements selected from oxygen atoms, carbon atoms and nitrogen atoms and a surface layer, said support having a surface provided with irregularities composed of spherical dimples, each

of which having an inside face provided with minute irregularities.

35. A light receiving member as defined in claim 34, wherein the irregularities on the surface of the support are composed of spherical dimples having the same radius of curvature.

36. A light receiving member as defined in claim 34, wherein the irregularities on the surface of the support are composed of spherical dimples having the same radius of curvature and the same width.

37. A light receiving member as defined in claim 34, wherein the irregularities on the surface of the support are those which are formed by a plurality of rigid spheres each of which having a surface provided with minute irregularities falling spontaneously on the surface of the support.

38. A light receiving member as defined in claim 37, wherein the irregularities on the surface of the support are those which are formed by the rigid spheres of almost the same diameter falling spontaneously on the surface of the support from almost the same height.

39. A light receiving member as defined in claim 34, wherein the spherical dimples have the radius of curvature  $R$  and the width  $D$  which satisfy the following equation

$$0.035 \leq D/R \leq 0.5.$$

40. A light receiving member as defined in claim 39, wherein the spherical dimple has the width  $D$  which satisfies the following equation

$$D \leq 0.5 \text{ mm.}$$

41. A light receiving member as defined in claim 34, wherein the minute irregularity has the height  $h$  which satisfies the following equation

$$0.5 \mu\text{m} \leq h \leq 20 \mu\text{m.}$$

42. A light receiving member as defined in claim 34, wherein the support is a metal member.

43. A light receiving member as defined in claim 34, wherein the photosensitive layer contains a substance for controlling the conductivity.

44. A light receiving member as defined in claim 34, wherein the light receiving layer comprises a charge injection inhibition layer containing a substance for controlling the conductivity as one of the constituent layers.

45. A light receiving member as defined in claim 34, wherein the light receiving layer comprises a barrier layer as one of the constituent layers.

46. A light receiving member as defined in claim 34, wherein the surface layer is composed of an amorphous material containing silicon atoms and at least one of the elements selected from oxygen atoms, carbon atoms and nitrogen atoms, and those elements selected from oxygen atoms, carbon atoms and nitrogen atoms contained in the materials for constituting the photosensitive layer and the surface layer are different from each other.

47. A light receiving member as defined in claim 34, wherein the surface layer is composed of an amorphous material containing silicon atoms and at least one of the elements selected from oxygen atoms, carbon atoms and

nitrogen atoms, and optical band gaps are matched at the interface between the photosensitive layer and the surface layer.

48. A light receiving member as defined in claim 34, wherein the surface layer has a reflection preventive function.

49. A light receiving member as defined in claim 48, wherein the surface layer is composed of at least one of the elements selected from inorganic fluorides, inorganic oxides and inorganic sulfides.

50. A light receiving member as defined in claim 49, wherein the thickness  $d$  of the surface layer can satisfy the following equation:

$$d = \frac{\lambda}{4n} m \quad (m \text{ is a positive odd number})$$

where  $n$  is a refractive index of the substance constituting the surface layer and  $\lambda$  is the wavelength of the irradiation light.

51. A light receiving member as defined in claim 49, wherein the refractive index  $n$  of the substance constituting the surface layer and the refractive index  $n_a$  of the amorphous material constituting the photosensitive layer in adjacent with the surface layer satisfies the following equation:

$$n = \sqrt{n_a}.$$

52. A light receiving member as defined in claim 34, wherein the surface layer is constituted as a multi-layered structure comprising an abrasion-resistant layer at the outermost side and a reflection preventive layer in the inside.

53. A light receiving member as defined in claim 52, wherein the surface layer is composed of an amorphous layer containing silicon atoms and at least one of the elements selected from oxygen atoms, carbon atoms and nitrogen atoms.

54. A light receiving member as defined in claim 52, wherein, the surface layer is composed of material selected from inorganic fluorides, inorganic oxides and inorganic sulfides.

55. An electrophotographic process comprising:  
(a) charging the light receiving member of claim 1; and

(b) irradiating said light receiving member with an electromagnetic wave carrying information, thereby forming an electrostatic image.

56. An electrophotographic process comprising:  
(a) charging the light receiving member of claim 13, and

(b) irradiating the light receiving member with an electromagnetic wave carrying information, thereby forming an electrostatic image.

57. An electrophotographic process comprising:  
(a) charging the light receiving member of claim 34, and

(b) irradiating the light receiving member with an electromagnetic wave carrying information, thereby forming an electrostatic image.

\* \* \* \* \*